

[54] ELECTRICAL RESISTORS, ELECTRICAL RESISTOR PASTE AND METHOD FOR MAKING THE SAME

[75] Inventors: Toshimitsu Honda; Tadahiko Yamada; Kazuji Onikata; Shoichi Tosaka, all of Gumma, Japan

[73] Assignee: Taiyo Yuden Co., Ltd., Tokyo, Japan

[21] Appl. No.: 138,439

[22] Filed: Dec. 28, 1987

[30] Foreign Application Priority Data

Feb. 28, 1987 [JP] Japan ..... 62-045615

Apr. 30, 1987 [JP] Japan ..... 62-104416

Apr. 30, 1987 [JP] Japan ..... 62-104415

[51] Int. Cl.<sup>5</sup> ..... H01B 1/06

[52] U.S. Cl. ..... 252/518; 252/520;

252/521

[58] Field of Search ..... 252/518, 521, 520; 338/22, 308, 20; 427/216, 217, 126.1, 126.2; 264/61, 60; 419/61, 64, 65; 420/429

[56] References Cited

U.S. PATENT DOCUMENTS

4,891,158 1/1990 Hatu ..... 252/518

4,940,849 7/1990 Morris et al. ..... 252/518

Attorney, Agent, or Firm—Birch, Stewart, Kolasch & Birch

[57] ABSTRACT

A fixed chip resistor or a thick-film electrical resistor providing in circuit boards and the like and, to an electrical resistor obtained by sintering in a non-oxidizing atmosphere, resistance pastes for producing an electrical resistor and a method for making such resistors. The aforesaid objects are achieved by the provision of an electrical resistor obtained using at least one molybdate belonging to the following groups (A) and (G) with or without a fluoride of an alkaline earth metal, and an electrical resistor paste obtained using the aforesaid components with or without a carbonate of an alkaline earth metals,

(A) Molybdates of alkaline earth metals,

(B) Molybdate of zinc,

(C) Molybdate of elements Y, La, Ce, Pr, Nd, Sm, Eu, Gd, Tb, Dy, Ho, Er, Tm, Yb and Lu, and complex molybdates of two or more of said elements,

(D) Molybdate of aluminum

(E) Molybdates of elements zirconium and hafnium, and complex molybdates thereof, and

(G) Molybdates of manganese.

17 Claims, 5 Drawing Sheets

Primary Examiner—Josephine Barr



FIG. 1



FIG. 2



FIG. 3



FIG. 4



FIG. 5



## FIG. 6

## X-RAY DIFFRACTION PATTERN

- PEAKS INHERENT IN  $\text{MgMoO}_4$
- PEAK INHERENT IN  $\text{CaF}_2$



## X-RAY DIFFRACTION PATTERN

**FIG. 7**



**X 900,000**

**F / G. 8**



X 900.000

**ELECTRICAL RESISTORS, ELECTRICAL  
RESISTOR PASTE AND METHOD FOR MAKING  
THE SAME**

**BACKGROUND OF THE INVENTION**

**1. Field of the Invention**

The present invention relates to a fixed chip resistor or a thick-film type electrical resistor provided in circuit boards and the like and, more particularly, to an electrical resistor capable of being obtained by sintering in a non-oxidizing atmosphere. The present invention also relates to a method for making such resistors.

**2. Statement of the Prior Art**

Electrical circuits of electronic equipment are generally constructed by mounting various electrical elements such as resistors, capacitors, diodes and transistors to circuit boards. With miniaturization of electronic equipment, however, much use has been made of circuit boards capable of increasing the density of such mounted electrical elements.

The resistors mounted to such circuit boards include a thick-film resistor formed by printing and firing a paste of a resistor material directly onto a circuit, a fixed chip resistor made by forming such a thick-film resistor across a pair of electrode terminals of a rectangular ceramic chip, and the like.

Hitherto, such a thick-film resistor has generally been formed on a circuit board in the following manner. A paste of a conductor material such as Ag or Ag-Pd is applied and fired on the surface of an alumina substrate obtained by sintering at, e.g., about 1500° C. Afterwards, a paste containing, e.g., RuO<sub>2</sub> as the main material of the resistor is applied on that surface by means of screen printing, etc., followed by firing at 750° to 850° C. and, if required, adjustment of a resistance value by means of laser trimming, etc.

However, recent heavy demands for reduction in the weight, thickness, size and cost of electronic equipment, etc. have led to intensive studies for reducing in the size and cost of circuit boards.

Referring to concrete measures to meet the former size reduction, multilayered circuit boards deserve the first mention, and formed resistors the second mention. Known examples of multilayered circuit boards include a multilayered circuitry board obtained by laminating ceramic green sheets, each having a paste of a conductor material such as Ag or Ag-Pd printed thereon, and simultaneously sintering them at 800° to 1100° C. in the air, while known examples of the formed resistor include a multilayered with a formed resistor, obtained by printing a paste of a RuO<sub>2</sub> base resistor material on a ceramic green sheet having said paste of a conductive material printed thereon, laminating such sheets, and then simultaneously sintering them.

Referring to concrete measures to achieve the latter cost reduction, multilayered circuitry boards have been put to practical use, and are obtained by using conductive materials based on inexpensive base metals such as Ni or Cu in place of those based on noble metals such as Ag or Ag-Pd, and sintering them simultaneously with green ceramic at 800° to 1100° C. in a neutral or reducing atmosphere to avoid any increase in resistance due to their oxidation, such as a nitrogen gas or a hydrogen-containing nitrogen gas. As disclosed in Japanese Patent Laid-Open (Kokai) Publication No. 56-153702 in particular, there are also known thick-film resistors, etc. which are obtained by applying a resistor material com-

prising MoSi<sub>2</sub>—TaSi<sub>2</sub> and glass on an alumina substrate including a copper (Cu) conductor followed by a heat treatment.

Where it is intended to simultaneously reduce the size and cost of circuit boards, the RuO<sub>2</sub> base resistor material undergoes a reducing reaction, when it is sintered simultaneously with green ceramic in a nitrogen gas or hydrogen-containing nitrogen atmosphere, and it does not provide any resistor.

Simultaneously sintering of the resistor material comprising MoSi<sub>2</sub>—TaSi<sub>2</sub> and glass and the green ceramic sheet in a non-oxidizing atmosphere also offers the problems that the substrate may warp due to a difference in the dislocation shrinkage curve, or may tend to swell easily due to the gas generated by the decomposing reaction of MoSi<sub>2</sub>—TaSi<sub>2</sub>. To solve such problems, it is known by way of example to use a resistor material comprising MoSi<sub>2</sub>-salts of metal fluorides (e.g. calcium fluoride) and glass, as disclosed in Japanese Patent Laid-Open (Kokai) Publication No. 60-198703. In this example, such warping or swelling of the substrate as mentioned above is not found.

However, when allowed to stand alone in a relative humidity of 95% for 1000 hours, the thick-film resistor obtained by applying such a resistor material comprising MoSi<sub>2</sub>-metal fluorides and glass on a green ceramic sheet and simultaneously sintering them shows a 5 to 10% increase in the resistance value and, hence, cannot perform its own resistor function.

Further, the conventional electrical resistors as mentioned above have posed some problem, when used as the resistor element for a circuit needing precise work, since it is impossible to decrease the temperature dependence coefficient of their resistance value to 1000 ppm/°C. or lower.

**SUMMARY OF THE INVENTION**

A first object of the present invention is to provide an electrical resistor which can be used as a fixed chip resistor or for general circuit boards, and can be laminated with a conductive material of a base metal and formed in a multilayered substrate.

A second object of the present invention is to provide an electrical resistor, the resistance value of which is stabilized.

A third object of the present invention is to provide an electrical resistor, in which the temperature coefficient of resistance value can be decreased.

A fourth object of the present invention is to provide an electrical resistor having excellent properties, which can be obtained even by sintering a resistor material in a reducing atmosphere.

A fifth object of the present invention is to provide an electrical resistor which can meet the reduction in both the size and cost of circuit substrates.

A sixth object of the present invention is to provide a method for making said electrical resistors, which can realize the performance thereof and further improve the properties thereof.

According to the present invention, the aforesaid objects are achieved by the provision of an electrical resistor obtained using at least one molybdate selected from the group consisting of (A) to (G) with or without a fluoride of an alkaline earth metal, and an electrical resistor paste obtained using the aforesaid components with or without a carbonate of an alkaline earth metal:

(A) Molybdates of alkaline earth metals,

- (B) Molybdate of zinc,
- (C) Molybdates of elements Y, La, Ce, Pr, Nd, Sm, Eu, Gd, Tb, Dy, Ho, Er, Tm, Yb and Lu, and complex molybdates of two or more of said elements,
- (D) Molybdate of aluminum
- (E) Molybdates of elements zirconium and hafnium, and complex molybdates thereof, and
- (G) Molybdates of manganese.

According to the present invention, there is also provided a method for making electrical resistors which have their properties improved by using a heat-treated resistor material, and an electrical resistor of the particulate structure obtained by the growth of acicular particles from bulk particles so as to improve its properties.

#### BRIEF DESCRIPTION OF THE DRAWINGS

The aforesaid and other objects and features of the present invention will become apparent from the following detailed description with reference to the accompanying drawings, which are given for the purpose of illustration alone, and in which:

FIG. 1 is a schematic view showing the structure of the electrical resistor according to the present invention;

FIG. 2 is a view of one embodiment of the production of the electrical resistor according to the present invention, in which a resistive film and a conductive are applied on a substrate, and are being formed into a multilayered structure, prior to sintering;

FIG. 3 is a sectional view of that sintered body taken on line III—III;

FIG. 4 is a sectional view of a sintered body of a multilayered structure using a conventional resistor material;

FIG. 5 is a view further illustrating that sintered body which is evolving gas;

FIG. 6 is an X-ray diffraction pattern, where the corresponding molybdate is detected from the electrical resistor of Sample No. 1 according to the example of the present invention;

FIG. 7 is a TEM 900,000 times enlargement photograph showing the structure of the electrical resistor, and

FIG. 8 is a TEM 900,000 times enlargement photograph showing the structure of the electrical resistor obtained by using the resistor material without the fluoride and the carbonate in the resistor material in FIG. 7.

#### DETAILED DESCRIPTION OF THE INVENTION

As illustrated as an example in FIG. 1, the electrical resistor according to the present invention is of the structure wherein spherical particles b and acicular

particles c are dispersed throughout glass a. In this example, the acicular particles are deposited to the spherical particles, or are allowed to be present in the vicinity thereof. A current may pass through such a structure formed by contacting particles or particles in the vicinity thereof. For instance, such a structure may be formed by the sintering treatment of bulk particles of a resistor material, thereby growing the products formed on the surfaces thereof in the acicular form.

As such a resistor body material, at least one molybdate group selected from the consisting of (A) to (G) may be used. For example, the following molybdates are representative of the invention.

##### (A) Molybdates of Alkaline Earth Metals

Preferable molybdates to this end are expressed in terms of the following general formulae:



wherein Me is the alkaline earth metal. For example, the following groups may be mentioned, e.g.,  $\text{MgMoO}_4$ ,  $\text{CaMoO}_4$ ,  $\text{SrMoO}_4$ ,  $\text{BaMoO}_4$ ,  $\text{BaMo}_2\text{O}_7$ ,  $\text{BaMo}_4\text{O}_{13}$ ,  $\text{BaMo}_7\text{O}_{24}$ ,  $\text{BaMo}_3\text{O}_{10}$ ,  $\text{Ca}_3\text{MoO}_6$ ,  $\text{Sr}_3\text{MoO}_6$ ,  $\text{Ba}_3\text{MoO}_6$ ,  $\text{Ba}_2\text{MoO}_5$ ,  $\text{Mg}_2\text{Mo}_3\text{O}_{11}$  and the like.

The following complex molybdates are also exemplified.



##### (B) Molybdates of Zinc

For instance,  $\text{ZnMoO}_4$ ,  $\text{ZnMo}_2\text{O}_7$ ,  $\text{Zn}_3\text{Mo}_2\text{O}_9$  are mentioned.

##### (C) Molybdates of Elements Y, La, Ce, Pr, Nd, Sm, Eu, Gd, Tb, Dy, Ho, Er, Tm, Yb and Lu and Complex Molybdates of Two or More of Said Element

Examples of such molybdates are tabulated in the following table.

| Molybdates of Various Element and Complex Molybdate There of |                                       |                           |                                          |                                       |                                       |
|--------------------------------------------------------------|---------------------------------------|---------------------------|------------------------------------------|---------------------------------------|---------------------------------------|
| $\text{Y}_6\text{MoO}_{12}$                                  | $\text{Y}_2\text{Mo}_3\text{O}_{12}$  | $\text{Y}_2\text{MoO}_5$  | $\text{Y}_4\text{MoO}_9$                 |                                       |                                       |
| $\text{La}_6\text{MoO}_{12}$                                 | $\text{La}_2\text{Mo}_3\text{O}_{12}$ | $\text{La}_2\text{MoO}_6$ | $\text{La}_2\text{Mo}_2\text{O}_9$       | $\text{La}_3\text{Mo}_2\text{O}_{10}$ | $\text{La}_2\text{Mo}_4\text{O}_{15}$ |
| $\text{Ce}_6\text{MoO}_{12}$                                 |                                       |                           | $\text{La}_4\text{MoO}_9$                | $\text{La}_3\text{Mo}_2\text{O}_9$    | $\text{La}_4\text{MoO}_8$             |
| $\text{Pr}_6\text{MoO}_{12}$                                 | $\text{Pr}_2\text{Mo}_3\text{O}_{12}$ | $\text{Pr}_2\text{MoO}_6$ | $\text{CeMo}_2\text{O}_8$                | $\text{Ce}_2\text{Mo}_3\text{O}_{13}$ |                                       |
| $\text{Nd}_6\text{MoO}_{12}$                                 | $\text{Nd}_2\text{Mo}_3\text{O}_{12}$ | $\text{Nd}_2\text{MoO}_6$ | $\text{Nd}_5\text{Mo}_3\text{O}_{16}$    |                                       |                                       |
| $\text{Sm}_6\text{MoO}_{12}$                                 | $\text{Sm}_2\text{Mo}_3\text{O}_{12}$ | $\text{Sm}_2\text{MoO}_6$ | $\text{Sm}_2\text{Mo}_2\text{O}_7$       | $\text{Sm}_2\text{Mo}_2\text{O}_9$    | $\text{Sm}_{18}\text{Mo}_{39}$        |
| $\text{Eu}_6\text{MoO}_{12}$                                 | $\text{Eu}_2\text{Mo}_3\text{O}_{12}$ | $\text{Eu}_2\text{MoO}_6$ | $\text{Eu}_3\text{MoO}_4$                | $\text{Eu}_2\text{Mo}_2\text{O}_7$    |                                       |
| $\text{Gd}_6\text{MoO}_{12}$                                 | $\text{Gd}_2\text{Mo}_3\text{O}_{12}$ | $\text{Gd}_2\text{MoO}_6$ | $\text{Gd}_2\text{Mo}_6\text{O}_{21}$    | $\text{Gd}_2\text{Mo}_4\text{O}_{15}$ |                                       |
| $\text{Tb}_6\text{MoO}_{12}$                                 | $\text{Tb}_2\text{Mo}_3\text{O}_{12}$ | $\text{Tb}_2\text{MoO}_6$ | $\text{Tb}_2\text{Mo}_2\text{O}_9$       |                                       |                                       |
| $\text{Dy}_6\text{MoO}_{12}$                                 |                                       | $\text{Dy}_2\text{MoO}_6$ |                                          |                                       |                                       |
| $\text{Ho}_6\text{MoO}_{12}$                                 | $\text{Ho}_2\text{Mo}_3\text{O}_{12}$ | $\text{Ho}_2\text{MoO}_6$ | $\text{Ho}_{10}\text{Mo}_2\text{O}_{21}$ |                                       |                                       |
| $\text{Er}_6\text{MoO}_{12}$                                 |                                       | $\text{Er}_2\text{MoO}_6$ |                                          |                                       |                                       |
| $\text{Tm}_6\text{MoO}_{12}$                                 |                                       | $\text{Tm}_2\text{MoO}_6$ |                                          |                                       |                                       |
| $\text{Yb}_6\text{MoO}_{12}$                                 |                                       |                           | $\text{Yb}_2\text{Mo}_4\text{O}_{15}$    |                                       |                                       |

-continued

| Molybdates of Various Element and Complex Molybdate There of |                                                 |                                                |
|--------------------------------------------------------------|-------------------------------------------------|------------------------------------------------|
| Lu <sub>6</sub> MoO <sub>12</sub>                            | Lu <sub>2</sub> Mo <sub>3</sub> O <sub>12</sub> | Lu <sub>2</sub> Mo <sub>2</sub> O <sub>9</sub> |

The following complex molybdates of two or more elements are also mentioned.

(Y<sub>x</sub>Ce<sub>y</sub>)MoO<sub>12</sub>, provided that x+y=6,

(Pr<sub>x</sub>Ey<sub>y</sub>)MoO<sub>12</sub>, provided that x+y=6,

(Gd<sub>x</sub>Dy<sub>y</sub>)MoO<sub>12</sub>, provided that x+y=6,

(Ho<sub>x</sub>Tm<sub>y</sub>Yb<sub>z</sub>)MoO<sub>12</sub>, provided that x+y+z=6.

(D) Molybdates of Aluminium

For instance, Al<sub>2</sub>Mo<sub>3</sub>O<sub>12</sub> is mentioned.

(E) Molybdates of Elements Zirconium and Hafnium, and Molybdates of Said Elements

For instance, ZrMo<sub>2</sub>O<sub>3</sub>, HfMo<sub>2</sub>O<sub>8</sub> and (Zr<sub>x</sub> Hf<sub>y</sub>)Mo<sub>2</sub>O<sub>3</sub>, provided that x+y=1, are mentioned.

(F) Molybdates of Elements Niobium and Tantalum

For instance, Nb<sub>2</sub>Mo<sub>3</sub>O<sub>14</sub>, Ta<sub>2</sub>Mo<sub>3</sub>O<sub>14</sub> and (Nb<sub>x</sub> Ta<sub>y</sub>)Mo<sub>3</sub>O<sub>14</sub>, provided that x+y=1, are mentioned.

(G) Molybdates of Manganese

For instance, MnMoO<sub>4</sub> is mentioned.

For use, at least one molybdate is selected from at least one molybdate group selected from the groups (A) to (G). When plural molybdates are selected from said at least one molybdate group, however, the single molybdates and/or complex molybdates of elements may be used.

The molybdates belonging to the aforesaid respective groups can be synthesized by the heat treatment of the oxides of the respective elements and molybdenum oxide (MoO<sub>3</sub>), but may be synthesized by the heat treatment of their precursors. For instance, the molybdates of alkaline earth metals may also be synthesized by mixing substances which provide the precursors of the respective oxides of alkaline earth metals with molybdenum oxide (MoO<sub>3</sub>) or its precursor in the predetermined molar ratio and heat-treating the resulting mixture. As an example, calcium carbonate (CaCO<sub>3</sub>) or calcium hydroxide [Ca(OH)<sub>2</sub>] which is, for instance, the precursor of CaO is mixed with molybdenum oxide (MoO<sub>3</sub>) or its precursor, for instance, molybdcic acid (H<sub>2</sub>MoO<sub>4</sub>) in the predetermined molar ratio, and the mixture is heat-treated. The heat-treatment conditions in this case are 600° to 1000° C. and 1 to 3 hours.

In the present invention, glass is preferably used. As such glass, use may be made of glass generally known in the art. Although the present invention is not limited to glass having a specific composition, it is to be noted that oxides such as Pb<sub>3</sub>O<sub>4</sub>, Bi<sub>2</sub>O<sub>3</sub>, SnO<sub>2</sub> and CdO may be reduced to metals which are likely to change the resistance value of resistors, when resistor materials containing them are sintered in a non-oxidizing atmosphere. Accordingly, where such a phenomenon is unpreferred, it is preferred that the glass used should not contain such oxides.

Preferable as the glass components are SiO<sub>2</sub>, B<sub>2</sub>O<sub>3</sub>, ZnO, CaO, SrO, ZrO<sub>2</sub> and the like. It is preferred that the compositional ratio of such oxides are:

SiO<sub>2</sub>; 12 to 33% by weight

B<sub>2</sub>O<sub>3</sub>; 20 to 35% by weight

ZnO or SrO; 13 to 33% by weight

CAO; 10 to 25% by weight

10 ZrO<sub>2</sub>; 15 to 45% by weight.

To make glass from the compositions of such oxides, the respective oxides are weighed and mixed together in the aforesaid compositional ratio. The mixture is charged in a crucible, in which it is molten at a temperature of 1200° to 1500° C. Thereafter, the melt is poured in, e.g., water for rapid cooling, and the thus obtained coarse glass powders are pulverized to the desired particle size (of, e.g., 10 μm or less) by a pulverizer such as a ball mill or vibration mill to obtain glass powders.

The precursors of the respective oxides may wholly or partly be used and molten into glass. For instance, CaO (calcium oxide) and B<sub>2</sub>O<sub>3</sub> (boron oxide) are obtained by the heat treatment of CaCO<sub>3</sub> (calcium carbonate) and boric acid (H<sub>3</sub>BO<sub>3</sub>), respectively. Hence, CaCO<sub>3</sub> and H<sub>2</sub>BO<sub>3</sub> may be used in place of the whole or a part of CaO and B<sub>2</sub>O<sub>3</sub>. The same also holds for other componential oxides.

The fluorides of alkaline earth metals used in the 30 present invention are expressed in terms of the general formula:

Me'F<sub>2</sub>

35 wherein Me' is the metal. As Me', use is made of alkaline earth metals, i.e., Mg, Ca, Sr and Ba. The respective salts of these metals may preferably be used along or in admixture. In the present invention, however, the fluorides of other metals may also be used in addition to 40 those of alkaline earth metals.

The molybdates of the elements belonging to said element groups and the glass powders obtained in the aforesaid manner are mixed together with or without the fluorides of alkaline earth metals, etc., and the mixtures may be used directly as resistor materials. In view of the resistance temperature properties of resistors, however, it is preferred to heat-treat and pulverize such mixtures and sinter the thus pulverized bodies as the resistor materials. The temperature for this heat treatment is preferably 800° to 1200° C. At a temperature departing from such a temperature range, the resistance value of the resulting resistors are apt to be influenced by delicate variations in the compositional ratio, which are caused by the operational conditions for the respective steps of processing the resistor materials into the electrical resistors. As a consequence, it is difficult to 55 stably obtain the desired resistance value.

The heat treatment is desirously effected in a non-oxidizing atmosphere. To this end, use is preferably made of nitrogen gas or other inert gas, which may or may not contain hydrogen gas.

To prepare a fixed chip resistor or a resistor for thick-film resistors from the thus obtained resistor material powders, the powders are applied on, e.g., a ceramic 65 green sheet, and the resulting produce is sintered. In this case, for instance, the aforesaid molybdate forming the resistor body is preferably used in the form of bulk particles such as spherical, oval or polygonal particles.

This is because it is preferably to allow the original matrixes of the acicular particles to remain in the process of the growth of the acicular particles during sintering. In order to form such a resistor body material into bulk particles, a binder such as glass may also be used.

For the purpose of applying such a resistor material comprising a molybdate and e.g., glass, a vehicle is mixed with the powders of such a resistor material so as to enable, e.g., screen printing. Prepared in this case, however, is a coating liquid to which a carbonate of an alkaline earth metal is added.

Such a carbonate may be expressed in terms of the general formula:



wherein  $\text{Me}''$  is preferably but not exclusively the alkaline earth metal such as Mg, Ca, Sr and Ba. However, carbonates of other metals may be used.

Although varying dependent upon the type and combination of the molybdates of the elements selected from the groups (A) to (G) as already referred to, the compositional ratio of the respective components of the resistor materials should preferably be within the following range, when one or plural molybdates are selected from the same group.

5 powders and 0.5 to 30.0% by weight of the fluoride of an alkaline earth metal.

An amount of the molybdate short excessively of the lower limit of the defined range and an amount of glass exceeding excessively the upper limit of the defined range are unpreferred, since the resistance value of the electrical resistor completed by sintering may become too high. On the contrary, when the amount of the said molybdate is too large and the amount of glass is too small, the binder ability of materials at the time of sintering may drop to such a degree that it is impossible to stably retain the sintered body on a circuit substrate. It is to be noted, however, that when the resistor is for instance laminated on and embedded in a circuit substrate, the molybdate and the fluoride of an alkaline earth metal may be used in an amount of not only higher than their upper limits but also 100%.

An amount of the fluoride of an alkaline earth metal either exceeding excessively the upper limit or short 20 excessively of the lower limit may also be unpreferred, since the temperature dependence coefficient of the finished electrical resistor exceeds  $\pm 500 \text{ ppm}/^\circ\text{C}$ . (the absolute value of  $\pm 500$  is larger than 500), when the carbonate of an alkaline earth metal is present, the value 25 may be made not to exceed  $\pm 300 \text{ ppm}/^\circ\text{C}$ .

It is further noted that when it is not intended to use both the carbonate and fluoride of an alkaline earth

| Group                             | Preferred Composition in weight % |        |        |        |        |        |        |
|-----------------------------------|-----------------------------------|--------|--------|--------|--------|--------|--------|
|                                   | A                                 | B      | C      | D      | E      | F      | G      |
| Molybdate                         | 40-95                             | 65-95  | 60-95  | 45-95  | 50-95  | 55-95  | 65-95  |
| Glass Powders                     | 4-59                              | 4-34   | 4-39   | 4-54   | 4-49   | 4-44   | 4-34   |
| Fluoride of Alkaline Earth Metal  | 0.5-25                            | 0.5-20 | 0.5-10 | 0.5-20 | 0.5-15 | 0.5-15 | 0.5-15 |
| Carbonate of Alkaline Earth Metal | 0.5-50                            | 0.5-30 | 0.5-25 | 0.5-25 | 0.5-45 | 0.5-40 | 0.5-25 |

Otherwise, when at least one molybdate is selected from at least one molybdate group of the groups (A) to

metal, it is preferable to apply the following compositional ratio.

| Group         | Preferred Composition in weight % |       |       |       |       |       |       |
|---------------|-----------------------------------|-------|-------|-------|-------|-------|-------|
|               | A                                 | B     | C     | D     | E     | F     | G     |
| Molybdate     | 30-96                             | 55-95 | 50-96 | 35-96 | 40-96 | 45-96 | 50-96 |
| Glass Powders | 4-70                              | 4-45  | 4-50  | 4-65  | 4-60  | 4-55  | 4-50  |

(G) as already referred to, preferred compositions are composed of 34.8 to 95.0% by weight of the molybdate, 2.1 to 49.5% by weight of glass powders, 0.3 29.9% by weight of the fluoride of an alkaline earth metal and 0.3 to 33.3% by weight of the carbonate of an alkaline earth metal.

It is noted that when the carbonate of an alkaline earth metal is not used, it is preferable to apply the following compositional ratio.

50 Otherwise, it is to be understood, however, that when at least one molybdate is selected from each of at least two groups of the aforesaid groups (A) to (G), preferred compositions are composed of 50-96% by weight of the molybdate and 4 to 50% by weight of the glass powders.

It is to be noted, however, that the fluorides of an alkaline earth metal and the carbonate of an alkaline earth metal may be used in an amount of departing from

| Group                            | Preferred Composition in weight % |          |          |        |          |          |          |
|----------------------------------|-----------------------------------|----------|----------|--------|----------|----------|----------|
|                                  | A                                 | B        | C        | D      | E        | F        | G        |
| Molybdate                        | 30-95                             | 60-95    | 55-95    | 40-95  | 40-95    | 50-95    | 55-95    |
| Glass Powders                    | 4.5-69.5                          | 4.5-39.5 | 4.5-44.5 | 4.5-59 | 4.5-54.5 | 4.5-49.5 | 4.5-44.5 |
| Fluoride of Alkaline Earth metal | 0.5-40                            | 0.5-20   | 0.3-30   | 0.5-30 | 0.5-20   | 0.5-25   | 0.3-30   |

Otherwise, it is to be understood, however, that when at least one molybdate is selected from each of at least two groups of the aforesaid groups (A) to (G), preferred compositions are composed of 35.0 to 95.6% by weight of the molybdate, 2.8 to 49.9% by weight of the glass

65 the defined range, if improvements in the temperature dependence coefficient of resistance is achieved.

Preferably, the aforesaid vehicle should be burned off anywhere prior to sintering. Preferably to this end are organic vehicles, i.e., in which resins are dissolved or

dispersed in organic solvents, if required, with the addition of various additives such as plasticizers and dispersants. Examples of the organic solvents include butyl carbitol acetate, butyl carbitol and turpentine oil, whilst examples of the resins include cellulose derivatives such as ethyl cellulose and nitrocellulose and other resins.

Although the proportion of the organic vehicles with the resistor material powders varies depending upon, e.g., the organic solvents and resins used, the ratio of the organic solvents to the resins to be applied should suitably be in a range of 20 to 50% by weight of the former with respect to 80 to 50% by weight of the latter. These components are pasted with the resistor material by three-roll milling.

The thus obtained resistor material paste is applied on a substrate, and is further subjected to the treatments to be described later to make a resistor. The substrate may be prepared not only by sintering a ceramic green sheet along with a conductive material and a resistor material, but also by previously sintering a ceramic green sheet and applying thereon a resistor material and a conductor material, followed by sintering. Such procedures may also be applied to the formation of laminates.

As the aforesaid ceramic green sheet, use may be made of that obtained by slip-casting a slurry, etc., said slurry being prepared by mixing the organic vehicle with an oxide mixture of ceramic constituents comprising, for instance, 35 to 45% by weight of aluminium oxide ( $Al_2O_3$ ), 25 to 35% by weight of silicon oxide ( $SiO_2$ ), 10 to 15% by weight of boron oxide ( $B_2O_3$ ), 7 to 13% by weight of calcium oxide ( $CaO$ ) and 7 to 10% by weight of magnesium oxide ( $MgO$ ). In this case, when the molybdate of the aforesaid groups is not used with glass, an increased amount of a glassy component may be contained in the aforesaid ceramic green sheet so as to achieve an effect similar to that achieved by the use of glass. The aforesaid organic vehicles may be comprised of acrylic resins such as acryl ester, resins such as polyvinyl butyral, plasticizers such as glycerin and diethyl phthalate, dispersants such as carbonates, and solvents such as organic solvents.

It is preferred that the aforesaid resistive material paste is applied on the ceramic green sheet by means of, e.g., screen printing and, after drying, is heat-treated at 400° to 500° C. to decompose and burn the resinous component.

In this case, a paste of a conductive material of a base metal such as Ni or Cu or a noble metal such as Ag or Ag-Pd is also simultaneously applied on the ceramic green sheet in the same manner.

The paste compositions of the conductive material of a base metal such as Ni or Cu or a noble metal such as Ag or Ag-Pd are exemplified by those obtained by adding 2 to 15% by weight of glass frits to 98 to 85% by weight of the powders of the respective metals.

The resistor material and/or the conductive material are/is incorporated into the ceramic green sheet in this manner. In the case of a fixed chip resistor, by this sintering it is possible to form the conductive material and/or the thick-film resistor material simultaneously into/on the substrates. On the other hand, in the case of the laminate, another similar ceramic green sheet is further put thereon, and after repeating this process, the multilayered board is sintered.

When the conductor material of a base metal such as Ni or Cu is used as the conductor material in this case, sintering should preferably be carried out in a nonoxidizing atmosphere so as to prevent any increase in the

resistance value due to its oxidation. The sintering temperature is exemplified by, e.g., 800° to 1100° C., and the sintering time is exemplified by, e.g., 0.5 to 2 hours. A nitrogen gas or other inert gases which may or may not contain a hydrogen gas may be used as the nonoxidizing atmosphere. When the conductor material of a noble metal such as Ag or Ag-Pd is used, on the other hand, sintering may be carried out in an oxidizing atmosphere of air, for instance.

The circuitry substrate having the conductor and/or resistor incorporated thereinto is completed in the manner as mentioned above. According to the present invention, however, any cracking, distortion, swelling, etc., which may be caused by sintering, are not found in the sintered substrate and the resistor, to say nothing of in the sintered substrate and the conductor, and the resistor shows a resistance value change within only  $\pm 0.1\%$  with respect to changes in a relative humidity of 10 to 90% at 25° C. Further, even after the resistor has been allowed to stand for at least 1000 hours in a high-temperature and-humidity atmosphere, the change in its resistance value is limited to within  $\pm 2\%$ , and the temperature-dependent coefficient of its resistance value in the case of using the fluorides can be reduced not to exceed  $\pm 500$  ppm/°C., while that in the case of using the fluorides and carbonates not to exceed  $\pm 300$  ppm/°C. Such effects appear to be due to the fact that the resistor is well matched with the conductor and the sintered substrate and on the basis of the unique humidity resistance of the resistor comprising the sintered body comprised of the molybdate of the aforesaid groups and glass; however, details thereon are not yet clarified. By X-ray diffraction analysis, the resistor has been found to contain the molybdate. Also, the presence of the bulk and acicular particles has been observed under a transmission type electron microscope (TEM).

In the present invention, the molybdates selected as mentioned above may be used; however, the whole or a part of the precursors of such molybdates may be used in place thereof by a heat treatment. In either cases, it is preferable that they are mixed with glass and heat-treated, and the resulting product is pulverized into a resistor material. Alternatively, the molybdates and/or their precursors may be mixed with the aforesaid vehicles, etc. without any heat treatment to prepare a paste, which is applied on, e.g., a ceramic green sheet, heat-treated for the removal of the organics, and is thereafter sintered directly into a resistor.

Referring to the glass used, it is to be understood that the mixed material of the oxides forming it may result in a sinterable state with the molybdate selected. The whole or a part of such oxides is put to a pasty state together with the molybdate selected and/or its precursor.

The paste is then applied on the substrate, and the aforesaid glassy components are formed into glass in the process of either one of the steps of burning off the organics and the later sintering step. The glass is sintered with the molybdate selected and/or its precursor to thereby prepare a resistor. For instance, since  $CaO$  (calcium oxide) and  $B_2O_3$  (boron oxide) that are the components of glass materials may be obtained from  $CaCO_3$  (calcium carbonate) and  $H_3BO_3$  (boric acid) by heating,  $CaCO_3$  and  $H_3BO_3$  may be used in place of the whole or part of  $CaO$  and  $B_2O_3$ , respectively.

By the resistor material referred to in the present disclosure is meant a material which may be comprised of the molybdate selected, the glass and the fluoride of an alkaline

earth metal as a result of the treating processes involved.

### EXAMPLES

The present invention will now be explained with reference to the following non-restrictive examples.

#### EXAMPLE 1

The respective components were weighed and mixed together according in the compositional ratio calculated as oxides and specified in Table 1.

TABLE 1

|         | Compositional Ratio in % by Weight |                               |      |      |      |                  |
|---------|------------------------------------|-------------------------------|------|------|------|------------------|
|         | SiO <sub>2</sub>                   | B <sub>2</sub> O <sub>3</sub> | ZnO  | CaO  | SrO  | ZrO <sub>2</sub> |
| Glass A | 20.0                               | 29.0                          | 13.0 | 11.0 | 11.0 | 17.0             |
| Glass B | 18.0                               | 28.5                          | 20.2 | 10.5 | —    | 23.0             |

The respective mixtures of Glass A and Glass B were separately molten in alumina crucibles at 1400° C., and

5

10

15

20

the obtained melts were poured in water for rapid cooling. The thus cooled products were taken out of the water, and were milled together with ethanol, and were pulverized by alumina balls into glass powders having a particle size of 10 µm or lower.

The respective molybdates belonging to the aforesaid groups (A) to (G) were synthesized from molybdenum oxide and the oxides of the respective elements. However, the molybdate of an alkaline earth metal was prepared by mixing molybdenum oxide with the carbonate of an alkaline earth metal in a molar ratio of 1:1 and heat-treating the mixture at 700° C. for 1 hour.

The powders obtained from each of Glass A and Glass B, the aforesaid molybdates and the fluorides of alkaline earth metals were weighed and mixed together in the proportions specified in the respective columns of Tables 2-9.

It is understood that Tables 2 to 8 correspond to the groups (A) to (G), and Table 9 indicates the proportions of the components selected from two or more groups.

TABLE 2

| Nos                                               | Molybdates<br>(wt. %) | (Ex. 1)(Group A)<br>Composition |                       |                      |                  |                  |                       |                   |
|---------------------------------------------------|-----------------------|---------------------------------|-----------------------|----------------------|------------------|------------------|-----------------------|-------------------|
|                                                   |                       | Glass<br>A<br>(wt. %)           | Glass<br>B<br>(wt. %) | Fluorides<br>(wt. %) |                  |                  | Carbonates<br>(wt. %) |                   |
|                                                   |                       |                                 |                       | SrF <sub>2</sub>     | BaF <sub>2</sub> | MgF <sub>2</sub> | CaF <sub>2</sub>      | SrCO <sub>3</sub> |
| <u>MgMoO<sub>4</sub></u>                          |                       |                                 |                       |                      |                  |                  |                       |                   |
| 1                                                 | 25                    | 58.4                            | —                     | —                    | —                | —                | 8.3                   | 8.3               |
| 2                                                 | 41.7                  | 41.7                            | —                     | —                    | —                | —                | 8.3                   | 8.3               |
| 3                                                 | 62.5                  | 20.9                            | —                     | —                    | —                | —                | 8.3                   | 8.3               |
| 4                                                 | 80                    | 3.4                             | —                     | —                    | —                | —                | 8.3                   | 8.3               |
| 5                                                 | 41.7                  | —                               | 41.7                  | —                    | —                | —                | 8.3                   | 8.3               |
| 6                                                 | 62.5                  | —                               | 20.9                  | —                    | —                | —                | 8.3                   | 8.3               |
| 7                                                 | 40                    | —                               | 59                    | —                    | —                | —                | 0.5                   | 0.5               |
| 8                                                 | 40                    | —                               | 5                     | —                    | —                | —                | 5                     | 50                |
| 9                                                 | 60                    | —                               | 5                     | —                    | —                | —                | 30                    | 5                 |
| 10                                                | 60                    | —                               | 20                    | —                    | —                | —                | 10                    | 10                |
| 11                                                | 80                    | —                               | 10                    | —                    | —                | —                | 5                     | 5                 |
| 12                                                | 80                    | —                               | 7                     | —                    | —                | —                | 3                     | 10                |
| 13                                                | 95                    | —                               | 4                     | —                    | —                | —                | 0.5                   | 0.5               |
| 14                                                | 40                    | —                               | 59                    | 0.5                  | —                | —                | 0.5                   | —                 |
| 15                                                | 40                    | —                               | 5                     | 5                    | —                | —                | 50                    | —                 |
| 16                                                | 60                    | —                               | 5                     | 30                   | —                | —                | 5                     | —                 |
| 17                                                | 60                    | —                               | 20                    | 10                   | —                | —                | 10                    | —                 |
| 18                                                | 80                    | —                               | 10                    | 5                    | —                | —                | 5                     | —                 |
| 19                                                | 80                    | —                               | 7                     | 3                    | —                | —                | 10                    | —                 |
| 20                                                | 95                    | —                               | 4                     | 0.5                  | —                | —                | 0.5                   | —                 |
| 21                                                | 60                    | —                               | 20                    | —                    | —                | —                | 10                    | —                 |
| 22                                                | 80                    | —                               | 7                     | —                    | —                | —                | 3                     | 10                |
| 23                                                | 60                    | —                               | 20                    | —                    | —                | —                | 10                    | —                 |
| 24                                                | 80                    | —                               | 7                     | —                    | —                | —                | 3                     | 10                |
| 25                                                | 60                    | —                               | 20                    | —                    | —                | —                | 10                    | —                 |
| 26                                                | 80                    | —                               | 7                     | —                    | —                | —                | 3                     | 10                |
| 27                                                | 60                    | —                               | 10                    | —                    | 20               | —                | —                     | 10                |
| 28                                                | 80                    | —                               | 10                    | —                    | 5                | —                | —                     | 5                 |
| 29                                                | 60                    | —                               | 10                    | 20                   | —                | —                | —                     | 10                |
| 30                                                | 80                    | —                               | 10                    | 5                    | —                | —                | —                     | 5                 |
| 31                                                | 60                    | —                               | 10                    | —                    | 20               | —                | —                     | 10                |
| 32                                                | 80                    | —                               | 10                    | 5                    | —                | —                | —                     | 5                 |
| 33                                                | 40                    | —                               | 5                     | 2                    | 2                | 1                | —                     | 25                |
| 34                                                | 60                    | —                               | 20                    | 5                    | 5                | —                | 3                     | 3                 |
| <u>Mg<sub>2</sub>Mo<sub>3</sub>O<sub>11</sub></u> |                       |                                 |                       |                      |                  |                  |                       |                   |
| 35                                                | 25                    | —                               | 58.4                  | —                    | —                | —                | 8.3                   | 8.3               |
| 36                                                | 41.7                  | —                               | 41.7                  | —                    | —                | —                | 8.3                   | 8.3               |
| 37                                                | 62.5                  | —                               | 20.9                  | —                    | —                | —                | 8.3                   | 8.3               |
| 38                                                | 80                    | —                               | 3.4                   | —                    | —                | —                | 8.3                   | 8.3               |
| 39                                                | 41.7                  | 41.7                            | —                     | —                    | —                | —                | 8.3                   | 8.3               |
| 40                                                | 62.5                  | 20.9                            | —                     | —                    | —                | —                | 8.3                   | 8.3               |
| 41                                                | 40                    | —                               | 59                    | 0.5                  | —                | —                | —                     | 0.5               |
| 42                                                | 30                    | —                               | 5                     | 5                    | —                | —                | —                     | 50                |
| 43                                                | 60                    | —                               | 5                     | 30                   | —                | —                | —                     | 5                 |
| 44                                                | 60                    | —                               | 20                    | 10                   | —                | —                | —                     | 10                |
| 45                                                | 80                    | —                               | 10                    | 5                    | —                | —                | —                     | 5                 |
| 46                                                | 80                    | —                               | 7                     | 3                    | —                | —                | —                     | 10                |
| 47                                                | 95                    | —                               | 4                     | 0.5                  | —                | —                | —                     | 0.5               |
| 48                                                | 60                    | —                               | 20                    | 10                   | —                | —                | —                     | 10                |
| 49                                                | 80                    | —                               | 7                     | 3                    | —                | —                | —                     | 10                |

TABLE 2-continued

| Nos | (Ex. 1)(Group A)<br>Composition      |                                                   |                       |                      |                  |                  |                  | Carbonates<br>(wt. %) |                   |                   |                   |
|-----|--------------------------------------|---------------------------------------------------|-----------------------|----------------------|------------------|------------------|------------------|-----------------------|-------------------|-------------------|-------------------|
|     | Molybdates<br>(wt. %)                | Glass<br>A<br>(wt. %)                             | Glass<br>B<br>(wt. %) | Fluorides<br>(wt. %) |                  |                  |                  | SrCO <sub>3</sub>     | BaCO <sub>3</sub> | MgCO <sub>3</sub> | CaCO <sub>3</sub> |
|     |                                      |                                                   |                       | SrF <sub>2</sub>     | BaF <sub>2</sub> | MgF <sub>2</sub> | CaF <sub>2</sub> |                       |                   |                   |                   |
| 50  | 60                                   |                                                   | 20                    | 10                   |                  |                  |                  | 10                    |                   |                   |                   |
| 51  | 80                                   | —                                                 | 7                     | 3                    |                  |                  |                  | 10                    |                   |                   |                   |
| 52  | 60                                   |                                                   | 20                    | 10                   |                  |                  |                  |                       | 10                |                   |                   |
| 53  | 80                                   |                                                   | 7                     | 3                    |                  |                  |                  |                       | 10                |                   |                   |
| 54  | 60                                   | —                                                 | 10                    |                      |                  | 20               |                  |                       |                   |                   | 10                |
| 55  | 80                                   | —                                                 | 10                    |                      |                  | 5                |                  |                       |                   |                   | 5                 |
| 56  | 60                                   | —                                                 | 10                    |                      |                  |                  | 20               |                       |                   |                   | 10                |
| 57  | 80                                   | —                                                 | 10                    |                      |                  |                  | 5                |                       |                   |                   | 5                 |
| 58  | 60                                   | —                                                 | 10                    |                      | 20               |                  |                  |                       |                   |                   | 10                |
| 59  | 80                                   | —                                                 | 10                    |                      | 5                |                  |                  |                       |                   |                   | 5                 |
| 60  | 40                                   | —                                                 | 5                     | 2                    |                  | 1                | 2                |                       |                   | 25                | 25                |
| 61  | 60                                   | —                                                 | 20                    | 5                    |                  | 5                | 5                | 3                     | 3                 |                   | 4                 |
|     | <u>MgMoO<sub>4</sub></u>             | <u>Mg<sub>2</sub>Mo<sub>3</sub>O<sub>11</sub></u> |                       |                      |                  |                  |                  |                       |                   |                   |                   |
| 62  | 40                                   | 40                                                | 3.4                   |                      |                  |                  |                  | 8.3                   | 8.3               |                   |                   |
| 63  | 30                                   | 30                                                | —                     | 20                   | 2.5              | 2.5              | 2.5              | 2.5                   | 2.5               | 2.5               | 2.5               |
|     | <u>CaMoO<sub>4</sub></u>             |                                                   |                       |                      |                  |                  |                  |                       |                   |                   |                   |
| 64  | 25                                   | 58.4                                              | —                     |                      |                  |                  |                  | 8.3                   | 8.3               |                   |                   |
| 65  | 41.7                                 | 41.7                                              | —                     |                      |                  |                  |                  | 8.3                   | 8.3               |                   |                   |
| 66  | 62.5                                 | 20.9                                              | —                     |                      |                  |                  |                  | 8.3                   | 8.3               |                   |                   |
| 67  | 80                                   | 3.4                                               | —                     |                      |                  |                  |                  | 8.3                   | 8.3               |                   |                   |
| 68  | 41.7                                 | —                                                 | 41.7                  |                      |                  |                  |                  | 8.3                   | 8.3               |                   |                   |
| 69  | 62.5                                 | —                                                 | 20.9                  |                      |                  |                  |                  | 8.3                   | 8.3               |                   |                   |
| 70  | 40                                   | 59                                                | 0.5                   |                      |                  |                  |                  |                       |                   |                   | 0.5               |
| 71  | 40                                   | 5                                                 | 5                     |                      |                  |                  |                  |                       |                   |                   | 50                |
| 72  | 60                                   | —                                                 | 5                     | 30                   |                  |                  |                  |                       |                   |                   | 5                 |
| 73  | 60                                   | —                                                 | 20                    | 10                   |                  |                  |                  |                       |                   |                   | 10                |
| 74  | 80                                   | —                                                 | 10                    | 5                    |                  |                  |                  |                       |                   |                   | 5                 |
| 75  | 80                                   | —                                                 | 7                     | 3                    |                  |                  |                  |                       |                   |                   | 10                |
| 76  | 95                                   | —                                                 | 4                     | 0.5                  |                  |                  |                  |                       |                   |                   | 0.5               |
| 77  | 40                                   | 59                                                | 0.5                   |                      |                  |                  | 0.5              |                       |                   |                   |                   |
| 78  | 40                                   | 5                                                 | 5                     |                      |                  |                  | 5                |                       |                   |                   | 50                |
| 79  | 60                                   | —                                                 | 5                     |                      |                  |                  | 30               |                       |                   |                   | 5                 |
| 80  | 60                                   | —                                                 | 20                    |                      |                  |                  | 10               |                       |                   |                   | 10                |
| 81  | 80                                   | —                                                 | 10                    |                      |                  |                  | 5                |                       |                   |                   | 5                 |
| 82  | 80                                   | —                                                 | 7                     |                      |                  |                  | 3                |                       |                   |                   | 10                |
| 83  | 95                                   | —                                                 | 4                     |                      |                  |                  | 0.5              |                       |                   |                   | 0.5               |
| 84  | 60                                   | —                                                 | 20                    | 10                   |                  |                  |                  |                       |                   |                   | 10                |
| 85  | 80                                   | —                                                 | 7                     | 3                    |                  |                  |                  |                       |                   |                   | 10                |
| 86  | 60                                   | —                                                 | 20                    | 10                   |                  |                  |                  | 10                    |                   |                   |                   |
| 87  | 80                                   | —                                                 | 7                     | 3                    |                  |                  |                  | 10                    |                   |                   |                   |
| 88  | 60                                   | —                                                 | 20                    | 10                   |                  |                  |                  |                       | 10                |                   |                   |
| 89  | 80                                   | —                                                 | 7                     | 3                    |                  |                  |                  |                       | 10                |                   |                   |
| 90  | 60                                   | —                                                 | 10                    |                      |                  | 20               |                  |                       |                   |                   | 10                |
| 91  | 80                                   | —                                                 | 10                    |                      |                  | 5                |                  |                       |                   |                   | 5                 |
| 92  | 60                                   | —                                                 | 10                    |                      |                  |                  | 20               |                       |                   |                   | 10                |
| 93  | 80                                   | —                                                 | 10                    |                      |                  |                  | 5                |                       |                   |                   | 5                 |
| 94  | 60                                   | —                                                 | 10                    |                      | 20               |                  |                  |                       |                   |                   | 10                |
| 95  | 80                                   | —                                                 | 10                    |                      | 5                |                  |                  |                       |                   |                   | 5                 |
| 96  | 40                                   | —                                                 | 5                     | 2                    |                  | 1                | 2                | 25                    |                   |                   | 25                |
| 97  | 60                                   | —                                                 | 20                    |                      | 5                | 5                | 3                | 3                     |                   |                   | 4                 |
|     | <u>Ca<sub>3</sub>MoO<sub>6</sub></u> |                                                   |                       |                      |                  |                  |                  |                       |                   |                   |                   |
| 98  | 25                                   | —                                                 | 58.4                  |                      |                  |                  |                  | 8.3                   | 8.3               |                   |                   |
| 99  | 41.7                                 | —                                                 | 41.7                  |                      |                  |                  |                  | 8.3                   | 8.3               |                   |                   |
| 100 | 62.5                                 | —                                                 | 20.9                  |                      |                  |                  |                  | 8.3                   | 8.3               |                   |                   |
| 101 | 80                                   | —                                                 | 3.4                   |                      |                  |                  |                  | 8.3                   | 8.3               |                   |                   |
| 102 | 41.7                                 | 41.7                                              | —                     |                      |                  |                  |                  | 8.3                   | 8.3               |                   |                   |
| 103 | 62.5                                 | 20.9                                              | —                     |                      |                  |                  |                  | 8.3                   | 8.3               |                   |                   |
| 104 | 40                                   | —                                                 | 59                    |                      | 0.5              |                  |                  |                       |                   |                   | 0.5               |
| 105 | 30                                   | —                                                 | 5                     |                      | 5                |                  |                  |                       |                   |                   | 50                |
| 106 | 60                                   | —                                                 | 5                     |                      | 30               |                  |                  |                       |                   |                   | 5                 |
| 107 | 60                                   | —                                                 | 20                    |                      | 10               |                  |                  |                       |                   |                   | 10                |
| 108 | 80                                   | —                                                 | 10                    |                      | 5                |                  |                  |                       |                   |                   | 5                 |
| 109 | 80                                   | —                                                 | 7                     |                      | 3                |                  |                  |                       |                   |                   | 10                |
| 110 | 95                                   | —                                                 | 4                     |                      | 0.5              |                  |                  |                       |                   |                   | 0.5               |
| 111 | 60                                   | —                                                 | 20                    |                      | 10               |                  |                  |                       |                   |                   | 10                |
| 112 | 80                                   | —                                                 | 7                     |                      | 3                |                  |                  |                       |                   |                   | 10                |
| 113 | 60                                   | —                                                 | 20                    |                      | 10               |                  |                  | 10                    |                   |                   |                   |
| 114 | 80                                   | —                                                 | 7                     |                      | 3                |                  |                  | 10                    |                   |                   |                   |
| 115 | 60                                   | —                                                 | 20                    |                      | 10               |                  |                  |                       | 10                |                   |                   |
| 116 | 80                                   | —                                                 | 7                     |                      | 3                |                  |                  |                       | 10                |                   |                   |
| 117 | 60                                   | —                                                 | 10                    |                      |                  | 20               |                  |                       |                   |                   | 10                |
| 118 | 80                                   | —                                                 | 10                    |                      |                  | 5                |                  |                       |                   |                   | 5                 |
| 119 | 60                                   | —                                                 | 10                    |                      |                  |                  | 20               |                       |                   |                   | 10                |
| 120 | 80                                   | —                                                 | 10                    |                      |                  |                  | 5                |                       |                   |                   | 5                 |
| 121 | 60                                   | —                                                 | 10                    | 20                   |                  |                  |                  |                       |                   |                   | 10                |

TABLE 2-continued

| Nos | (Ex. 1)(Group A)                     |                                      |         |         |                  |                  |                   |                  |                   |                    |                   |                   |
|-----|--------------------------------------|--------------------------------------|---------|---------|------------------|------------------|-------------------|------------------|-------------------|--------------------|-------------------|-------------------|
|     | Molybdates                           |                                      | Glass A |         | Glass B          |                  | Fluorides (wt. %) |                  |                   | Carbonates (wt. %) |                   |                   |
|     | (wt. %)                              | (wt. %)                              | (wt. %) | (wt. %) | SrF <sub>2</sub> | BaF <sub>2</sub> | MgF <sub>2</sub>  | CaF <sub>2</sub> | SrCO <sub>3</sub> | BaCO <sub>3</sub>  | MgCO <sub>3</sub> | CaCO <sub>3</sub> |
| 122 | 80                                   | —                                    | —       | 10      | 5                | 2                | 2                 | 1                | 3                 | 3                  | 5                 | 25                |
| 123 | 40                                   | —                                    | —       | 5       | 2                | 2                | 1                 | 3                | 3                 | 4                  | 25                | 25                |
| 124 | 60                                   | —                                    | 20      | 5       | 5                | 2.5              | 2.5               | 2.5              | 2.5               | 2.5                | 2.5               | 2.5               |
|     | <u>CaMoO<sub>4</sub></u>             | <u>Ca<sub>3</sub>MoO<sub>6</sub></u> |         |         |                  |                  |                   |                  |                   |                    |                   |                   |
| 125 | 40                                   | 40                                   | 3.4     | —       | 2.5              | 2.5              | 2.5               | 8.3              | 8.3               | 2.5                | 2.5               | 2.5               |
| 126 | 30                                   | 30                                   | —       | 20      | 2.5              | 2.5              | 2.5               | 2.5              | 2.5               | 2.5                | 2.5               | 2.5               |
|     | <u>SrMoO<sub>4</sub></u>             |                                      |         |         |                  |                  |                   |                  |                   |                    |                   |                   |
| 127 | 25                                   | —                                    | 58.4    | —       |                  |                  |                   | 8.3              | 8.3               |                    |                   |                   |
| 128 | 41.7                                 | —                                    | 41.7    | —       |                  |                  |                   | 8.3              | 8.3               |                    |                   |                   |
| 129 | 62.5                                 | —                                    | 20.9    | —       |                  |                  |                   | 8.3              | 8.3               |                    |                   |                   |
| 130 | 80                                   | —                                    | 3.4     | —       |                  |                  |                   | 8.3              | 8.3               |                    |                   |                   |
| 131 | 41.7                                 | —                                    | 41.7    | —       |                  |                  |                   | 8.3              | 8.3               |                    |                   |                   |
| 132 | 62.5                                 | —                                    | 20.9    | —       |                  |                  |                   | 8.3              | 8.3               |                    |                   |                   |
| 133 | 40                                   | —                                    | 59      | —       |                  |                  |                   | 0.5              | 0.5               |                    |                   |                   |
| 134 | 40                                   | —                                    | 5       | —       |                  |                  |                   | 5                | 50                |                    |                   |                   |
| 135 | 60                                   | —                                    | 5       | —       |                  |                  |                   | 30               | 5                 |                    |                   |                   |
| 136 | 60                                   | —                                    | 20      | —       |                  |                  |                   | 10               | 10                |                    |                   |                   |
| 137 | 80                                   | —                                    | 10      | —       |                  |                  |                   | 5                | 5                 |                    |                   |                   |
| 138 | 80                                   | —                                    | 7       | —       |                  |                  |                   | 3                | 10                |                    |                   |                   |
| 139 | 95                                   | —                                    | 4       | —       |                  |                  |                   | 0.5              | 0.5               |                    |                   |                   |
| 140 | 40                                   | —                                    | 59      | —       | 0.5              |                  |                   |                  |                   |                    | 0.5               |                   |
| 141 | 40                                   | —                                    | 5       | —       | 5                |                  |                   |                  |                   |                    | 50                |                   |
| 142 | 60                                   | —                                    | 5       | —       | 30               |                  |                   |                  |                   |                    | 5                 |                   |
| 143 | 60                                   | —                                    | 20      | —       | 10               |                  |                   |                  |                   |                    | 10                |                   |
| 144 | 80                                   | —                                    | 10      | —       | 5                |                  |                   |                  |                   |                    | 5                 |                   |
| 145 | 80                                   | —                                    | 7       | —       | 3                |                  |                   |                  |                   |                    | 10                |                   |
| 146 | 95                                   | —                                    | 4       | —       | 0.5              |                  |                   |                  |                   |                    | 0.5               |                   |
| 147 | 60                                   | —                                    | 20      | —       |                  |                  |                   | 10               |                   |                    | 10                |                   |
| 148 | 80                                   | —                                    | 7       | —       |                  |                  |                   | 3                |                   |                    | 10                |                   |
| 149 | 60                                   | —                                    | 20      | —       |                  |                  |                   | 10               |                   |                    | 10                |                   |
| 150 | 80                                   | —                                    | 7       | —       |                  |                  |                   | 3                |                   |                    | 10                |                   |
| 151 | 60                                   | —                                    | 20      | —       |                  |                  |                   | 10               |                   |                    | 10                |                   |
| 152 | 80                                   | —                                    | 7       | —       |                  |                  |                   | 3                |                   |                    | 10                |                   |
| 153 | 60                                   | —                                    | 10      | —       |                  |                  |                   | 20               |                   |                    | 10                |                   |
| 154 | 80                                   | —                                    | 10      | —       |                  |                  |                   | 5                |                   |                    | 5                 |                   |
| 155 | 60                                   | —                                    | 10      | —       |                  |                  |                   | 20               |                   |                    | 10                |                   |
| 156 | 80                                   | —                                    | 10      | 5       | —                |                  |                   |                  |                   |                    | 5                 |                   |
| 157 | 60                                   | —                                    | 10      | —       |                  |                  |                   | 20               |                   |                    | 10                |                   |
| 158 | 80                                   | —                                    | 10      | —       |                  |                  |                   | 5                |                   |                    | 5                 |                   |
| 159 | 40                                   | —                                    | 5       | —       |                  |                  |                   | 2                | 1                 |                    | 25                |                   |
| 160 | 60                                   | —                                    | 20      | —       |                  |                  |                   | 5                | 5                 |                    | 3                 |                   |
|     | <u>Sr<sub>3</sub>MoO<sub>6</sub></u> |                                      |         |         |                  |                  |                   |                  |                   |                    |                   |                   |
| 161 | 25                                   | —                                    | 58.4    | —       |                  |                  |                   | 8.3              | 8.3               |                    |                   |                   |
| 162 | 41.7                                 | —                                    | 41.7    | —       |                  |                  |                   | 8.3              | 8.3               |                    |                   |                   |
| 163 | 62.5                                 | —                                    | 20.9    | —       |                  |                  |                   | 8.3              | 8.3               |                    |                   |                   |
| 164 | 80                                   | —                                    | 3.4     | —       |                  |                  |                   | 8.3              | 8.3               |                    |                   |                   |
| 165 | 41.7                                 | 41.7                                 | —       | —       |                  |                  |                   | 8.3              | 8.3               |                    |                   |                   |
| 166 | 62.5                                 | 20.9                                 | —       | —       |                  |                  |                   | 8.3              | 8.3               |                    |                   |                   |
| 167 | 40                                   | —                                    | 59      | 0.5     | —                |                  |                   |                  |                   |                    | 0.5               |                   |
| 168 | 40                                   | —                                    | 5       | 5       | —                |                  |                   |                  |                   |                    | 50                |                   |
| 169 | 60                                   | —                                    | 5       | 30      | —                |                  |                   |                  |                   |                    | 5                 |                   |
| 170 | 60                                   | —                                    | 20      | 10      | —                |                  |                   |                  |                   |                    | 10                |                   |
| 171 | 80                                   | —                                    | 10      | 5       | —                |                  |                   |                  |                   |                    | 5                 |                   |
| 172 | 80                                   | —                                    | 7       | 3       | —                |                  |                   |                  |                   |                    | 10                |                   |
| 173 | 95                                   | —                                    | 4       | 0.5     | —                |                  |                   |                  |                   |                    | 0.5               |                   |
| 174 | 60                                   | —                                    | 20      | 10      | —                |                  |                   |                  |                   |                    | 10                |                   |
| 175 | 80                                   | —                                    | 7       | 3       | —                |                  |                   |                  |                   |                    | 10                |                   |
| 176 | 60                                   | —                                    | 20      | 10      | —                |                  |                   |                  |                   |                    | 10                |                   |
| 177 | 80                                   | —                                    | 7       | 3       | —                |                  |                   |                  |                   |                    | 10                |                   |
| 178 | 60                                   | —                                    | 20      | 10      | —                |                  |                   |                  |                   |                    | 10                |                   |
| 179 | 80                                   | —                                    | 7       | 3       | —                |                  |                   |                  |                   |                    | 10                |                   |
| 180 | 60                                   | —                                    | 10      | —       |                  |                  |                   | 20               |                   |                    | 10                |                   |
| 181 | 80                                   | —                                    | 10      | —       |                  |                  |                   | 5                |                   |                    | 5                 |                   |
| 182 | 60                                   | —                                    | 10      | —       |                  |                  |                   | 20               |                   |                    | 10                |                   |
| 183 | 80                                   | —                                    | 10      | —       |                  |                  |                   | 5                |                   |                    | 5                 |                   |
| 184 | 60                                   | —                                    | 10      | —       |                  |                  |                   | 20               |                   |                    | 10                |                   |
| 185 | 80                                   | —                                    | 10      | —       |                  |                  |                   | 5                |                   |                    | 5                 |                   |
| 186 | 40                                   | —                                    | 5       | —       |                  |                  |                   | 2                | 1                 |                    | 25                |                   |
| 187 | 60                                   | —                                    | 20      | —       |                  |                  |                   | 5                | 5                 |                    | 3                 |                   |
|     | <u>SrMoO<sub>4</sub></u>             | <u>Sr<sub>3</sub>MoO<sub>6</sub></u> | —       |         |                  |                  |                   |                  |                   |                    |                   |                   |
| 188 | 40                                   | 40                                   | 3.4     | —       | 2.5              | 2.5              | 2.5               | 8.3              | 8.3               | 2.5                | 2.5               | 2.5               |
| 189 | 30                                   | 30                                   | —       | 20      | 2.5              | 2.5              | 2.5               | 2.5              | 2.5               | 2.5                | 2.5               | 2.5               |
|     | <u>BaMoO<sub>4</sub></u>             |                                      |         |         |                  |                  |                   |                  |                   |                    |                   |                   |
| 190 | 25                                   | —                                    | 58.4    | —       |                  |                  |                   | 8.3              | 8.3               |                    |                   |                   |
| 191 | 41.7                                 | —                                    | 41.7    | —       |                  |                  |                   | 8.3              | 8.3               |                    |                   |                   |

TABLE 2-continued

(Ex. 1)(Group A)

Composition

| Nos                                                           | Molybdates<br>(wt. %)                                                                           | Glass<br>A<br>(wt. %)            | Glass<br>B<br>(wt. %)            | Fluorides<br>(wt. %) |                  |                  |                  | Carbonates<br>(wt. %) |                   |                   |                   |
|---------------------------------------------------------------|-------------------------------------------------------------------------------------------------|----------------------------------|----------------------------------|----------------------|------------------|------------------|------------------|-----------------------|-------------------|-------------------|-------------------|
|                                                               |                                                                                                 |                                  |                                  | SrF <sub>2</sub>     | BaF <sub>2</sub> | MgF <sub>2</sub> | CaF <sub>2</sub> | SrCO <sub>3</sub>     | BaCO <sub>3</sub> | MgCO <sub>3</sub> | CaCO <sub>3</sub> |
| 192                                                           | 62.5                                                                                            | 20.9                             | —                                |                      |                  |                  | 8.3              | 8.3                   |                   |                   |                   |
| 193                                                           | 80                                                                                              | 3.4                              | —                                |                      |                  |                  | 8.3              | 8.3                   |                   |                   |                   |
| 194                                                           | 41.7                                                                                            | —                                | 41.7                             |                      |                  |                  | 8.3              | 8.3                   |                   |                   |                   |
| 195                                                           | 62.5                                                                                            | —                                | 20.9                             |                      |                  |                  | 8.3              | 8.3                   |                   |                   |                   |
| 196                                                           | 40                                                                                              | —                                | 59                               | 0.5                  |                  |                  |                  |                       |                   | 0.5               |                   |
| 197                                                           | 40                                                                                              | —                                | 5                                | 5                    |                  |                  |                  |                       |                   | 50                |                   |
| 198                                                           | 60                                                                                              | —                                | 5                                | 30                   |                  |                  |                  |                       |                   | 5                 |                   |
| 199                                                           | 60                                                                                              | —                                | 20                               | 10                   |                  |                  |                  |                       |                   | 10                |                   |
| 200                                                           | 80                                                                                              | —                                | 7                                | 3                    |                  |                  |                  |                       |                   | 10                |                   |
| 201                                                           | 95                                                                                              | —                                | 4                                | 0.5                  |                  |                  |                  |                       |                   | 0.5               |                   |
| 202                                                           | 60                                                                                              | —                                | 20                               | 10                   |                  |                  |                  |                       | 10                |                   |                   |
| 203                                                           | 60                                                                                              | —                                | 20                               | 10                   |                  |                  |                  | 10                    |                   |                   |                   |
| 204                                                           | 60                                                                                              | —                                | 20                               | 10                   |                  |                  |                  | 10                    |                   |                   |                   |
| 205                                                           | 80                                                                                              | —                                | 7                                | 3                    |                  |                  |                  |                       |                   | 10                |                   |
| 206                                                           | 80                                                                                              | —                                | 10                               | 3                    |                  |                  |                  |                       |                   | 10                |                   |
| 207                                                           | 80                                                                                              | —                                | 7                                | 5                    |                  |                  |                  |                       |                   | 10                |                   |
| 208                                                           | 40                                                                                              | —                                | 5                                | 5                    |                  |                  |                  |                       |                   | 0.5               |                   |
| 209                                                           | 40                                                                                              | —                                | 5                                | 2.5                  |                  |                  | 5                |                       |                   | 10                |                   |
| 210                                                           | 40                                                                                              | —                                | 5                                | 2.5                  |                  |                  | 2.5              |                       |                   | 10                |                   |
| <u>Ba<sub>2</sub>MoO<sub>5</sub></u>                          |                                                                                                 |                                  |                                  |                      |                  |                  |                  |                       |                   |                   |                   |
| 211                                                           | 25                                                                                              | —                                | 58.4                             |                      |                  |                  | 8.3              | 8.3                   |                   |                   |                   |
| 212                                                           | 41.7                                                                                            | —                                | 41.7                             |                      |                  |                  | 8.3              | 8.3                   |                   |                   |                   |
| 213                                                           | 62.5                                                                                            | —                                | 20.9                             |                      |                  |                  | 8.3              | 8.3                   |                   |                   |                   |
| 214                                                           | 80                                                                                              | —                                | 3.4                              |                      |                  |                  | 8.3              | 8.3                   |                   |                   |                   |
| 215                                                           | 40                                                                                              | —                                | 59                               | 0.5                  |                  |                  |                  |                       |                   | 0.5               |                   |
| 216                                                           | 40                                                                                              | —                                | 5                                | 5                    |                  |                  |                  |                       |                   | 50                |                   |
| 217                                                           | 60                                                                                              | —                                | 20                               | 10                   |                  |                  |                  |                       |                   | 10                |                   |
| 218                                                           | 60                                                                                              | —                                | 5                                | 30                   |                  |                  |                  |                       |                   | 5                 |                   |
| 219                                                           | 80                                                                                              | —                                | 7                                | 3                    |                  |                  |                  |                       |                   | 10                |                   |
| 220                                                           | 95                                                                                              | —                                | 4                                | 0.5                  |                  |                  |                  |                       |                   | 0.5               |                   |
| 221                                                           | 60                                                                                              | —                                | 20                               | 10                   |                  |                  |                  | 3                     | 3                 |                   | 4                 |
| 222                                                           | 60                                                                                              | —                                | 20                               | 10                   |                  |                  |                  |                       |                   |                   | 10                |
| 223                                                           | 60                                                                                              | —                                | 20                               | 10                   |                  |                  |                  |                       | 10                |                   |                   |
| 224                                                           | 80                                                                                              | —                                | 7                                | 3                    |                  |                  |                  |                       |                   | 10                |                   |
| 225                                                           | 80                                                                                              | —                                | 7                                | 3                    |                  |                  |                  |                       |                   | 10                |                   |
| 226                                                           | 80                                                                                              | —                                | 7                                | 20                   |                  |                  | 10               |                       |                   | 10                |                   |
| 227                                                           | 60                                                                                              | —                                | 5                                | 10                   |                  |                  | 10               |                       |                   | 5                 |                   |
| 228                                                           | 60                                                                                              | —                                | 5                                | 20                   |                  |                  | 10               | 2.5                   |                   |                   | 2.5               |
| 229                                                           | 60                                                                                              | —                                | 5                                | 10                   | 10               |                  | 10               |                       |                   |                   | 2                 |
| <u>Ba<sub>3</sub>MoO<sub>6</sub></u>                          |                                                                                                 |                                  |                                  |                      |                  |                  |                  |                       |                   |                   |                   |
| 230                                                           | 41.7                                                                                            | 41.7                             | 41.7                             |                      |                  |                  | 8.3              | 8.3                   |                   |                   |                   |
| 231                                                           | 62.5                                                                                            | 20.9                             | 20.9                             |                      |                  |                  | 8.3              | 8.3                   |                   |                   |                   |
| 232                                                           | 41.7                                                                                            | —                                | 41.7                             |                      |                  |                  | 8.3              | 8.3                   |                   |                   |                   |
| 233                                                           | 62.5                                                                                            | —                                | 20.9                             |                      |                  |                  | 8.3              | 8.3                   |                   |                   |                   |
| 234                                                           | 40                                                                                              | —                                | 59                               | 0.5                  |                  |                  |                  | 0.5                   |                   |                   |                   |
| 235                                                           | 40                                                                                              | —                                | 5                                | 5                    |                  |                  |                  | 5                     |                   | 50                |                   |
| 236                                                           | 60                                                                                              | —                                | 20                               | 10                   |                  |                  | 10               |                       |                   | 10                |                   |
| 237                                                           | 60                                                                                              | —                                | 5                                | 30                   |                  |                  | 30               |                       |                   | 5                 |                   |
| 238                                                           | 80                                                                                              | —                                | 7                                | 3                    |                  |                  | 3                |                       |                   | 10                |                   |
| 239                                                           | 95                                                                                              | —                                | 4                                | 0.5                  |                  |                  | 0.5              |                       |                   | 0.5               |                   |
| 240                                                           | 60                                                                                              | —                                | 20                               | 10                   |                  |                  | 10               |                       |                   | 10                |                   |
| 241                                                           | 60                                                                                              | —                                | 20                               | 10                   |                  |                  | 10               |                       |                   | 10                |                   |
| 242                                                           | 60                                                                                              | —                                | 20                               | 10                   |                  |                  | 10               |                       | 10                |                   |                   |
| 243                                                           | 80                                                                                              | —                                | 7                                | 3                    |                  |                  | 3                | 10                    |                   |                   |                   |
| 244                                                           | 80                                                                                              | —                                | 7                                | 3                    |                  |                  | 3                | 10                    |                   |                   |                   |
| 245                                                           | 80                                                                                              | —                                | 7                                | 3                    |                  |                  | 3                | 10                    |                   |                   |                   |
| <u>BaMoO<sub>4</sub></u> <u>Ba<sub>3</sub>MoO<sub>6</sub></u> |                                                                                                 |                                  |                                  |                      |                  |                  |                  |                       |                   |                   |                   |
| 246                                                           | 40                                                                                              | 40                               | 40                               |                      |                  |                  | 1.5              | 1.5                   | 5                 |                   | 5                 |
|                                                               | BaMoO <sub>4</sub>                                                                              | Ba <sub>3</sub> MoO <sub>6</sub> | Ba <sub>2</sub> MoO <sub>5</sub> |                      |                  |                  |                  |                       |                   |                   |                   |
| 247                                                           | 30                                                                                              | 20                               | 20                               | 7                    | 1                | 0.5              | 0.5              | 1                     | 3                 | 3                 | 2                 |
| 248                                                           | 20.8                                                                                            | 20.8                             | 20.8                             |                      |                  |                  |                  | 8.4                   | 8.4               |                   | 2                 |
| 249                                                           | (Mg <sub>0.3</sub> Ca <sub>0.7</sub> )MoO <sub>4</sub> 41.7                                     |                                  |                                  | 41.7                 | —                | 8.3              |                  |                       |                   |                   | 8.3               |
| 250                                                           | (Mg <sub>0.7</sub> Ca <sub>0.3</sub> )MoO <sub>4</sub> 41.7                                     |                                  |                                  | 41.7                 | —                | 8.3              |                  |                       |                   |                   | 8.3               |
| 251                                                           | (Ca <sub>0.3</sub> Sr <sub>0.7</sub> )MoO <sub>4</sub> 41.7                                     |                                  |                                  | 41.7                 | —                | 8.3              |                  |                       |                   |                   | 8.3               |
| 252                                                           | (Ca <sub>0.7</sub> Sr <sub>0.3</sub> )MoO <sub>4</sub> 41.7                                     |                                  |                                  | 41.7                 | —                | 8.3              |                  |                       |                   |                   | 8.3               |
| 253                                                           | (Mg <sub>0.3</sub> Ba <sub>0.7</sub> )MoO <sub>4</sub> 41.7                                     |                                  |                                  | 41.7                 | —                | 8.3              |                  |                       |                   |                   | 8.3               |
| 254                                                           | (Mg <sub>0.7</sub> Ba <sub>0.3</sub> )MoO <sub>4</sub> 41.7                                     |                                  |                                  | 41.7                 | —                | 8.3              |                  |                       |                   |                   | 8.3               |
| 255                                                           | (Mg <sub>0.2</sub> Ba <sub>0.2</sub> Ba <sub>0.6</sub> )MoO <sub>4</sub> 41.7                   |                                  |                                  | 41.7                 | —                | 8.3              |                  |                       |                   |                   | 8.3               |
| 256                                                           | (Mg <sub>0.3</sub> Ba <sub>0.4</sub> Ba <sub>0.3</sub> )MoO <sub>4</sub> 41.7                   |                                  |                                  | 41.7                 | —                | 8.3              |                  |                       |                   |                   | 8.3               |
| 257                                                           | (Ca <sub>0.2</sub> Sr <sub>0.6</sub> Ba <sub>0.2</sub> )MoO <sub>4</sub> 41.7                   |                                  |                                  | 41.7                 | —                | 8.3              |                  |                       |                   |                   | 8.3               |
| 258                                                           | (Ca <sub>0.4</sub> Sr <sub>0.3</sub> Ba <sub>0.3</sub> )MoO <sub>4</sub> 41.7                   |                                  |                                  | 41.7                 | —                | 8.3              |                  |                       |                   |                   | 8.3               |
| 259                                                           | (Mg <sub>0.2</sub> Ba <sub>0.2</sub> Sr <sub>0.2</sub> Ba <sub>0.4</sub> )MoO <sub>4</sub> 41.7 |                                  |                                  | 41.7                 | —                | 8.3              |                  |                       |                   |                   | 8.3               |
| 260                                                           | (Mg <sub>0.2</sub> Ba <sub>0.3</sub> Sr <sub>0.3</sub> Ba <sub>0.2</sub> )MoO <sub>4</sub> 41.7 |                                  |                                  | 41.7                 | —                | 8.3              |                  |                       |                   |                   | 8.3               |
| 261                                                           | (Ca <sub>2.0</sub> Sr <sub>1.0</sub> )MoO <sub>6</sub> 41.7                                     |                                  |                                  | 41.7                 | —                | 8.3              |                  |                       |                   |                   | 8.3               |
| 262                                                           | (Ca <sub>1.0</sub> Sr <sub>2.0</sub> )MoO <sub>6</sub> 41.7                                     |                                  |                                  | 41.7                 | —                | 8.3              |                  |                       |                   |                   | 8.3               |

TABLE 2-continued

| Nos | Molybdates<br>(wt. %)                                     | Composition<br>(Ex. 1)(Group A) |              |                  |                  |                  |                  | Carbonates<br>(wt. %) |                   |                   |                   |
|-----|-----------------------------------------------------------|---------------------------------|--------------|------------------|------------------|------------------|------------------|-----------------------|-------------------|-------------------|-------------------|
|     |                                                           | Glass                           |              | Fluorides        |                  | Carbonates       |                  |                       |                   |                   |                   |
|     |                                                           | A<br>(wt. %)                    | B<br>(wt. %) | SrF <sub>2</sub> | BaF <sub>2</sub> | MgF <sub>2</sub> | CaF <sub>2</sub> | SrCO <sub>3</sub>     | BaCO <sub>3</sub> | MgCO <sub>3</sub> | CaCO <sub>3</sub> |
| 263 | (Sr <sub>2</sub> 0Ba <sub>1</sub> 0)MoO <sub>6</sub> 41.7 | 41.7                            | —            | 8.3              |                  |                  |                  |                       |                   |                   | 8.3               |
| 264 | (Sr <sub>1</sub> 0Ba <sub>2</sub> 0)MoO <sub>6</sub> 41.7 | 41.7                            | —            | 8.3              |                  |                  |                  |                       |                   |                   | 8.3               |
| 265 | MgMoO <sub>4</sub> 29.2                                   | —                               | 20.8         |                  |                  |                  | 8.3              | 8.3                   |                   |                   |                   |
|     | Ca <sub>3</sub> MoO <sub>6</sub> 33.4                     |                                 |              |                  |                  |                  |                  |                       |                   |                   |                   |
| 266 | CaMoO <sub>4</sub> 29.2                                   | —                               | 20.8         |                  |                  |                  | 8.3              | 8.3                   |                   |                   |                   |
|     | Sr <sub>3</sub> MoO <sub>6</sub> 33.4                     |                                 |              |                  |                  |                  |                  |                       |                   |                   |                   |
| 267 | SrMoO <sub>4</sub> 29.2                                   | —                               | 20.8         |                  |                  |                  | 8.3              | 8.3                   |                   |                   |                   |
|     | Ba <sub>2</sub> MoO <sub>5</sub> 33.4                     |                                 |              |                  |                  |                  |                  |                       |                   |                   |                   |
| 268 | BaMoO <sub>4</sub> 29.2                                   | —                               | 20.8         |                  |                  |                  | 8.3              | 8.3                   |                   |                   |                   |
|     | Mg <sub>2</sub> Mo <sub>3</sub> O <sub>11</sub> 33.4      |                                 |              |                  |                  |                  |                  |                       |                   |                   |                   |
| 269 | MgMoO <sub>4</sub> 20.8                                   | —                               | 20.8         |                  |                  |                  | 8.3              | 8.3                   |                   |                   |                   |
|     | Sr <sub>3</sub> MoO <sub>6</sub> 20.8                     |                                 |              |                  |                  |                  |                  |                       |                   |                   |                   |
| 270 | Ba <sub>3</sub> MoO <sub>6</sub> 20.8                     | —                               | 20.8         |                  |                  |                  | 8.3              | 8.3                   |                   |                   |                   |
|     | Mg <sub>2</sub> Mo <sub>3</sub> O <sub>11</sub> 12.5      |                                 |              |                  |                  |                  |                  |                       |                   |                   |                   |
|     | CaMoO <sub>4</sub> 16.7                                   |                                 |              |                  |                  |                  |                  |                       |                   |                   |                   |
|     | SrMoO <sub>4</sub> 16.7                                   |                                 |              |                  |                  |                  |                  |                       |                   |                   |                   |
|     | BaMoO <sub>4</sub> 16.7                                   |                                 |              |                  |                  |                  |                  |                       |                   |                   |                   |
| 271 | MgMoO <sub>4</sub> 30                                     | —                               | 20           |                  |                  |                  | 10               | 10                    |                   |                   |                   |
|     | Ca <sub>3</sub> MoO <sub>6</sub> 30                       |                                 |              |                  |                  |                  |                  |                       |                   |                   |                   |
| 272 | CaMoO <sub>4</sub> 30                                     | —                               | 20           |                  |                  |                  | 10               | 10                    |                   |                   |                   |
|     | Sr <sub>3</sub> MoO <sub>6</sub> 30                       |                                 |              |                  |                  |                  |                  |                       |                   |                   |                   |
| 273 | SrMoO <sub>4</sub> 30                                     | —                               | 20           |                  |                  |                  | 10               | 10                    |                   |                   |                   |
|     | Ba <sub>2</sub> MoO <sub>5</sub> 30                       |                                 |              |                  |                  |                  |                  |                       |                   |                   |                   |
| 274 | BaMoO <sub>4</sub> 30                                     | —                               | 20           |                  |                  |                  | 10               | 10                    |                   |                   |                   |
|     | Mg <sub>2</sub> Mo <sub>3</sub> O <sub>11</sub> 30        |                                 |              |                  |                  |                  |                  |                       |                   |                   |                   |
| 275 | MgMoO <sub>4</sub> 20                                     | —                               | 20           |                  |                  |                  | 10               | 10                    |                   |                   |                   |
|     | Sr <sub>3</sub> MoO <sub>6</sub> 20                       |                                 |              |                  |                  |                  |                  |                       |                   |                   |                   |
|     | Ba <sub>3</sub> MoO <sub>6</sub> 20                       |                                 |              |                  |                  |                  |                  |                       |                   |                   |                   |
| 276 | Mg <sub>2</sub> Mo <sub>3</sub> O <sub>11</sub> 15        | —                               | 20           |                  |                  |                  | 10               | 10                    |                   |                   |                   |
|     | CaMoO <sub>4</sub> 15                                     |                                 |              |                  |                  |                  |                  |                       |                   |                   |                   |
|     | SrMoO <sub>4</sub> 15                                     |                                 |              |                  |                  |                  |                  |                       |                   |                   |                   |
|     | BaMoO <sub>4</sub> 15                                     |                                 |              |                  |                  |                  |                  |                       |                   |                   |                   |

TABLE 3

(Ex. 1-Group B)

| NOs                                  | Molybdate<br>(wt. %) | Glass        |              | Fluorides<br>(wt. %) |                  |                  | Carbonate<br>(wt. %) |                   |                   |                   |   |
|--------------------------------------|----------------------|--------------|--------------|----------------------|------------------|------------------|----------------------|-------------------|-------------------|-------------------|---|
|                                      |                      | A<br>(wt. %) | B<br>(wt. %) | SrF <sub>2</sub>     | BaF <sub>2</sub> | MgF <sub>2</sub> | CaF <sub>2</sub>     | SrCO <sub>3</sub> | BaCO <sub>3</sub> | MgCO <sub>3</sub> |   |
| <u>ZnMoO<sub>4</sub></u>             |                      |              |              |                      |                  |                  |                      |                   |                   |                   |   |
| 1                                    | 45.9                 | 37.5         | —            |                      |                  |                  | 8.3                  | 8.3               |                   |                   |   |
| 2                                    | 54.2                 | 29.2         | —            |                      |                  |                  | 8.3                  | 8.3               |                   |                   |   |
| 3                                    | 66.7                 | 16.7         | —            |                      |                  |                  | 8.3                  | 8.3               |                   |                   |   |
| 4                                    | 80                   | 3.4          | —            |                      |                  |                  | 8.3                  | 8.3               |                   |                   |   |
| 5                                    | 54.2                 | —            | 29.2         |                      |                  |                  | 8.3                  | 8.3               |                   |                   |   |
| 6                                    | 66.7                 | —            | 16.7         |                      |                  |                  | 8.3                  | 8.3               |                   |                   |   |
| 7                                    | 65                   | —            | 34           |                      |                  | 0.5              |                      |                   |                   | 0.5               |   |
| 8                                    | 65                   | —            | 4            |                      |                  | 1                |                      |                   |                   | 30                |   |
| 9                                    | 75                   | —            | 4            |                      |                  | 20               |                      |                   |                   | 1                 |   |
| 10                                   | 75                   | —            | 10           |                      |                  | 3                |                      |                   |                   | 12                |   |
| 11                                   | 85                   | —            | 5            |                      |                  | 5                |                      |                   |                   | 5                 |   |
| 12                                   | 95                   | —            | 4            |                      |                  | 0.5              |                      |                   |                   | 0.5               |   |
| 13                                   | 65                   | —            | 4            |                      |                  | 1                |                      |                   |                   | 30                |   |
| 14                                   | 75                   | —            | 10           |                      |                  | 3                |                      |                   |                   | 12                |   |
| 15                                   | 65                   | —            | 4            |                      |                  | 1                |                      |                   |                   | 30                |   |
| 16                                   | 75                   | —            | 10           |                      |                  | 3                |                      |                   |                   | 12                |   |
| 17                                   | 65                   | —            | 4            |                      |                  | 1                |                      |                   |                   | 30                |   |
| 18                                   | 75                   | —            | 10           |                      |                  | 3                |                      |                   |                   | 12                |   |
| 19                                   | 75                   | —            | 4            |                      |                  |                  | 20                   |                   |                   |                   | 1 |
| 20                                   | 85                   | —            | 5            |                      |                  |                  | 5                    |                   |                   |                   | 5 |
| 21                                   | 75                   | —            | 4            | 20                   |                  |                  |                      |                   |                   |                   | 1 |
| 22                                   | 85                   | —            | 5            | 5                    |                  |                  |                      |                   |                   |                   | 5 |
| 23                                   | 75                   | —            | 4            |                      | 20               |                  |                      |                   |                   |                   | 1 |
| 24                                   | 85                   | —            | 5            |                      | 5                |                  |                      |                   |                   |                   | 5 |
| 25                                   | 75                   | —            | 10           |                      |                  | 3                |                      | 6                 | 6                 |                   |   |
| 26                                   | 75                   | —            | 10           | 1.5                  |                  |                  | 1.5                  |                   | 6                 |                   | 6 |
| 27                                   | 75                   | —            | 10           | 1                    | 1                |                  | 1                    | 4                 | 4                 |                   | 4 |
| <u>ZnMo<sub>2</sub>O<sub>7</sub></u> |                      |              |              |                      |                  |                  |                      |                   |                   |                   |   |
| 28                                   | 45.9                 | 37.5         | —            |                      |                  |                  | 8.3                  | 8.3               |                   |                   |   |
| 29                                   | 54.2                 | 29.2         | —            |                      |                  |                  | 8.3                  | 8.3               |                   |                   |   |
| 30                                   | 66.7                 | 16.7         | —            |                      |                  |                  | 8.3                  | 8.3               |                   |                   |   |
| 31                                   | 80                   | 3.4          | —            |                      |                  |                  | 8.3                  | 8.3               |                   |                   |   |

TABLE 3-continued

(Ex. 1-Group B)

| NOs                                              | Molybdate<br>(wt. %)                                | Glass<br>A<br>(wt. %) | Glass<br>B<br>(wt. %) | Fluorides<br>(wt. %) |                  |                  | Carbonate<br>(wt. %) |                   |                   |                   |                   |
|--------------------------------------------------|-----------------------------------------------------|-----------------------|-----------------------|----------------------|------------------|------------------|----------------------|-------------------|-------------------|-------------------|-------------------|
|                                                  |                                                     |                       |                       | SrF <sub>2</sub>     | BaF <sub>2</sub> | MgF <sub>2</sub> | CaF <sub>2</sub>     | SrCO <sub>3</sub> | BaCO <sub>3</sub> | MgCO <sub>3</sub> | CaCO <sub>3</sub> |
| 32                                               | 54.2                                                | —                     | 29.2                  |                      |                  |                  | 8.3                  | 8.3               |                   |                   |                   |
| 33                                               | 66.7                                                | —                     | 16.7                  |                      |                  |                  | 8.3                  | 8.3               |                   |                   |                   |
| 34                                               | 65                                                  | —                     | 34                    |                      |                  |                  | 0.5                  | 0.5               |                   |                   |                   |
| 35                                               | 65                                                  | —                     | 4                     |                      |                  |                  | 1                    | 30                |                   |                   |                   |
| 36                                               | 75                                                  | —                     | 4                     |                      |                  |                  | 20                   | 1                 |                   |                   |                   |
| 37                                               | 75                                                  | —                     | 10                    |                      |                  |                  | 3                    | 12                |                   |                   |                   |
| 38                                               | 85                                                  | —                     | 5                     |                      |                  |                  | 5                    | 5                 |                   |                   |                   |
| 39                                               | 95                                                  | —                     | 4                     |                      |                  |                  | 0.5                  | 0.5               |                   |                   |                   |
| 40                                               | 65                                                  | —                     | 4                     |                      |                  |                  | 1                    |                   | 30                |                   |                   |
| 41                                               | 75                                                  | —                     | 10                    |                      |                  |                  | 3                    |                   | 12                |                   |                   |
| 42                                               | 65                                                  | —                     | 4                     |                      |                  |                  | 1                    |                   |                   | 30                |                   |
| 43                                               | 75                                                  | —                     | 10                    |                      |                  |                  | 3                    |                   |                   | 12                |                   |
| 44                                               | 65                                                  | —                     | 4                     |                      |                  |                  | 1                    |                   | 30                |                   |                   |
| 45                                               | 75                                                  | —                     | 10                    |                      |                  |                  | 3                    |                   | 12                |                   |                   |
| 46                                               | 75                                                  | —                     | 4                     |                      |                  | 20               |                      | 1                 |                   |                   |                   |
| 47                                               | 85                                                  | —                     | 5                     |                      |                  | 5                |                      | 5                 |                   |                   |                   |
| 48                                               | 75                                                  | —                     | 4                     | 20                   |                  |                  |                      | 1                 |                   |                   |                   |
| 49                                               | 85                                                  | —                     | 5                     | 5                    |                  |                  |                      | 5                 |                   |                   |                   |
| 50                                               | 75                                                  | —                     | 4                     |                      | 20               |                  |                      | 1                 |                   |                   |                   |
| 51                                               | 85                                                  | —                     | 5                     |                      | 5                |                  |                      | 5                 |                   |                   |                   |
| 52                                               | 65                                                  | —                     | 4                     |                      |                  |                  | 1                    |                   | 15                | 15                |                   |
| 53                                               | 65                                                  | —                     | 4                     | 0.5                  |                  | 0.5              | 0.5                  | 20                | 15                |                   | 10                |
| 54                                               | 65                                                  | —                     | 4                     |                      |                  |                  | 0.5                  | 15                |                   |                   | 15                |
| <u>Zn<sub>3</sub>Mo<sub>2</sub>O<sub>9</sub></u> |                                                     |                       |                       |                      |                  |                  |                      |                   |                   |                   |                   |
| 55                                               | 54.2                                                | 29.2                  | —                     |                      |                  |                  | 8.3                  | 8.3               |                   |                   |                   |
| 56                                               | 66.7                                                | 16.7                  | —                     |                      |                  |                  | 8.3                  | 8.3               |                   |                   |                   |
| 57                                               | 54.2                                                | —                     | 29.2                  |                      |                  |                  | 8.3                  | 8.3               |                   |                   |                   |
| 58                                               | 66.7                                                | —                     | 16.7                  |                      |                  |                  | 8.3                  | 8.3               |                   |                   |                   |
| 59                                               | 65                                                  | —                     | 34                    | 0.5                  |                  |                  |                      |                   | 0.5               |                   |                   |
| 60                                               | 65                                                  | —                     | 4                     | 1                    |                  |                  |                      |                   | 30                |                   |                   |
| 61                                               | 75                                                  | —                     | 4                     | 20                   |                  |                  |                      |                   | 1                 |                   |                   |
| 62                                               | 75                                                  | —                     | 10                    | 3                    |                  |                  |                      |                   | 12                |                   |                   |
| 63                                               | 85                                                  | —                     | 5                     | 5                    |                  |                  |                      |                   | 5                 |                   |                   |
| 64                                               | 95                                                  | —                     | 4                     | 0.5                  |                  |                  |                      |                   | 0.5               |                   |                   |
| 65                                               | 65                                                  | —                     | 4                     | 1                    |                  |                  |                      |                   | 30                |                   |                   |
| 66                                               | 75                                                  | —                     | 10                    | 3                    |                  |                  |                      |                   | 12                |                   |                   |
| 67                                               | 65                                                  | —                     | 4                     | 1                    |                  |                  |                      |                   |                   | 30                |                   |
| 68                                               | 75                                                  | —                     | 10                    | 3                    |                  |                  |                      |                   |                   | 12                |                   |
| 69                                               | 65                                                  | —                     | 4                     | 1                    |                  |                  |                      | 30                |                   |                   |                   |
| 70                                               | 75                                                  | —                     | 10                    | 3                    |                  |                  |                      | 12                |                   |                   |                   |
| 71                                               | 75                                                  | —                     | 4                     |                      | 20               |                  |                      |                   | 1                 |                   |                   |
| 72                                               | 85                                                  | —                     | 5                     |                      | 5                |                  |                      |                   | 5                 |                   |                   |
| 73                                               | 75                                                  | —                     | 4                     |                      |                  | 20               |                      |                   | 1                 |                   |                   |
| 74                                               | 85                                                  | —                     | 5                     |                      |                  | 5                |                      |                   | 5                 |                   |                   |
| 75                                               | 75                                                  | —                     | 4                     |                      | 20               |                  |                      |                   | 1                 |                   |                   |
| 76                                               | 85                                                  | —                     | 5                     |                      | 5                |                  |                      |                   | 5                 |                   |                   |
| 77                                               | 85                                                  | —                     | 5                     | 5                    |                  |                  |                      | 2.5               |                   | 2.5               |                   |
| 78                                               | 85                                                  | —                     | 5                     |                      | 2.5              | 2.5              |                      | 2.5               |                   | 2.5               |                   |
| 79                                               | 85                                                  | —                     | 5                     | 2.5                  | 2.5              |                  | 3                    | 1                 | 3                 |                   | 1                 |
| 80                                               | ZnMoO <sub>4</sub> 35                               | —                     | 10                    |                      |                  |                  |                      |                   |                   |                   | 12                |
|                                                  | ZnMo <sub>2</sub> O <sub>7</sub> 40                 |                       |                       |                      |                  |                  |                      |                   |                   |                   |                   |
| 81                                               | ZnMoO <sub>4</sub> 25                               | 16.7                  | —                     |                      |                  |                  |                      | 8.3               | 8.3               |                   |                   |
|                                                  | ZnMo <sub>2</sub> O <sub>7</sub> 25                 |                       |                       |                      |                  |                  |                      |                   |                   |                   |                   |
|                                                  | Zn <sub>3</sub> Mo <sub>2</sub> O <sub>9</sub> 16.7 |                       |                       |                      |                  |                  |                      |                   |                   |                   |                   |
| 82                                               | ZnMoO <sub>4</sub> 20                               | —                     | 10                    | 1.5                  |                  |                  |                      | 1.5               |                   | 6                 | 6                 |
|                                                  | ZnMo <sub>2</sub> O <sub>7</sub> 25                 |                       |                       |                      |                  |                  |                      |                   |                   |                   |                   |
|                                                  | Zn <sub>3</sub> Mo <sub>2</sub> O <sub>9</sub> 30   |                       |                       |                      |                  |                  |                      |                   |                   |                   |                   |
| 83                                               | ZnMoO <sub>4</sub> 20                               | —                     | 10                    | 1                    | 1                | 0.5              | 0.5                  | 3                 | 3                 | 3                 | 3                 |
|                                                  | ZnMo <sub>2</sub> O <sub>7</sub> 25                 |                       |                       |                      |                  |                  |                      |                   |                   |                   |                   |
|                                                  | Zn <sub>3</sub> Mo <sub>2</sub> O <sub>9</sub> 30   |                       |                       |                      |                  |                  |                      |                   |                   |                   |                   |

TABLE 4

(Ex. 1-Group C)

| NOs | Molybdate<br>Al <sub>2</sub> Mo <sub>3</sub> O <sub>12</sub><br>(wt. %) | Glass<br>A<br>(wt. %) | Glass<br>B<br>(wt. %) | Fluorides<br>(wt. %) |                  |                  | Carbonate<br>(wt. %) |                   |                   |                   |  |
|-----|-------------------------------------------------------------------------|-----------------------|-----------------------|----------------------|------------------|------------------|----------------------|-------------------|-------------------|-------------------|--|
|     |                                                                         |                       |                       | SrF <sub>2</sub>     | BaF <sub>2</sub> | MgF <sub>2</sub> | SrCO <sub>3</sub>    | BaCO <sub>3</sub> | MgCO <sub>3</sub> | CaCO <sub>3</sub> |  |
| 1   | 41.7                                                                    | 41.7                  | —                     |                      |                  | 8.3              | 8.3                  |                   |                   |                   |  |
| 2   | 54.2                                                                    | 29.2                  | —                     |                      |                  | 8.3              | 8.3                  |                   |                   |                   |  |
| 3   | 66.7                                                                    | 16.7                  | —                     |                      |                  | 8.3              | 8.3                  |                   |                   |                   |  |
| 4   | 80                                                                      | 3.4                   | —                     |                      |                  | 8.3              | 8.3                  |                   |                   |                   |  |
| 5   | 41.7                                                                    | —                     | 41.7                  |                      |                  | 8.3              | 8.3                  |                   |                   |                   |  |
| 6   | 54.2                                                                    | —                     | 29.3                  |                      |                  | 8.3              | 8.3                  |                   |                   |                   |  |

TABLE 4-continued

| NOS | Molybdate<br>$\text{Al}_2\text{Mo}_3\text{O}_{12}$<br>(wt. %) | (Ex. 1-Group C)<br>Composition |                       |                      |                |                |                | Carbonate<br>(<br>%<br>) |  |
|-----|---------------------------------------------------------------|--------------------------------|-----------------------|----------------------|----------------|----------------|----------------|--------------------------|--|
|     |                                                               | Glass<br>A<br>(wt. %)          | Glass<br>B<br>(wt. %) | Fluorides<br>(wt. %) |                |                |                |                          |  |
|     |                                                               |                                |                       | $\text{SrF}_2$       | $\text{BaF}_2$ | $\text{MgF}_2$ | $\text{CaF}_2$ |                          |  |
| 7   | 66.7                                                          | —                              | 16.7                  |                      |                |                | 8.3            | 8.3                      |  |
| 8   | 80                                                            | —                              | 3.4                   |                      |                |                | 8.3            | 8.3                      |  |
| 9   | 66.8                                                          | 8.3                            | 8.3                   |                      |                |                | 8.3            | 8.3                      |  |
| 10  | 60                                                            | —                              | 39                    | 0.5                  |                |                | 0.5            |                          |  |
| 11  | 60                                                            | —                              | 5                     | 10                   |                |                | 25             |                          |  |
| 12  | 75                                                            | —                              | 10                    | 5                    |                |                | 10             |                          |  |
| 13  | 85                                                            | —                              | 7                     | 3                    |                |                | 5              |                          |  |
| 14  | 95                                                            | —                              | 4                     | 0.5                  |                |                | 0.5            |                          |  |
| 15  | 60                                                            | —                              | 39                    |                      | 0.5            |                |                | 0.5                      |  |
| 16  | 60                                                            | —                              | 5                     |                      | 10             |                |                | 25                       |  |
| 17  | 75                                                            | —                              | 10                    |                      | 5              |                |                | 10                       |  |
| 18  | 85                                                            | —                              | 7                     |                      | 3              |                |                | 5                        |  |
| 19  | 95                                                            | —                              | 4                     |                      | 0.5            |                |                | 0.5                      |  |
| 20  | 75                                                            | —                              | 10                    | 5                    |                |                |                | 10                       |  |
| 21  | 85                                                            | —                              | 7                     | 3                    |                |                |                | 5                        |  |
| 22  | 75                                                            | —                              | 10                    | 5                    |                |                |                |                          |  |
| 23  | 85                                                            | —                              | 7                     | 3                    |                |                |                | 10                       |  |
| 24  | 75                                                            | —                              | 10                    | 5                    |                |                | 10             |                          |  |
| 25  | 85                                                            | —                              | 7                     | 3                    |                |                | 5              |                          |  |
| 26  | 75                                                            | —                              | 10                    |                      | 5              |                | 10             |                          |  |
| 27  | 85                                                            | —                              | 7                     |                      | 3              |                | 5              |                          |  |
| 28  | 75                                                            | —                              | 10                    |                      |                | 5              | 10             |                          |  |
| 29  | 85                                                            | —                              | 7                     |                      |                | 3              | 5              |                          |  |
| 30  | 75                                                            | —                              | 10                    | 5                    |                |                | 10             |                          |  |
| 31  | 85                                                            | —                              | 7                     | 3                    |                |                | 5              |                          |  |
| 32  | 75                                                            | —                              | 10                    |                      | 5              |                | 5              |                          |  |
| 33  | 75                                                            | —                              | 10                    | 2.5                  |                | 2.5            | 5              |                          |  |
| 34  | 75                                                            | —                              | 10                    | 2                    | 2              | 1              | 3              |                          |  |
| 35  | 85                                                            | —                              | 7                     | 1                    | 1              |                | 2              | 1                        |  |

TABLE 5

| NOS | Molybdate<br>$\text{ZrMo}_2\text{O}_8$<br>(wt. %) | (Ex. 1-Group D)<br>Composition |                       |                      |                |                |                | Carbonates<br>(wt. %) |  |
|-----|---------------------------------------------------|--------------------------------|-----------------------|----------------------|----------------|----------------|----------------|-----------------------|--|
|     |                                                   | Glass<br>A<br>(wt. %)          | Glass<br>B<br>(wt. %) | Fluorides<br>(wt. %) |                |                |                |                       |  |
|     |                                                   |                                |                       | $\text{SrF}_2$       | $\text{BaF}_2$ | $\text{MgF}_2$ | $\text{CaF}_2$ |                       |  |
| 1   | 29.2                                              | 54.2                           | —                     |                      |                |                | 8.3            | 8.3                   |  |
| 2   | 45.9                                              | 37.5                           | —                     |                      |                |                | 8.3            | 8.3                   |  |
| 3   | 62.5                                              | 20.9                           | —                     |                      |                |                | 8.3            | 8.3                   |  |
| 4   | 80                                                | 3.4                            | —                     |                      |                |                | 8.3            | 8.3                   |  |
| 5   | 45.9                                              | —                              | 37.5                  |                      |                |                | 8.3            | 8.3                   |  |
| 6   | 62.5                                              | —                              | 20.9                  |                      |                |                | 8.3            | 8.3                   |  |
| 7   | 45                                                | —                              | 54                    | 0.5                  |                |                |                | 0.5                   |  |
| 8   | 45                                                | —                              | 4                     | 1                    |                |                |                | 50                    |  |
| 9   | 60                                                | —                              | 20                    | 5                    |                |                |                | 15                    |  |
| 10  | 60                                                | —                              | 10                    | 20                   |                |                |                | 10                    |  |
| 11  | 80                                                | —                              | 10                    | 5                    |                |                |                | 5                     |  |
| 12  | 80                                                | —                              | 7                     | 10                   |                |                |                | 3                     |  |
| 13  | 95                                                | —                              | 4                     | 0.5                  |                |                |                | 0.5                   |  |
| 14  | 45                                                | —                              | 54                    |                      | 0.5            |                |                | 0.5                   |  |
| 15  | 45                                                | —                              | 4                     |                      | 1              |                |                | 50                    |  |
| 16  | 60                                                | —                              | 20                    |                      | 5              |                |                | 15                    |  |
| 17  | 60                                                | —                              | 10                    |                      | 20             |                |                | 10                    |  |
| 18  | 80                                                | —                              | 10                    |                      | 5              |                |                | 5                     |  |
| 19  | 80                                                | —                              | 7                     |                      | 10             |                |                | 3                     |  |
| 20  | 95                                                | —                              | 4                     |                      | 0.5            |                |                | 0.5                   |  |
| 21  | 60                                                | —                              | 20                    | 5                    |                |                |                | 15                    |  |
| 22  | 80                                                | —                              | 10                    | 5                    |                |                |                | 5                     |  |
| 23  | 60                                                | —                              | 20                    | 5                    |                |                |                | 15                    |  |
| 24  | 80                                                | —                              | 10                    | 5                    |                |                |                | 5                     |  |
| 25  | 60                                                | —                              | 20                    | 5                    |                |                | 15             |                       |  |
| 26  | 80                                                | —                              | 10                    | 5                    |                |                | 5              |                       |  |
| 27  | 60                                                | —                              | 10                    |                      | 20             |                |                | 10                    |  |
| 28  | 80                                                | —                              | 7                     |                      | 10             |                |                | 3                     |  |
| 29  | 60                                                | —                              | 10                    |                      |                | 20             |                | 10                    |  |
| 30  | 80                                                | —                              | 7                     |                      |                | 10             |                | 3                     |  |
| 31  | 60                                                | —                              | 10                    | 20                   |                |                |                | 10                    |  |
| 32  | 80                                                | —                              | 7                     | 10                   |                |                |                | 3                     |  |
| 33  | 45                                                | —                              | 4                     | 1                    |                | 0.5            | 30             |                       |  |
| 34  | 45                                                | —                              | 4                     |                      | 0.5            | 0.5            | 20             | 10                    |  |

 $\text{HfMo}_2\text{O}_8$

TABLE 5-continued

(Ex. 1-Group D)

Composition

| NOs                                                                  | Molybdate<br>(wt. %)             | Glass        |              | Fluorides<br>(wt. %) |                  |                  | Carbonates<br>(wt. %) |                   |                   |                   |
|----------------------------------------------------------------------|----------------------------------|--------------|--------------|----------------------|------------------|------------------|-----------------------|-------------------|-------------------|-------------------|
|                                                                      |                                  | A<br>(wt. %) | B<br>(wt. %) | SrF <sub>2</sub>     | BaF <sub>2</sub> | MgF <sub>2</sub> | CaF <sub>2</sub>      | SrCO <sub>3</sub> | BaCO <sub>3</sub> | MgCO <sub>3</sub> |
| 35                                                                   | 29.2                             | —            | 54.2         |                      |                  |                  | 8.3                   | 8.3               |                   |                   |
| 36                                                                   | 45.9                             | —            | 37.5         |                      |                  |                  | 8.3                   | 8.3               |                   |                   |
| 37                                                                   | 62.5                             | —            | 20.9         |                      |                  |                  | 8.3                   | 8.3               |                   |                   |
| 38                                                                   | 80                               | —            | 3.4          |                      |                  |                  | 8.3                   | 8.3               |                   |                   |
| 39                                                                   | 45.9                             | 37.5         | —            |                      |                  |                  | 8.3                   | 8.3               |                   |                   |
| 40                                                                   | 62.5                             | 20.9         | —            |                      |                  |                  | 8.3                   | 8.3               |                   |                   |
| 41                                                                   | 45                               | —            | 54           |                      |                  |                  | 0.5                   | 0.5               |                   |                   |
| 42                                                                   | 45                               | —            | 4            |                      |                  |                  | 1                     | 50                |                   |                   |
| 43                                                                   | 60                               | —            | 20           |                      |                  |                  | 5                     | 15                |                   |                   |
| 44                                                                   | 60                               | —            | 10           |                      |                  |                  | 20                    | 10                |                   |                   |
| 45                                                                   | 80                               | —            | 10           |                      |                  |                  | 5                     | 5                 |                   |                   |
| 46                                                                   | 80                               | —            | 7            |                      |                  |                  | 10                    | 3                 |                   |                   |
| 47                                                                   | 95                               | —            | 4            |                      |                  |                  | 0.5                   | 0.5               |                   |                   |
| 48                                                                   | 60                               | —            | 20           |                      |                  |                  | 5                     |                   | 15                |                   |
| 49                                                                   | 80                               | —            | 10           |                      |                  |                  | 5                     |                   | 5                 |                   |
| 50                                                                   | 60                               | —            | 20           |                      |                  |                  | 5                     |                   |                   | 15                |
| 51                                                                   | 80                               | —            | 10           |                      |                  |                  | 5                     |                   |                   | 5                 |
| 52                                                                   | 60                               | —            | 20           |                      |                  |                  | 5                     |                   | 15                |                   |
| 53                                                                   | 80                               | —            | 10           |                      |                  |                  | 5                     |                   | 5                 |                   |
| 54                                                                   | 60                               | —            | 10           |                      |                  | 20               |                       | 10                |                   |                   |
| 55                                                                   | 80                               | —            | 7            |                      |                  | 10               |                       | 3                 |                   |                   |
| 56                                                                   | 60                               | —            | 10           | 20                   |                  |                  |                       | 10                |                   |                   |
| 57                                                                   | 80                               | —            | 7            | 10                   |                  |                  |                       | 3                 |                   |                   |
| 58                                                                   | 60                               | —            | 10           |                      | 20               |                  |                       | 10                |                   |                   |
| 59                                                                   | 80                               | —            | 7            |                      | 10               |                  |                       | 3                 |                   |                   |
| 60                                                                   | 45                               | —            | 4            |                      |                  |                  | 1                     |                   | 30                |                   |
| 61                                                                   | 45                               | —            | 4            | 0.5                  | 0.5              |                  |                       | 20                | 10                | 20                |
| <u>(Zr<sub>0.5</sub>Mo<sub>0.5</sub>)Mo<sub>2</sub>O<sub>8</sub></u> |                                  |              |              |                      |                  |                  |                       |                   |                   |                   |
| 62                                                                   | 80                               | —            | 10           | 1                    | 2                | 1                | 1                     | 1                 | 1                 | 2                 |
| 63                                                                   | ZrMo <sub>2</sub> O <sub>8</sub> | 40           | —            | 10                   | 5                |                  |                       | 5                 |                   |                   |
| 64                                                                   | HfMo <sub>2</sub> O <sub>8</sub> | 40           | —            | 10                   | 1                | 2                | 1                     | 1                 | 1                 | 2                 |
|                                                                      | HfMo <sub>2</sub> O <sub>8</sub> | 40           | —            |                      |                  |                  |                       |                   |                   |                   |

TABLE 6

(Ex. 1-Group E)

Composition

| NOs | Molybdates<br>(wt. %)                | Glass        |              | Fluorides<br>(wt. %) |                  |                  | Carbonate<br>(%) |                   |                   |                   |
|-----|--------------------------------------|--------------|--------------|----------------------|------------------|------------------|------------------|-------------------|-------------------|-------------------|
|     |                                      | A<br>(wt. %) | B<br>(wt. %) | SrF <sub>2</sub>     | BaF <sub>2</sub> | MgF <sub>2</sub> | CaF <sub>2</sub> | SrCO <sub>3</sub> | BaCO <sub>3</sub> | MgCO <sub>3</sub> |
|     | <u>Y<sub>6</sub>MoO<sub>12</sub></u> |              |              |                      |                  |                  |                  |                   |                   |                   |
| 1   | 33.4                                 | 50           | —            |                      |                  |                  | 8.3              | 8.3               |                   |                   |
| 2   | 45.9                                 | 37.5         | —            |                      |                  |                  | 8.3              | 8.3               |                   |                   |
| 3   | 62.5                                 | 20.9         | —            |                      |                  |                  | 8.3              | 8.3               |                   |                   |
| 4   | 80                                   | 3.4          | —            |                      |                  |                  | 8.3              | 8.3               |                   |                   |
| 5   | 45.9                                 | —            | 37.5         |                      |                  |                  | 8.3              | 8.3               |                   |                   |
| 6   | 62.5                                 | —            | 20.9         |                      |                  |                  | 8.3              | 8.3               |                   |                   |
| 7   | 50                                   | —            | 49           | 0.5                  |                  |                  |                  |                   | 0.5               |                   |
| 8   | 50                                   | —            | 20           | 10                   |                  |                  |                  |                   | 20                |                   |
| 9   | 50                                   | —            | 4            | 1                    |                  |                  |                  |                   | 45                |                   |
| 10  | 65                                   | —            | 10           | 15                   |                  |                  |                  |                   | 10                |                   |
| 11  | 65                                   | —            | 20           | 10                   |                  |                  |                  |                   | 5                 |                   |
| 12  | 80                                   | —            | 10           | 5                    |                  |                  |                  |                   | 5                 |                   |
| 13  | 80                                   | —            | 5            | 7.5                  |                  |                  |                  |                   | 7.5               |                   |
| 14  | 95                                   | —            | 4            | 0.5                  |                  |                  |                  |                   | 0.5               |                   |
| 15  | 50                                   | —            | 49           |                      |                  | 0.5              |                  | 0.5               |                   |                   |
| 16  | 50                                   | —            | 20           |                      |                  | 10               |                  | 20                |                   |                   |
| 17  | 50                                   | —            | 4            |                      |                  | 1                |                  | 45                |                   |                   |
| 18  | 65                                   | —            | 10           |                      |                  | 15               |                  | 10                |                   |                   |
| 19  | 65                                   | —            | 20           |                      |                  | 10               |                  | 5                 |                   |                   |
| 20  | 80                                   | —            | 10           |                      |                  | 5                |                  | 5                 |                   |                   |
| 21  | 80                                   | —            | 5            |                      |                  | 7.5              |                  | 7.5               |                   |                   |
| 22  | 95                                   | —            | 4            |                      |                  | 0.5              |                  | 0.5               |                   |                   |
| 23  | 50                                   | —            | 20           | 10                   |                  |                  |                  |                   | 20                |                   |
| 24  | 80                                   | —            | 10           | 5                    |                  |                  |                  |                   | 5                 |                   |
| 25  | 50                                   | —            | 20           | 10                   |                  |                  | 20               |                   |                   |                   |
| 26  | 80                                   | —            | 10           | 5                    |                  |                  | 10               |                   |                   |                   |
| 27  | 50                                   | —            | 20           | 10                   |                  |                  | 20               |                   |                   |                   |
| 28  | 80                                   | —            | 10           | 5                    |                  |                  | 5                |                   |                   |                   |
| 29  | 65                                   | —            | 20           |                      |                  | 10               |                  |                   | 5                 |                   |
| 30  | 80                                   | —            | 10           |                      |                  | 5                |                  |                   | 5                 |                   |
| 31  | 65                                   | —            | 20           |                      |                  | 10               |                  |                   | 5                 |                   |

TABLE 6-continued

| NOs                                   | Molybdates<br>(wt. %) | Composition<br>(Ex. 1-Group E) |                  |                       |                  |                      |                   |                          |                   |  |
|---------------------------------------|-----------------------|--------------------------------|------------------|-----------------------|------------------|----------------------|-------------------|--------------------------|-------------------|--|
|                                       |                       | Glass<br>A<br>(wt. %)          |                  | Glass<br>B<br>(wt. %) |                  | Fluorides<br>(wt. %) |                   | Carbonate<br>(<br>%<br>) |                   |  |
|                                       |                       | SrF <sub>2</sub>               | BaF <sub>2</sub> | MgF <sub>2</sub>      | CaF <sub>2</sub> | SrCO <sub>3</sub>    | BaCO <sub>3</sub> | MgCO <sub>3</sub>        | CaCO <sub>3</sub> |  |
| 32                                    | 80                    | —                              | 10               |                       |                  | 5                    |                   |                          | 5                 |  |
| 33                                    | 65                    | —                              | 20               | 10                    |                  |                      |                   |                          | 5                 |  |
| 34                                    | 80                    | —                              | 10               | 5                     |                  |                      |                   |                          | 5                 |  |
| 35                                    | 50                    | —                              | 20               | 10                    |                  |                      |                   | 10                       | 10                |  |
| 36                                    | 50                    | —                              | 20               | 5                     | 5                | 10                   | 10                |                          |                   |  |
| 37                                    | 50                    | —                              | 20               | 3                     | 4                | 5                    | 5                 | 10                       |                   |  |
| 38                                    | 50                    | —                              | 20               | 3                     | 3                | 2                    | 5                 | 5                        | 5                 |  |
| <u>La<sub>6</sub>MoO<sub>12</sub></u> |                       |                                |                  |                       |                  |                      |                   |                          |                   |  |
| 39                                    | 33.4                  | —                              | 50               |                       |                  | 8.3                  | 8.3               |                          |                   |  |
| 40                                    | 45.9                  | —                              | 37.5             |                       |                  | 8.3                  | 8.3               |                          |                   |  |
| 41                                    | 62.5                  | —                              | 20.9             |                       |                  | 8.3                  | 8.3               |                          |                   |  |
| 42                                    | 80                    | —                              | 3.4              |                       |                  | 8.3                  | 8.3               |                          |                   |  |
| 43                                    | 45.9                  | 37.5                           | —                |                       |                  | 8.3                  | 8.3               |                          |                   |  |
| 44                                    | 62.5                  | 20.9                           | —                |                       |                  | 8.3                  | 8.3               |                          |                   |  |
| 45                                    | 50                    | —                              | 49               | 0.5                   |                  |                      |                   | 0.5                      |                   |  |
| 46                                    | 50                    | —                              | 20               | 10                    |                  |                      |                   | 20                       |                   |  |
| 47                                    | 50                    | —                              | 4                | 1                     |                  |                      |                   | 45                       |                   |  |
| 48                                    | 65                    | —                              | 10               | 15                    |                  |                      |                   | 10                       |                   |  |
| 49                                    | 65                    | —                              | 20               | 10                    |                  |                      |                   | 5                        |                   |  |
| 50                                    | 80                    | —                              | 10               | 5                     |                  |                      |                   | 5                        |                   |  |
| 51                                    | 80                    | —                              | 5                | 7.5                   |                  |                      |                   | 7.5                      |                   |  |
| 52                                    | 95                    | —                              | 4                | 0.5                   |                  |                      |                   | 0.5                      |                   |  |
| 53                                    | 80                    | —                              | 5                | 7.5                   |                  |                      |                   | 7.5                      |                   |  |
| 54                                    | 50                    | —                              | 20               |                       | 5                | 5                    |                   | 20                       |                   |  |
| 55                                    | 50                    | —                              | 20               | 5                     | 5                |                      |                   | 20                       |                   |  |
| 56                                    | 50                    | —                              | 20               | 4                     | 3                | 3                    |                   | 20                       |                   |  |
| <u>Ce<sub>6</sub>MoO<sub>12</sub></u> |                       |                                |                  |                       |                  |                      |                   |                          |                   |  |
| 57                                    | 45.9                  | 37.5                           | —                |                       |                  | 8.3                  | 8.3               |                          |                   |  |
| 58                                    | 62.5                  | —                              | 20.9             |                       |                  | 8.3                  | 8.3               |                          |                   |  |
| 59                                    | 80                    | —                              | 5                | 7.5                   |                  |                      |                   | 7.5                      |                   |  |
| <u>Pr<sub>6</sub>MoO<sub>12</sub></u> |                       |                                |                  |                       |                  |                      |                   |                          |                   |  |
| 60                                    | 45.9                  | 37.5                           | —                |                       |                  | 8.3                  | 8.3               |                          |                   |  |
| 61                                    | 62.5                  | —                              | 20.9             |                       |                  | 8.3                  | 8.3               |                          |                   |  |
| 62                                    | 80                    | —                              | 5                | 7.5                   |                  |                      |                   | 7.5                      |                   |  |
| <u>Nd<sub>6</sub>MoO<sub>12</sub></u> |                       |                                |                  |                       |                  |                      |                   |                          |                   |  |
| 63                                    | 45.9                  | 37.5                           | —                |                       |                  | 8.3                  | 8.3               |                          |                   |  |
| 64                                    | 62.5                  | —                              |                  |                       | 8.3              | 8.3                  |                   |                          |                   |  |
| 65                                    | 80                    | —                              | 5                | 7.5                   |                  |                      |                   | 7.5                      |                   |  |
| <u>Sm<sub>6</sub>MoO<sub>12</sub></u> |                       |                                |                  |                       |                  |                      |                   |                          |                   |  |
| 66                                    | 45.9                  | 37.5                           | —                |                       |                  | 8.3                  | 8.3               |                          |                   |  |
| 67                                    | 62.5                  | —                              | 20.9             |                       |                  | 8.3                  | 8.3               |                          |                   |  |
| 68                                    | 80                    | —                              | 5                | 7.5                   |                  |                      |                   | 7.5                      |                   |  |
| <u>Eu<sub>6</sub>MoO<sub>12</sub></u> |                       |                                |                  |                       |                  |                      |                   |                          |                   |  |
| 69                                    | 45.9                  | 37.5                           | —                |                       |                  | 8.3                  | 8.3               |                          |                   |  |
| 70                                    | 62.5                  | —                              | 20.9             |                       |                  | 8.3                  | 8.3               |                          |                   |  |
| 71                                    | 80                    | —                              | 5                | 7.5                   |                  |                      |                   | 7.5                      |                   |  |
| <u>Gd<sub>6</sub>MoO<sub>12</sub></u> |                       |                                |                  |                       |                  |                      |                   |                          |                   |  |
| 72                                    | 45.9                  | 37.5                           | —                |                       |                  | 8.3                  | 8.3               |                          |                   |  |
| 73                                    | 62.5                  | —                              | 20.9             |                       |                  | 8.3                  | 8.3               |                          |                   |  |
| 74                                    | 80                    | —                              | 5                | 7.5                   |                  |                      |                   | 7.5                      |                   |  |
| <u>Tb<sub>6</sub>MoO<sub>12</sub></u> |                       |                                |                  |                       |                  |                      |                   |                          |                   |  |
| 75                                    | 45.9                  | 37.5                           | —                |                       |                  | 8.3                  | 8.3               |                          |                   |  |
| 76                                    | 62.5                  | —                              | 20.9             |                       |                  | 8.3                  | 8.3               |                          |                   |  |
| 77                                    | 80                    | —                              | 5                | 7.5                   |                  |                      |                   | 7.5                      |                   |  |
| <u>Dy<sub>6</sub>MoO<sub>12</sub></u> |                       |                                |                  |                       |                  |                      |                   |                          |                   |  |
| 78                                    | 45.9                  | 37.5                           | —                |                       |                  | 8.3                  | 8.3               |                          |                   |  |
| 79                                    | 62.5                  | —                              | 20.9             |                       |                  | 8.3                  | 8.3               |                          |                   |  |
| 80                                    | 80                    | —                              | 5                | 7.5                   |                  |                      |                   | 7.5                      |                   |  |
| <u>Ho<sub>6</sub>MoO<sub>12</sub></u> |                       |                                |                  |                       |                  |                      |                   |                          |                   |  |
| 81                                    | 45.9                  | 37.5                           | —                |                       |                  | 8.3                  | 8.3               |                          |                   |  |
| 82                                    | 62.5                  | —                              | 20.9             |                       |                  | 8.3                  | 8.3               |                          |                   |  |
| 83                                    | 80                    | —                              | 5                | 7.5                   |                  |                      |                   | 7.5                      |                   |  |
| <u>Er<sub>6</sub>MoO<sub>12</sub></u> |                       |                                |                  |                       |                  |                      |                   |                          |                   |  |
| 84                                    | 45.9                  | 37.5                           | —                |                       |                  | 8.3                  | 8.3               |                          |                   |  |
| 85                                    | 62.5                  | —                              | 20.9             |                       |                  | 8.3                  | 8.3               |                          |                   |  |
| 86                                    | 80                    | —                              | 5                | 7.5                   |                  |                      |                   | 7.5                      |                   |  |
| <u>Tm<sub>6</sub>MoO<sub>12</sub></u> |                       |                                |                  |                       |                  |                      |                   |                          |                   |  |
| 87                                    | 45.9                  | 37.5                           | —                |                       |                  | 8.3                  | 8.3               |                          |                   |  |
| 88                                    | 62.5                  | —                              | 20.9             |                       |                  | 8.3                  | 8.3               |                          |                   |  |
| 89                                    | 80                    | —                              | 5                | 7.5                   |                  |                      |                   | 7.5                      |                   |  |
| <u>Yb<sub>6</sub>MoO<sub>12</sub></u> |                       |                                |                  |                       |                  |                      |                   |                          |                   |  |
| 90                                    | 45.9                  | 37.5                           | —                |                       |                  | 8.3                  | 8.3               |                          |                   |  |
| 91                                    | 62.5                  | —                              | 20.9             |                       |                  | 8.3                  | 8.3               |                          |                   |  |

TABLE 6-continued

| NOS | Molybdates<br>(wt. %)                                                                                                | Composition  |              |                  |                  |                  |                  |                   |                   |
|-----|----------------------------------------------------------------------------------------------------------------------|--------------|--------------|------------------|------------------|------------------|------------------|-------------------|-------------------|
|     |                                                                                                                      | Glass        |              | Fluorides        |                  | Carbonate        |                  |                   |                   |
|     |                                                                                                                      | A<br>(wt. %) | B<br>(wt. %) | SrF <sub>2</sub> | BaF <sub>2</sub> | MgF <sub>2</sub> | CaF <sub>2</sub> | SrCO <sub>3</sub> | BaCO <sub>3</sub> |
| 92  | 80<br><u>Lu<sub>6</sub>MoO<sub>12</sub></u>                                                                          | —            | 5            | 7.5              |                  |                  |                  |                   | 7.5               |
| 93  | 45.9                                                                                                                 | 37.5         | —            |                  |                  | 8.3              | 8.3              |                   |                   |
| 94  | 62.5                                                                                                                 | —            | 20.9         |                  |                  | 8.3              | 8.3              |                   |                   |
| 95  | 80                                                                                                                   | —            | 5            | 7.5              |                  |                  |                  |                   | 7.5               |
| 96  | (Y <sub>3.0</sub> Ce <sub>3.0</sub> )MoO <sub>12</sub> 65                                                            | —            | 20           | 10               |                  |                  |                  | 5                 |                   |
| 97  | (Pr <sub>3.0</sub> Eu <sub>3.0</sub> )MoO <sub>12</sub> 65                                                           | —            | 20           | 10               |                  |                  |                  | 5                 |                   |
| 98  | (Gd <sub>3.0</sub> Dy <sub>3.0</sub> )MoO <sub>12</sub> 65                                                           | —            | 20           | 10               |                  |                  |                  | 5                 |                   |
| 99  | (La <sub>2.0</sub> Nd <sub>2.0</sub> Tb <sub>2.0</sub> )MoO <sub>12</sub><br>65                                      | —            | 20           | 10               |                  |                  |                  | 5                 |                   |
| 100 | (Ho <sub>2.0</sub> Tm <sub>2.0</sub> Yb <sub>2.0</sub> )MoO <sub>12</sub><br>65                                      | —            | 20           | 10               |                  |                  | 5                |                   |                   |
| 101 | Y <sub>6</sub> MoO <sub>12</sub> 40<br>La <sub>6</sub> MoO <sub>12</sub> 40                                          | —            | 5            |                  |                  | 7.5              | 7.5              |                   |                   |
| 102 | Nd <sub>6</sub> MoO <sub>12</sub> 40<br>Sm <sub>6</sub> MoO <sub>12</sub> 40                                         | —            | 5            |                  |                  | 7.5              | 7.5              |                   |                   |
| 103 | Gd <sub>6</sub> MoO <sub>12</sub> 40<br>Dy <sub>6</sub> MoO <sub>12</sub> 40                                         | —            | 5            |                  |                  | 7.5              | 7.5              |                   |                   |
| 104 | Ho <sub>6</sub> MoO <sub>12</sub> 20<br>Er <sub>6</sub> MoO <sub>12</sub> 30<br>Tm <sub>6</sub> MoO <sub>12</sub> 30 | —            | 5            |                  |                  | 7.5              | 7.5              |                   |                   |
| 105 | Yb <sub>6</sub> MoO <sub>12</sub> 20<br>Lu <sub>6</sub> MoO <sub>12</sub> 30<br>Eu <sub>6</sub> MoO <sub>12</sub> 30 | —            | 5            |                  |                  | 7.5              | 7.5              |                   |                   |

TABLE 7

| NOS                                               | Molybdates<br>(wt. %) | Composition  |              |                  |                  |                       |                  |                   |                   |
|---------------------------------------------------|-----------------------|--------------|--------------|------------------|------------------|-----------------------|------------------|-------------------|-------------------|
|                                                   |                       | Glass        |              | Fluorides        |                  | Carbonates<br>(wt. %) |                  |                   |                   |
|                                                   |                       | A<br>(wt. %) | B<br>(wt. %) | SrF <sub>2</sub> | BaF <sub>2</sub> | MgF <sub>2</sub>      | CaF <sub>2</sub> | SrCO <sub>3</sub> | BaCO <sub>3</sub> |
| <u>Nb<sub>2</sub>Mo<sub>3</sub>O<sub>14</sub></u> |                       |              |              |                  |                  |                       |                  |                   |                   |
| 1                                                 | 37.5                  | 45.9         | —            |                  |                  | 8.3                   | 8.3              |                   |                   |
| 2                                                 | 54.2                  | 29.2         | —            |                  |                  | 8.3                   | 8.3              |                   |                   |
| 3                                                 | 66.7                  | 16.7         | —            |                  |                  | 8.3                   | 8.3              |                   |                   |
| 4                                                 | 80                    | 3.4          | —            |                  |                  | 8.3                   | 8.3              |                   |                   |
| 5                                                 | 54.2                  | —            | 29.2         |                  |                  | 8.3                   | 8.3              |                   |                   |
| 6                                                 | 66.7                  | —            | 16.7         |                  |                  | 8.3                   | 8.3              |                   |                   |
| 7                                                 | 55                    | —            | 44           | 0.5              |                  |                       |                  | 0.5               |                   |
| 8                                                 | 55                    | —            | 4            | 1                |                  |                       |                  | 40                |                   |
| 9                                                 | 70                    | —            | 10           | 15               |                  |                       |                  | 5                 |                   |
| 10                                                | 70                    | —            | 10           | 5                |                  |                       |                  | 15                |                   |
| 11                                                | 80                    | —            | 7            | 3                |                  |                       |                  | 10                |                   |
| 12                                                | 95                    | —            | 4            | 0.5              |                  |                       |                  | 0.5               |                   |
| 13                                                | 70                    | —            | 10           | 15               |                  |                       |                  | 5                 |                   |
| 14                                                | 80                    | —            | 7            | 3                |                  |                       |                  | 10                |                   |
| 15                                                | 70                    | —            | 10           | 15               |                  | 5                     |                  |                   |                   |
| 16                                                | 80                    | —            | 7            | 3                |                  | 10                    |                  |                   |                   |
| 17                                                | 70                    | —            | 10           | 15               |                  |                       | 5                |                   |                   |
| 18                                                | 80                    | —            | 7            | 3                |                  |                       | 10               |                   |                   |
| 19                                                | 55                    | —            | 4            | 1                |                  |                       |                  | 40                |                   |
| 20                                                | 70                    | —            | 10           | 5                |                  |                       |                  | 15                |                   |
| 21                                                | 55                    | —            | 4            |                  | 1                |                       |                  | 40                |                   |
| 22                                                | 70                    | —            | 10           |                  | 5                |                       |                  | 15                |                   |
| 23                                                | 55                    | —            | 4            | 1                |                  |                       |                  | 40                |                   |
| 24                                                | 70                    | —            | 10           | 5                |                  |                       |                  | 15                |                   |
| 25                                                | 70                    | —            | 10           | 5                |                  | 10                    |                  |                   | 5                 |
| 26                                                | 70                    | —            | 10           | 2.5              |                  | 2.5                   | 5                |                   | 5                 |
| <u>Ta<sub>2</sub>Mo<sub>3</sub>O<sub>14</sub></u> |                       |              |              |                  |                  |                       |                  |                   |                   |
| 27                                                | 37.5                  | —            | 45.9         |                  |                  | 8.3                   | 8.3              |                   |                   |
| 28                                                | 54.2                  | —            | 29.2         |                  |                  | 8.3                   | 8.3              |                   |                   |
| 29                                                | 66.7                  | —            | 16.7         |                  |                  | 8.3                   | 8.3              |                   |                   |
| 30                                                | 80                    | —            | 3.4          |                  |                  | 8.3                   | 8.3              |                   |                   |
| 31                                                | 54.2                  | 29.2         | —            |                  |                  | 8.3                   | 8.3              |                   |                   |
| 32                                                | 66.7                  | 16.7         | —            |                  |                  | 8.3                   | 8.3              |                   |                   |
| 33                                                | 55                    | —            | 44           |                  |                  | 0.5                   | 0.5              |                   |                   |
| 34                                                | 55                    | —            | 4            |                  |                  | 1                     | 40               |                   |                   |
| 35                                                | 70                    | —            | 10           |                  | 15               | 5                     |                  |                   |                   |
| 36                                                | 70                    | —            | 10           |                  |                  | 5                     | 15               |                   |                   |
| 37                                                | 80                    | —            | 7            |                  |                  | 3                     | 10               |                   |                   |
| 38                                                | 95                    | —            | 4            |                  |                  | 0.5                   | 0.5              |                   |                   |
| 39                                                | 70                    | —            | 10           |                  | 15               |                       |                  | 5                 |                   |

TABLE 7-continued

| Nos | Molybdates<br>(wt. %)                                                 | Composition  |              |                      |                  |                   |                  | Carbonates<br>(wt. %) |                   |                   |
|-----|-----------------------------------------------------------------------|--------------|--------------|----------------------|------------------|-------------------|------------------|-----------------------|-------------------|-------------------|
|     |                                                                       | Glass        |              | Fluorides<br>(wt. %) |                  | SrCO <sub>3</sub> |                  |                       | BaCO <sub>3</sub> |                   |
|     |                                                                       | A<br>(wt. %) | B<br>(wt. %) | SrF <sub>2</sub>     | BaF <sub>2</sub> | MgF <sub>2</sub>  | CaF <sub>2</sub> |                       |                   | MgCO <sub>3</sub> |
| 40  | 80                                                                    | —            | 7            |                      |                  |                   | 3                |                       |                   | 10                |
| 41  | 70                                                                    | —            | 10           |                      |                  |                   | 15               |                       |                   | 5                 |
| 42  | 80                                                                    | —            | 7            |                      |                  |                   | 3                |                       |                   | 10                |
| 43  | 70                                                                    | —            | 10           |                      |                  |                   | 15               |                       |                   | 5                 |
| 44  | 80                                                                    | —            | 7            |                      |                  |                   | 3                |                       |                   | 10                |
| 45  | 55                                                                    | —            | 4            |                      |                  |                   | 1                |                       |                   | 40                |
| 46  | 70                                                                    | —            | 10           |                      |                  |                   | 5                |                       |                   | 15                |
| 47  | 55                                                                    | —            | 4            | 1                    |                  |                   |                  |                       |                   | 40                |
| 48  | 70                                                                    | —            | 10           | 5                    |                  |                   |                  |                       |                   | 15                |
| 49  | 55                                                                    | —            | 4            |                      | 1                |                   |                  |                       |                   | 40                |
| 50  | 70                                                                    | —            | 10           |                      | 5                |                   |                  |                       |                   | 15                |
| 51  | 70                                                                    | —            | 10           |                      | 2.5              |                   | 2.5              | 10                    |                   | 5                 |
| 52  | 70                                                                    | —            | 10           | 2                    | 2                | 1                 |                  | 5                     |                   | 5                 |
| 53  | (Nb <sub>1.0</sub> Ta <sub>1.0</sub> )Mo <sub>3</sub> O <sub>14</sub> | 80           | 7            | 1                    | 1                | 0.5               | 0.5              | 3                     | 3                 | 2                 |
| 54  | Nb <sub>2</sub> Mo <sub>3</sub> O <sub>14</sub> 40                    | —            | 7            | 1                    | 1                | 0.5               | 0.5              | 3                     | 3                 | 2                 |
|     | Ta <sub>2</sub> Mo <sub>3</sub> O <sub>14</sub> 40                    |              |              |                      |                  |                   |                  |                       |                   |                   |

TABLE 8

| Nos | Molybdate<br>MnMoO <sub>4</sub><br>(wt. %) | Composition  |              |                      |                  |                   |                  | Carbonates<br>(wt. %) |                   |                   |
|-----|--------------------------------------------|--------------|--------------|----------------------|------------------|-------------------|------------------|-----------------------|-------------------|-------------------|
|     |                                            | Glass        |              | Fluorides<br>(wt. %) |                  | SrCO <sub>3</sub> |                  |                       | BaCO <sub>3</sub> |                   |
|     |                                            | A<br>(wt. %) | B<br>(wt. %) | SrF <sub>2</sub>     | BaF <sub>2</sub> | MgF <sub>2</sub>  | CaF <sub>2</sub> |                       |                   | MgCO <sub>3</sub> |
| 1   | 41.7                                       | 41.7         | —            |                      |                  |                   | 8.3              | 8.3                   |                   |                   |
| 2   | 54.2                                       | 29.2         | —            |                      |                  |                   | 8.3              | 8.3                   |                   |                   |
| 3   | 66.7                                       | 16.7         | —            |                      |                  |                   | 8.3              | 8.3                   |                   |                   |
| 4   | 80                                         | 3.4          | —            |                      |                  |                   | 8.3              | 8.3                   |                   |                   |
| 5   | 41.7                                       | —            | 41.7         |                      |                  |                   | 8.3              | 8.3                   |                   |                   |
| 6   | 54.2                                       | —            | 29.2         |                      |                  |                   | 8.3              | 8.3                   |                   |                   |
| 7   | 66.7                                       | —            | 16.7         |                      |                  |                   | 8.3              | 8.3                   |                   |                   |
| 8   | 80                                         | —            | 3.4          |                      |                  |                   | 8.3              | 8.3                   |                   |                   |
| 9   | 66.8                                       | 8.3          | 8.3          |                      |                  |                   | 8.3              | 8.3                   |                   |                   |
| 10  | 65                                         | —            | 34           |                      | 0.5              |                   |                  | 0.5                   |                   |                   |
| 11  | 65                                         | —            | 5            |                      | 5                |                   |                  | 25                    |                   |                   |
| 12  | 75                                         | —            | 10           |                      | 5                |                   |                  | 10                    |                   |                   |
| 13  | 75                                         | —            | 5            |                      | 15               |                   |                  | 5                     |                   |                   |
| 14  | 85                                         | —            | 7            |                      | 3                |                   |                  | 5                     |                   |                   |
| 15  | 95                                         | —            | 4            |                      | 0.5              |                   |                  | 0.5                   |                   |                   |
| 16  | 65                                         | —            | 34           |                      |                  | 0.5               |                  |                       | 0.5               |                   |
| 17  | 65                                         | —            | 5            |                      |                  | 5                 |                  |                       | 25                |                   |
| 18  | 75                                         | —            | 10           |                      |                  | 5                 |                  |                       | 10                |                   |
| 19  | 75                                         | —            | 5            |                      |                  | 15                |                  |                       | 5                 |                   |
| 20  | 85                                         | —            | 7            |                      |                  | 3                 |                  |                       | 5                 |                   |
| 21  | 95                                         | —            | 4            |                      |                  | 0.5               |                  |                       | 0.5               |                   |
| 22  | 75                                         | —            | 10           |                      | 5                |                   |                  |                       | 10                |                   |
| 23  | 85                                         | —            | 7            |                      | 3                |                   |                  |                       | 5                 |                   |
| 24  | 75                                         | —            | 10           |                      | 5                |                   |                  |                       |                   | 10                |
| 25  | 85                                         | —            | 7            |                      | 3                |                   |                  |                       |                   | 5                 |
| 26  | 75                                         | —            | 10           |                      | 5                |                   |                  |                       | 10                |                   |
| 27  | 85                                         | —            | 7            |                      | 3                |                   |                  |                       | 5                 |                   |
| 28  | 75                                         | —            | 5            |                      |                  | 15                |                  |                       | 5                 |                   |
| 29  | 85                                         | —            | 7            |                      |                  | 3                 |                  |                       | 5                 |                   |
| 30  | 75                                         | —            | 5            | 15                   |                  |                   |                  |                       |                   |                   |
| 31  | 85                                         | —            | 7            | 3                    |                  |                   |                  |                       |                   |                   |
| 32  | 75                                         | —            | 5            |                      | 15               |                   |                  |                       |                   |                   |
| 33  | 85                                         | —            | 7            | 3                    |                  |                   |                  |                       |                   |                   |
| 34  | 65                                         | —            | 5            |                      | 5                |                   |                  |                       | 15                |                   |
| 35  | 65                                         | —            | 5            | 2.5                  |                  | 2.5               | 15               |                       | 10                |                   |
| 36  | 65                                         | —            | 7            | 1                    | 1                | 1                 | 10               |                       | 5                 | 10                |

TABLE 9

| Nos | A                          | B                          | C                                        | D                                                       | E | F | G | Glass |   |                          |                           |
|-----|----------------------------|----------------------------|------------------------------------------|---------------------------------------------------------|---|---|---|-------|---|--------------------------|---------------------------|
|     |                            |                            |                                          |                                                         |   |   |   | A     | B | Fluorides                | Carbonates                |
| 1   | MgMoO <sub>4</sub><br>24.7 | ZnMoO <sub>4</sub><br>24.8 |                                          |                                                         |   |   |   | 49.5  |   | MgF <sub>2</sub><br>0.5  | MgCO <sub>3</sub><br>0.5  |
| 2   | CaMoO <sub>4</sub><br>25.0 |                            | Y <sub>6</sub> MoO <sub>12</sub><br>25.0 |                                                         |   |   |   | 33.3  |   | MgF <sub>2</sub><br>8.3  | MgCO <sub>3</sub><br>8.3  |
| 3   | SrMoO <sub>4</sub><br>25.0 |                            |                                          | Al <sub>2</sub> Mo <sub>3</sub> O <sub>12</sub><br>25.0 |   |   |   | 21.4  |   | MgF <sub>2</sub><br>14.3 | MgCO <sub>3</sub><br>14.3 |

TABLE 9-continued

(Ex. 1-plural Groups)

| Nos | A                                               | B                                               | C                                               | D                                               | E                                               | F                                               | G                  | Glass |      | Flourides        | Carbonates        |
|-----|-------------------------------------------------|-------------------------------------------------|-------------------------------------------------|-------------------------------------------------|-------------------------------------------------|-------------------------------------------------|--------------------|-------|------|------------------|-------------------|
|     |                                                 |                                                 |                                                 |                                                 |                                                 |                                                 |                    | A     | B    |                  |                   |
| 4   | BaMoO <sub>4</sub>                              |                                                 |                                                 |                                                 | ZrMo <sub>2</sub> O <sub>8</sub>                |                                                 |                    |       |      | MgF <sub>2</sub> | MgCo <sub>3</sub> |
|     | 25.0                                            |                                                 |                                                 |                                                 | 25.0                                            |                                                 |                    | 12.5  |      | 18.7             | 18.8              |
| 5   | Mg <sub>2</sub> Mo <sub>3</sub> O <sub>11</sub> |                                                 |                                                 |                                                 |                                                 | Nb <sub>2</sub> Mo <sub>3</sub> O <sub>14</sub> |                    |       |      | MgF <sub>2</sub> | MgCo <sub>3</sub> |
|     | 24.2                                            |                                                 |                                                 |                                                 |                                                 | 24.2                                            |                    | 5.4   |      | 23.1             | 23.1              |
| 6   | Ca <sub>3</sub> MoO <sub>6</sub>                |                                                 |                                                 |                                                 |                                                 |                                                 | MnMoO <sub>4</sub> |       |      | CaF <sub>2</sub> | MgCo <sub>3</sub> |
|     | 47.5                                            |                                                 |                                                 |                                                 |                                                 |                                                 | 47.5               | 4.0   |      | 0.5              | 0.5               |
| 7   |                                                 | ZnMo <sub>2</sub> O <sub>7</sub>                | La <sub>2</sub> Mo <sub>2</sub> O <sub>4</sub>  |                                                 |                                                 |                                                 |                    |       | 45.3 | CaF <sub>2</sub> | CaCo <sub>3</sub> |
|     |                                                 | 22.6                                            | 22.6                                            |                                                 |                                                 |                                                 |                    |       |      | 9.0              | 0.5               |
| 8   |                                                 | Zn <sub>3</sub> Mo <sub>2</sub> O <sub>9</sub>  |                                                 | Al <sub>2</sub> Mo <sub>3</sub> O <sub>12</sub> |                                                 |                                                 |                    |       |      | CaF <sub>2</sub> | CaCo <sub>3</sub> |
|     |                                                 | 23.1                                            |                                                 | 23.1                                            |                                                 |                                                 |                    |       |      | 15.4             | 7.6               |
| 9   |                                                 | ZnMoO <sub>4</sub>                              |                                                 |                                                 | HfMo <sub>2</sub> O <sub>8</sub>                |                                                 |                    |       |      | CaF <sub>2</sub> | CaCo <sub>3</sub> |
|     |                                                 | 23.3                                            |                                                 |                                                 | 23.3                                            |                                                 |                    |       |      | 20.0             | 13.4              |
| 10  |                                                 | ZnMo <sub>2</sub> O <sub>7</sub>                |                                                 |                                                 |                                                 | Ta <sub>2</sub> Mo <sub>3</sub> O <sub>14</sub> |                    |       |      | CaF <sub>2</sub> | CaCo <sub>3</sub> |
|     |                                                 | 23.1                                            |                                                 |                                                 |                                                 | 23.1                                            |                    | 11.6  |      | 24.9             | 17.3              |
| 11  |                                                 | Zn <sub>3</sub> Mo <sub>2</sub> O <sub>9</sub>  |                                                 |                                                 |                                                 |                                                 | MnMoO <sub>4</sub> |       |      | SrF <sub>2</sub> | CaCo <sub>3</sub> |
|     |                                                 | 32.0                                            |                                                 |                                                 |                                                 |                                                 | 32.0               | 7.1   |      | 0.4              | 28.5              |
| 12  |                                                 | CeMo <sub>2</sub> O <sub>8</sub>                | Al <sub>2</sub> Mo <sub>3</sub> O <sub>12</sub> |                                                 |                                                 |                                                 |                    |       |      | SrF <sub>2</sub> | CaCo <sub>3</sub> |
|     |                                                 | 30.0                                            | 30.0                                            |                                                 |                                                 |                                                 |                    |       |      | 6.3              | 31.2              |
| 13  |                                                 | Pr <sub>2</sub> MoO <sub>6</sub>                |                                                 | ZrMoO <sub>8</sub>                              |                                                 |                                                 |                    |       |      | SrF <sub>2</sub> | SrCo <sub>3</sub> |
|     |                                                 | 20.7                                            |                                                 | 20.7                                            |                                                 |                                                 |                    |       |      | 16.6             | 0.5               |
| 14  |                                                 | Nd <sub>2</sub> Mo <sub>3</sub> O <sub>12</sub> |                                                 |                                                 | Nb <sub>2</sub> Mo <sub>3</sub> O <sub>14</sub> |                                                 |                    |       |      | SrF <sub>2</sub> | SrCo <sub>3</sub> |
|     |                                                 | 21.4                                            |                                                 |                                                 | 21.4                                            |                                                 |                    |       |      | 21.4             | 7.2               |
| 15  |                                                 | Sm <sub>6</sub> MoO <sub>12</sub>               |                                                 |                                                 |                                                 | MnMoO <sub>4</sub>                              |                    |       |      | SrF <sub>2</sub> | SrCo <sub>3</sub> |
|     |                                                 | 21.5                                            |                                                 |                                                 |                                                 | 21.5                                            | 18.4               |       |      | 26.4             | 12.3              |
| 16  |                                                 |                                                 | Al <sub>2</sub> Mo <sub>3</sub> O <sub>12</sub> | HfMo <sub>2</sub> O <sub>8</sub>                |                                                 |                                                 |                    |       |      | BaF <sub>2</sub> | SrCo <sub>3</sub> |
|     |                                                 |                                                 | 30.7                                            | 30.7                                            |                                                 |                                                 |                    |       |      | 0.4              | 22.9              |
| 17  |                                                 |                                                 | Al <sub>2</sub> Mo <sub>3</sub> O <sub>12</sub> |                                                 | Ta <sub>2</sub> Mo <sub>3</sub> O <sub>14</sub> |                                                 |                    |       |      | BaF <sub>2</sub> | SrCo <sub>3</sub> |
|     |                                                 |                                                 | 30.0                                            |                                                 | 30.0                                            |                                                 |                    |       |      | 6.7              | 26.6              |
| 18  |                                                 |                                                 | Al <sub>2</sub> Mo <sub>3</sub> O <sub>12</sub> |                                                 |                                                 | MnMoO <sub>4</sub>                              |                    |       |      | BaF <sub>2</sub> | SrCo <sub>3</sub> |
|     |                                                 |                                                 | 28.2                                            |                                                 |                                                 | 28.2                                            | 2.4                |       |      | 11.8             | 29.4              |
| 19  |                                                 |                                                 |                                                 | ZrMo <sub>2</sub> O <sub>8</sub>                | Nb <sub>2</sub> Mo <sub>3</sub> O <sub>14</sub> |                                                 |                    |       |      | BaF <sub>2</sub> | BaCo <sub>3</sub> |
|     |                                                 |                                                 |                                                 | 19.2                                            | 19.2                                            |                                                 |                    |       |      | 22.9             | 0.4               |
| 20  |                                                 |                                                 |                                                 | HfMo <sub>2</sub> O <sub>8</sub>                |                                                 | MnMoO <sub>4</sub>                              |                    |       |      | BaF <sub>2</sub> | BaCo <sub>3</sub> |
|     |                                                 |                                                 |                                                 | 19.6                                            |                                                 | 19.6                                            | 26.1               |       |      | 18.1             | 6.6               |
| 21  |                                                 |                                                 |                                                 |                                                 | Ta <sub>2</sub> Mo <sub>3</sub> O <sub>14</sub> | MnMoO <sub>4</sub>                              |                    |       |      | MgF <sub>2</sub> | BaCo <sub>3</sub> |
|     |                                                 |                                                 |                                                 |                                                 | 29.0                                            | 29.0                                            | 24.9               |       |      | 0.4              | 16.7              |
| 22  | Sr <sub>3</sub> MoO <sub>6</sub>                | ZnMoO <sub>4</sub>                              | Eu <sub>2</sub> Mo <sub>2</sub> O <sub>7</sub>  |                                                 |                                                 |                                                 |                    |       |      | MgF <sub>2</sub> | BaCo <sub>3</sub> |
|     | 28.6                                            | 14.3                                            | 14.3                                            |                                                 |                                                 |                                                 |                    |       |      | 7.1              | 21.4              |
| 23  | BaMo <sub>2</sub> O <sub>7</sub>                | ZnMo <sub>2</sub> O <sub>7</sub>                |                                                 | Al <sub>2</sub> Mo <sub>3</sub> O <sub>12</sub> |                                                 |                                                 |                    |       |      | MgF <sub>2</sub> | BaCo <sub>3</sub> |
|     | 18.8                                            | 18.8                                            |                                                 | 18.8                                            |                                                 |                                                 |                    |       |      | 12.5             | 25.0              |
| 24  | Ba <sub>2</sub> MoO <sub>6</sub>                | Zn <sub>3</sub> Mo <sub>2</sub> O <sub>9</sub>  |                                                 |                                                 | ZrMo <sub>2</sub> O <sub>8</sub>                |                                                 |                    |       |      | MgF <sub>2</sub> | BaCo <sub>3</sub> |
|     | 22.2                                            | 22.2                                            |                                                 |                                                 | 8.9                                             |                                                 |                    |       |      | 16.7             | 27.8              |
| 25  | MgMoO <sub>4</sub>                              | ZnMoO <sub>4</sub>                              |                                                 |                                                 |                                                 | Nb <sub>2</sub> Mo <sub>3</sub> O <sub>14</sub> |                    |       |      | MgF <sub>2</sub> | MgCo <sub>3</sub> |
|     | 13.9                                            | 7.0                                             |                                                 |                                                 |                                                 | 13.9                                            |                    |       |      | 30.0             | 0.4               |
| 26  | CaNoO <sub>4</sub>                              | ZnMo <sub>2</sub> O <sub>7</sub>                |                                                 |                                                 |                                                 | MnMoO <sub>4</sub>                              |                    |       |      | CaF <sub>2</sub> | MgCo <sub>3</sub> |
|     | 18.1                                            | 18.1                                            |                                                 |                                                 |                                                 | 18.1                                            | 36.2               |       |      | 0.5              | 9.0               |
| 27  | SrMoO <sub>4</sub>                              |                                                 | Gd <sub>6</sub> MoO <sub>12</sub>               | Al <sub>2</sub> Mo <sub>3</sub> O <sub>12</sub> |                                                 |                                                 |                    |       |      | CaF <sub>2</sub> | MgCo <sub>3</sub> |
|     | 7.7                                             |                                                 | 23.1                                            | 23.1                                            |                                                 |                                                 |                    |       |      | 7.7              | 15.3              |
| 28  | BaMo <sub>4</sub> O <sub>13</sub>               |                                                 | Tb <sub>2</sub> Mo <sub>3</sub> O <sub>12</sub> |                                                 | HfMo <sub>2</sub> O <sub>8</sub>                |                                                 |                    |       |      | CaF <sub>2</sub> | MgCo <sub>3</sub> |
|     | 13.3                                            |                                                 | 26.7                                            |                                                 | 13.3                                            |                                                 |                    |       |      | 13.4             | 20.0              |
| 29  | Mg <sub>2</sub> Mo <sub>3</sub> O <sub>11</sub> |                                                 | Dy <sub>2</sub> MoO <sub>6</sub>                |                                                 |                                                 | Ta <sub>2</sub> Mo <sub>3</sub> O <sub>14</sub> |                    |       |      | CaF <sub>2</sub> | MgCo <sub>3</sub> |
|     | 23.5                                            |                                                 | 23.5                                            |                                                 |                                                 | 5.9                                             |                    |       |      | 17.6             | 23.6              |
| 30  | Ca <sub>3</sub> MoO <sub>12</sub>               |                                                 | HO <sub>6</sub> MoO <sub>12</sub>               |                                                 |                                                 | MnMoO <sub>4</sub>                              |                    |       |      | CaF <sub>2</sub> | MgCo <sub>3</sub> |
|     | 8.3                                             |                                                 | 20.7                                            |                                                 |                                                 | 20.7                                            | 2.1                |       |      | 22.3             | 25.9              |
| 31  | Sr <sub>3</sub> MoO <sub>6</sub>                |                                                 | Al <sub>2</sub> Mo <sub>3</sub> O <sub>12</sub> | ZrMo <sub>2</sub> O <sub>8</sub>                |                                                 |                                                 |                    |       |      | SrF <sub>2</sub> | CaCo <sub>3</sub> |
|     | 9.9                                             |                                                 | 29.7                                            | 9.9                                             |                                                 |                                                 |                    |       |      | 0.5              | 0.5               |
| 32  | BaMo <sub>7</sub> O <sub>24</sub>               |                                                 | Al <sub>2</sub> Mo <sub>3</sub> O <sub>12</sub> |                                                 | Nb <sub>2</sub> Mo <sub>3</sub> O <sub>14</sub> |                                                 |                    |       |      | SrF <sub>2</sub> | CaCo <sub>3</sub> |
|     | 8.3                                             |                                                 | 25.0                                            |                                                 | 16.7                                            |                                                 |                    |       |      | 8.3              | 8.4               |
| 33  | MgMoO <sub>4</sub>                              |                                                 | Al <sub>2</sub> Mo <sub>3</sub> O <sub>12</sub> |                                                 |                                                 | MnMoO <sub>4</sub>                              |                    |       |      | SrF <sub>2</sub> | CaCo <sub>3</sub> |
|     | 14.3                                            |                                                 | 14.3                                            |                                                 |                                                 | 21.4                                            | 21.4               |       |      | 14.3             | 14.3              |
| 34  | CaMoO <sub>4</sub>                              |                                                 | HfMo <sub>2</sub> O <sub>8</sub>                | Ta <sub>2</sub> Mo <sub>3</sub> O <sub>14</sub> |                                                 |                                                 |                    |       |      | SrF <sub>2</sub> | CaCo <sub>3</sub> |
|     | 25.0                                            |                                                 | 12.5                                            | 12.5                                            |                                                 |                                                 |                    |       |      | 18.7             | 18.8              |
| 35  | SrMoO <sub>4</sub>                              |                                                 | ZrMo <sub>2</sub> O <sub>8</sub>                |                                                 | MnMoO <sub>4</sub>                              |                                                 |                    |       |      | SrF <sub>2</sub> | CaCo <sub>3</sub> |
|     | 16.4                                            |                                                 | 16.4                                            |                                                 | 16.4                                            |                                                 | 5.5                |       |      | 23.5             | 21.8              |
| 36  | BaMoO <sub>4</sub>                              |                                                 |                                                 | Nb <sub>2</sub> Mo <sub>3</sub> O <sub>14</sub> | MnMoO <sub>4</sub>                              |                                                 |                    |       |      | 04970027-06206   | CaCo <sub>3</sub> |
|     |                                                 |                                                 |                                                 |                                                 |                                                 |                                                 |                    |       |      | BaF <sub>2</sub> |                   |
|     | 26.6                                            |                                                 |                                                 |                                                 |                                                 |                                                 |                    |       |      | 0.3              | 33.2              |
| 37  |                                                 | Zn <sub>3</sub> Mo <sub>2</sub> O <sub>9</sub>  | Er <sub>2</sub> MoO <sub>6</sub>                | Al <sub>2</sub> Mo <sub>3</sub> O <sub>12</sub> |                                                 |                                                 |                    |       |      | BaF <sub>2</sub> | SrCo <sub>3</sub> |
|     |                                                 | 18.1                                            | 18.1                                            | 9.0                                             |                                                 |                                                 |                    |       |      | 9.0              | 0.5               |
| 38  |                                                 | ZnMoO <sub>4</sub>                              | Tm <sub>6</sub> MoO <sub>12</sub>               |                                                 | HfMo <sub>2</sub> O <sub>8</sub>                |                                                 |                    |       |      | BaF <sub>2</sub> | SrCo <sub>3</sub> |
|     |                                                 | 7.7                                             | 23.1                                            |                                                 | 1.54                                            |                                                 |                    |       |      | 15.3             | 7.7               |
| 39  |                                                 | ZnMo <sub>2</sub> O <sub>7</sub>                | Yb <sub>2</sub> Mo <sub>4</sub> O <sub>15</sub> |                                                 |                                                 | Ta <sub>2</sub> Mo <sub>3</sub> O <sub>14</sub> |                    |       |      | BaF <sub>2</sub> | SrCo <sub>3</sub> |
|     |                                                 | 6.7                                             | 13.3                                            |                                                 |                                                 | 26.7                                            |                    |       |      | 20.0             | 13.3              |
| 40  |                                                 | Zn <sub>3</sub> Mo <sub>2</sub> O <sub>9</sub>  | Lu <sub>2</sub> Mo <sub>3</sub> O <sub>12</sub> |                                                 |                                                 | MnMoO <sub>4</sub>                              |                    |       |      | BaF <sub>2</sub> | SrCo <sub>3</sub> |
|     |                                                 | 12.3                                            | 12.3                                            |                                                 |                                                 | 11.6                                            |                    |       |      | 24.9             | 17.3              |
| 41  |                                                 | ZnMoO <sub>4</sub>                              |                                                 | Al <sub>2</sub> Mo <sub>3</sub> O <sub>12</sub> | ZrMo <sub>2</sub> O <sub>8</sub>                |                                                 |                    |       |      | MgF <sub>2</sub> | SrCo <sub>3</sub> |
|     |                                                 | 28.5                                            |                                                 | 28.5                                            | 7.1                                             |                                                 |                    |       |      | 7.1              | 28.4              |

TABLE 9-continued

(Ex. 1-plural Groups)

| Nos | A                                               | B                                               | C                                               | D                                               | E                                               | F                                               | G                  | Glass |     | Fluorides        | Carbonates        |
|-----|-------------------------------------------------|-------------------------------------------------|-------------------------------------------------|-------------------------------------------------|-------------------------------------------------|-------------------------------------------------|--------------------|-------|-----|------------------|-------------------|
|     |                                                 |                                                 |                                                 |                                                 |                                                 |                                                 |                    | A     | B   |                  |                   |
| 42  |                                                 | ZnMo <sub>2</sub> O <sub>7</sub>                |                                                 | Al <sub>2</sub> Mo <sub>3</sub> O <sub>12</sub> |                                                 | Nb <sub>2</sub> Mo <sub>3</sub> O <sub>14</sub> |                    |       | 2.5 | MgF <sub>2</sub> | SrCo <sub>3</sub> |
|     |                                                 | 25.0                                            |                                                 | 18.8                                            |                                                 | 16.2                                            |                    |       |     | 6.3              | 31.2              |
| 43  |                                                 | Zn <sub>3</sub> Mo <sub>2</sub> O <sub>9</sub>  |                                                 | Al <sub>2</sub> Mo <sub>3</sub> O <sub>12</sub> |                                                 |                                                 | MnMoO <sub>4</sub> |       |     | MgF <sub>2</sub> | BaCo <sub>3</sub> |
|     |                                                 | 16.6                                            |                                                 | 16.6                                            |                                                 |                                                 | 8.2                |       |     | 16.6             | 0.5               |
| 44  |                                                 | ZnMoO <sub>4</sub>                              |                                                 |                                                 | HfMo <sub>2</sub> O <sub>8</sub>                | Ta <sub>2</sub> Mo <sub>3</sub> O <sub>14</sub> |                    |       |     | MgF <sub>2</sub> | BaCo <sub>3</sub> |
|     |                                                 | 14.3                                            |                                                 |                                                 | 14.3                                            | 14.3                                            |                    |       |     | 21.4             | 7.1               |
| 45  |                                                 | ZnMo <sub>2</sub> O <sub>7</sub>                |                                                 |                                                 | ZrMo <sub>2</sub> O <sub>8</sub>                |                                                 | MnMoO <sub>4</sub> |       |     | MgF <sub>2</sub> | BaCo <sub>3</sub> |
|     |                                                 | 18.4                                            |                                                 |                                                 | 18.4                                            |                                                 | 6.1                |       |     | 26.4             | 12.3              |
| 46  |                                                 | Zn <sub>3</sub> Mo <sub>2</sub> O <sub>9</sub>  |                                                 |                                                 |                                                 | Nb <sub>2</sub> Mo <sub>3</sub> O <sub>14</sub> | MnMoO <sub>4</sub> |       |     | CaF <sub>2</sub> | BaCo <sub>3</sub> |
|     |                                                 | 23.0                                            |                                                 |                                                 |                                                 | 23.0                                            | 15.3               |       |     | 0.4              | 23.0              |
| 47  |                                                 |                                                 | Y <sub>2</sub> Mo <sub>3</sub> O <sub>12</sub>  | Al <sub>2</sub> Mo <sub>3</sub> O <sub>12</sub> | HfMo <sub>2</sub> O <sub>8</sub>                |                                                 |                    |       |     | CaF <sub>2</sub> | BaCo <sub>3</sub> |
|     |                                                 |                                                 | 6.7                                             | 26.7                                            | 26.7                                            |                                                 |                    |       |     | 6.7              | 26.5              |
| 48  |                                                 | La <sub>6</sub> MoO <sub>12</sub>               | Al <sub>2</sub> Mo <sub>3</sub> O <sub>12</sub> |                                                 |                                                 | Ta <sub>2</sub> Mo <sub>3</sub> O <sub>14</sub> |                    |       |     | CaF <sub>2</sub> | BaCo <sub>3</sub> |
|     |                                                 | 29.4                                            | 9.4                                             |                                                 |                                                 | 17.6                                            |                    |       |     | 2.4              | 29.4              |
| 49  |                                                 | Ce <sub>2</sub> Mo <sub>3</sub> O <sub>13</sub> | Al <sub>2</sub> Mo <sub>3</sub> O <sub>12</sub> |                                                 |                                                 |                                                 | MnMoO <sub>4</sub> |       |     | CaF <sub>2</sub> | MgCo <sub>3</sub> |
|     |                                                 | 23.0                                            | 7.7                                             |                                                 |                                                 |                                                 | 7.7                |       |     | 38.3             | 0.3               |
| 50  |                                                 | Pr <sub>2</sub> Mo <sub>3</sub> O <sub>12</sub> |                                                 | ZrMo <sub>2</sub> O <sub>8</sub>                |                                                 | Nb <sub>2</sub> Mo <sub>3</sub> O <sub>14</sub> |                    |       |     | CaF <sub>2</sub> | MgCo <sub>3</sub> |
|     |                                                 | 19.6                                            |                                                 | 13.1                                            |                                                 | 6.5                                             |                    |       |     | 22.1             | 6.6               |
| 51  |                                                 | Nd <sub>2</sub> MoO <sub>6</sub>                |                                                 | HfMo <sub>2</sub> O <sub>8</sub>                |                                                 |                                                 | MnMoO <sub>4</sub> |       |     | SrF <sub>2</sub> | MgCo <sub>3</sub> |
|     |                                                 | 24.9                                            |                                                 | 24.9                                            |                                                 |                                                 | 8.3                |       |     | 24.9             | 16.6              |
| 52  |                                                 | Sm <sub>3</sub> MoO <sub>12</sub>               |                                                 |                                                 |                                                 | Ta <sub>2</sub> Mo <sub>3</sub> O <sub>14</sub> | MnMoO <sub>4</sub> |       |     | SrF <sub>2</sub> | MgCo <sub>3</sub> |
|     |                                                 | 21.4                                            |                                                 |                                                 |                                                 | 28.6                                            | 7.1                |       |     | 14.3             | 21.5              |
| 53  |                                                 |                                                 | Al <sub>2</sub> Mo <sub>3</sub> O <sub>12</sub> | ZrMo <sub>2</sub> O <sub>8</sub>                |                                                 | Nb <sub>2</sub> Mo <sub>3</sub> O <sub>14</sub> |                    |       |     | SrF <sub>2</sub> | MgCo <sub>3</sub> |
|     |                                                 |                                                 | 18.7                                            | 18.7                                            |                                                 | 18.7                                            |                    |       |     | 6.3              | 25.0              |
| 54  |                                                 |                                                 | Al <sub>2</sub> Mo <sub>3</sub> O <sub>12</sub> | HfMo <sub>2</sub> O <sub>8</sub>                |                                                 |                                                 | MnMoO <sub>4</sub> |       |     | SrF <sub>2</sub> | MgCo <sub>3</sub> |
|     |                                                 |                                                 | 16.7                                            | 16.7                                            |                                                 |                                                 | 20.0               |       |     | 2.2              | 27.7              |
| 55  |                                                 |                                                 | Al <sub>2</sub> Mo <sub>3</sub> O <sub>12</sub> |                                                 | Ta <sub>2</sub> Mo <sub>3</sub> O <sub>14</sub> | MnMoO <sub>4</sub>                              |                    |       |     | SrF <sub>2</sub> | CaCo <sub>3</sub> |
|     |                                                 |                                                 | 7.0                                             |                                                 | 13.9                                            | 13.9                                            | 34.8               |       |     | 30.0             | 0.4               |
| 56  |                                                 |                                                 |                                                 | ZrMo <sub>2</sub> O <sub>8</sub>                | Nb <sub>2</sub> Mo <sub>3</sub> O <sub>14</sub> | MnMoO <sub>4</sub>                              |                    |       |     | BaF <sub>2</sub> | CaCo <sub>3</sub> |
|     |                                                 |                                                 |                                                 | 9.0                                             | 18.1                                            | 27.1                                            | 36.2               |       |     | 0.5              | 9.1               |
| 57  | Mg <sub>2</sub> Mo <sub>3</sub> O <sub>11</sub> | ZnMoO <sub>4</sub>                              | EuMoO <sub>4</sub>                              | Al <sub>2</sub> Mo <sub>3</sub> O <sub>12</sub> |                                                 |                                                 |                    |       |     | BaF <sub>2</sub> | CaCo <sub>3</sub> |
|     | 7.7                                             | 15.4                                            | 15.4                                            | 15.4                                            |                                                 |                                                 |                    |       |     | 23.1             | 15.3              |
| 58  | Ca <sub>3</sub> MoO <sub>6</sub>                | ZnMo <sub>2</sub> O <sub>7</sub>                | Gd <sub>2</sub> Mo <sub>6</sub> O <sub>21</sub> |                                                 | HfMo <sub>2</sub> O <sub>8</sub>                |                                                 |                    |       |     | BaF <sub>2</sub> | CaCo <sub>3</sub> |
|     | 13.3                                            | 13.3                                            | 13.3                                            |                                                 | 13.3                                            |                                                 |                    |       |     | 13.3             | 20.1              |
| 59  | Sr <sub>3</sub> MoO <sub>6</sub>                | Zn <sub>2</sub> Mo <sub>2</sub> O <sub>9</sub>  | Tb <sub>6</sub> MoO <sub>12</sub>               |                                                 |                                                 | Ta <sub>2</sub> Mo <sub>3</sub> O <sub>14</sub> |                    |       |     | BaF <sub>2</sub> | CaCo <sub>3</sub> |
|     | 8.8                                             | 8.8                                             | 17.6                                            |                                                 |                                                 | 17.6                                            |                    |       |     | 5.9              | 23.7              |
| 60  | Ba <sub>2</sub> MoO <sub>5</sub>                | ZnMoO <sub>4</sub>                              | Dy <sub>6</sub> MoO <sub>12</sub>               |                                                 |                                                 |                                                 | MnMoO <sub>4</sub> |       |     | BaF <sub>2</sub> | CaCo <sub>3</sub> |
|     | 15.5                                            | 15.5                                            | 15.5                                            |                                                 |                                                 |                                                 | 3.1                |       |     | 2.1              | 26.0              |
| 61  | MgMoO <sub>4</sub>                              | ZnMo <sub>2</sub> O <sub>7</sub>                |                                                 | Al <sub>2</sub> Mo <sub>3</sub> O <sub>12</sub> | ZrMo <sub>2</sub> O <sub>8</sub>                |                                                 |                    |       |     | MgF <sub>2</sub> | SrCo <sub>3</sub> |
|     | 10                                              | 10                                              |                                                 | 10                                              | 20                                              |                                                 |                    |       |     | 0.5              | 0.5               |
| 62  | CaMoO <sub>4</sub>                              | Zn <sub>3</sub> Mo <sub>2</sub> O <sub>9</sub>  |                                                 | Al <sub>2</sub> Mo <sub>3</sub> O <sub>12</sub> |                                                 | Nb <sub>2</sub> Mo <sub>3</sub> O <sub>14</sub> |                    |       |     | MgF <sub>2</sub> | SrCo <sub>3</sub> |
|     | 12.5                                            | 12.5                                            |                                                 | 12.5                                            |                                                 | 12.5                                            |                    |       |     | 8.3              | 8.4               |
| 63  | SrMoO <sub>4</sub>                              | ZnMoO <sub>4</sub>                              |                                                 | Al <sub>2</sub> Mo <sub>3</sub> O <sub>12</sub> |                                                 |                                                 | MnMoO <sub>4</sub> |       |     | MgF <sub>2</sub> | SrCo <sub>3</sub> |
|     | 14.3                                            | 1.43                                            |                                                 | 10.7                                            |                                                 |                                                 | 10.7               |       |     | 21.4             | 14.3              |
| 64  | BaMoO <sub>4</sub>                              | ZnMo <sub>2</sub> O <sub>7</sub>                |                                                 |                                                 | HfMo <sub>2</sub> O <sub>8</sub>                | Ta <sub>2</sub> Mo <sub>3</sub> O <sub>14</sub> |                    |       |     | MgF <sub>2</sub> | SrCo <sub>3</sub> |
|     | 9.4                                             | 15.6                                            |                                                 |                                                 | 15.6                                            | 9.4                                             |                    |       |     | 12.5             | 18.7              |
| 65  | Mg <sub>2</sub> Mo <sub>3</sub> O <sub>11</sub> | Zn <sub>3</sub> Mo <sub>2</sub> O <sub>9</sub>  |                                                 |                                                 | ZrMo <sub>2</sub> O <sub>8</sub>                |                                                 | MnMoO <sub>4</sub> |       |     | MgF <sub>2</sub> | SrCo <sub>3</sub> |
|     | 10.9                                            | 10.9                                            |                                                 |                                                 | 13.7                                            |                                                 | 13.7               |       |     | 5.5              | 21.8              |
| 66  | Ca <sub>3</sub> MoO <sub>3</sub>                | ZnMoO                                           |                                                 | Nb <sub>2</sub> Mo <sub>3</sub> O <sub>14</sub> | MnMoO <sub>4</sub>                              |                                                 |                    |       |     | CaF <sub>2</sub> | SrCo <sub>3</sub> |
|     | 15.9                                            | 15.9                                            |                                                 |                                                 |                                                 | 15.9                                            | 15.9               |       |     | 0.3              | 33.3              |
| 67  | Sr <sub>3</sub> MoO <sub>6</sub>                |                                                 | Ho <sub>2</sub> Mo <sub>3</sub> O <sub>12</sub> | Al <sub>2</sub> Mo <sub>3</sub> O <sub>12</sub> | HfMo <sub>2</sub> O <sub>8</sub>                |                                                 |                    |       |     | CaF <sub>2</sub> | BaCo <sub>3</sub> |
|     | 9.0                                             |                                                 | 13.6                                            | 13.6                                            | 9.0                                             |                                                 |                    |       |     | 9.0              | 0.5               |
| 68  | BaMo <sub>3</sub> O <sub>10</sub>               |                                                 | Er <sub>6</sub> MoO <sub>12</sub>               | Al <sub>2</sub> Mo <sub>3</sub> O <sub>12</sub> |                                                 | Ta <sub>2</sub> Mo <sub>3</sub> O <sub>14</sub> |                    |       |     | CaF <sub>2</sub> | BaCo <sub>3</sub> |
|     | 7.7                                             |                                                 | 15.4                                            | 7.7                                             |                                                 | 15.4                                            |                    |       |     | 30.8             | 7.6               |
| 69  | MgMoO <sub>4</sub>                              |                                                 | Tm <sub>2</sub> Mo <sub>6</sub> O <sub>12</sub> | Al <sub>2</sub> Mo <sub>3</sub> O <sub>12</sub> |                                                 |                                                 | MnMoO <sub>4</sub> |       |     | CaF <sub>2</sub> | BaCo <sub>3</sub> |
|     | 13.3                                            |                                                 | 10.0                                            | 10.0                                            |                                                 |                                                 | 13.3               |       |     | 20.0             | 13.4              |
| 70  | CaMoO <sub>4</sub>                              |                                                 | Yb <sub>6</sub> MoO <sub>12</sub>               |                                                 | ZrMo <sub>2</sub> O <sub>8</sub>                | Nb <sub>2</sub> Mo <sub>3</sub> O <sub>14</sub> |                    |       |     | CaF <sub>2</sub> | BaCo <sub>3</sub> |
|     | 17.3                                            |                                                 | 5.8                                             |                                                 | 17.3                                            | 5.8                                             |                    |       |     | 24.9             | 17.3              |
| 71  | SrMoO <sub>4</sub>                              |                                                 | Lu <sub>6</sub> MoO <sub>12</sub>               |                                                 | HfMo <sub>2</sub> O <sub>8</sub>                |                                                 | MnMoO <sub>4</sub> |       |     | SrF <sub>2</sub> | BaCo <sub>3</sub> |
|     | 17.8                                            |                                                 | 14.2                                            |                                                 | 17.8                                            |                                                 | 14.2               |       |     | 0.4              | 28.5              |
| 72  | BaMoO <sub>4</sub>                              |                                                 | Yb <sub>6</sub> MoO <sub>12</sub>               |                                                 |                                                 | Ta <sub>2</sub> Mo <sub>3</sub> O <sub>14</sub> | MnMoO <sub>4</sub> |       |     | SrF <sub>2</sub> | BaCo <sub>3</sub> |
|     | 18.7                                            |                                                 | 18.7                                            |                                                 |                                                 | 18.7                                            | 3.8                |       |     | 6.3              | 31.3              |
| 73  | Mg <sub>2</sub> Mo <sub>3</sub> O <sub>11</sub> |                                                 |                                                 | Al <sub>2</sub> Mo <sub>3</sub> O <sub>12</sub> | ZrMo <sub>2</sub> O <sub>8</sub>                | Nb <sub>2</sub> Mo <sub>3</sub> O <sub>14</sub> |                    |       |     | SrF <sub>2</sub> | MgCo <sub>3</sub> |
|     | 12.4                                            |                                                 |                                                 | 12.4                                            | 8.3                                             | 8.3                                             |                    |       |     | 16.7             | 0.4               |
| 74  | Ca <sub>3</sub> MoO <sub>6</sub>                |                                                 |                                                 | Al <sub>2</sub> Mo <sub>3</sub> O <sub>12</sub> | HfMo <sub>2</sub> O <sub>8</sub>                |                                                 | MnMoO <sub>4</sub> |       |     | SrF <sub>2</sub> | MgCo <sub>3</sub> |
|     | 7.1                                             |                                                 |                                                 | 14.3                                            | 14.3                                            |                                                 | 7.1                |       |     | 21.4             | 7.2               |
| 75  | Sr <sub>3</sub> MoO <sub>6</sub>                |                                                 |                                                 | Al <sub>2</sub> Mo <sub>3</sub> O <sub>12</sub> |                                                 | Ta <sub>2</sub> Mo <sub>3</sub> O <sub>14</sub> | MnMoO <sub>4</sub> |       |     | SrF <sub>2</sub> | MgCo <sub>3</sub> |
|     | 12.3                                            |                                                 |                                                 | 12.3                                            |                                                 | 9.2                                             | 9.2                |       |     | 26.4             | 12.2              |
| 76  | BaMo <sub>2</sub> O <sub>7</sub>                |                                                 |                                                 |                                                 | ZrMo <sub>2</sub> O <sub>8</sub>                | Nb <sub>2</sub> Mo <sub>3</sub> O <sub>14</sub> | MnMoO <sub>4</sub> |       |     | BaF <sub>2</sub> | MgCo <sub>3</sub> |
|     | 15.3                                            |                                                 |                                                 |                                                 | 15.3                                            | 15.3                                            | 15.3               |       |     | 0.4              | 23.1              |
| 77  | ZnMo <sub>2</sub> O <sub>7</sub>                | La <sub>2</sub> Mo <sub>3</sub> O <sub>12</sub> | Al <sub>2</sub> Mo <sub>3</sub> O <sub>12</sub> | HfMo <sub>2</sub> O <sub>8</sub>                |                                                 |                                                 |                    |       |     | BaF <sub>2</sub> | MgCo <sub>3</sub> |
|     | 13.3                                            | 6.7                                             | 20.0                                            | 20.0                                            |                                                 |                                                 |                    |       |     | 6.7              | 26.6              |
| 78  | Zn <sub>3</sub> Mo <sub>2</sub> O <sub>9</sub>  | Pr <sub>6</sub> MoO <sub>12</sub>               | Al <sub>2</sub> Mo <sub>3</sub> O <sub>12</sub> |                                                 | Ta <sub>2</sub> Mo <sub>3</sub> O <sub>14</sub> |                                                 |                    |       |     | BaF <sub>2</sub> | MgCo <sub>3</sub> |
|     | 8.8                                             | 14.7                                            | 20.6                                            |                                                 | 12.4                                            |                                                 |                    |       |     | 2.4              | 29.4              |
| 79  | ZnMoO <sub>4</sub>                              | Nd <sub>6</sub> MoO <sub>12</sub>               | Al <sub>2</sub> Mo <sub>3</sub> O <sub>12</sub> |                                                 |                                                 | MnMoO <sub>4</sub>                              |                    |       |     | BaF <sub>2</sub> | CaCo <sub>3</sub> |
|     | 7.7                                             | 7.7                                             | 7.7                                             |                                                 |                                                 | 15.3                                            |                    |       |     | 38.3             | 0.4               |
| 80  | ZnMo <sub>2</sub> O <sub>7</sub>                | Sm <sub>2</sub> Mo <sub>3</sub> O <sub>12</sub> |                                                 | ZrMo <sub>2</sub> O <sub>8</sub>                | Nb <sub>2</sub> Mo <sub>3</sub> O <sub>14</sub> |                                                 |                    |       |     | BaF <sub>2</sub> | CaCo <sub>3</sub> |
|     | 9.8                                             | 9.8                                             |                                                 | 9.8                                             | 9.8                                             |                                                 |                    |       |     | 26.1             | 6.6               |

TABLE 9-continued

(Ex. 1-plural Groups)

| Nos  | A                                               | B                                              | C                                               | D                                               | E                                | F                                               | G                  | Glass            |                   | Flourides | Carbonates |
|------|-------------------------------------------------|------------------------------------------------|-------------------------------------------------|-------------------------------------------------|----------------------------------|-------------------------------------------------|--------------------|------------------|-------------------|-----------|------------|
|      |                                                 |                                                |                                                 |                                                 |                                  |                                                 |                    | A                | B                 |           |            |
| 81   |                                                 | Zn <sub>3</sub> Mo <sub>2</sub> O <sub>9</sub> | Eu <sub>2</sub> MoO <sub>6</sub>                |                                                 | HfMo <sub>2</sub> O <sub>8</sub> |                                                 | MnMoO <sub>4</sub> | MgF <sub>2</sub> | CaCo <sub>3</sub> |           |            |
|      |                                                 | 12.4                                           | 16.6                                            |                                                 | 12.4                             |                                                 | 16.6               | 0.4              | 16.1              |           |            |
| 82   |                                                 | ZnMoO <sub>4</sub>                             | Gd <sub>2</sub> Mo <sub>3</sub> O <sub>12</sub> |                                                 |                                  | Ta <sub>2</sub> Mo <sub>3</sub> O <sub>14</sub> | MnMoO <sub>4</sub> | MgF <sub>2</sub> | CaCo <sub>3</sub> |           |            |
|      |                                                 | 14.3                                           | 14.3                                            |                                                 |                                  | 14.3                                            | 14.3               | 7.1              | 21.4              |           |            |
| 83   |                                                 | ZnMo <sub>2</sub> O <sub>7</sub>               |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> |                    | MgF <sub>2</sub> | CaCo <sub>3</sub> |           |            |
|      |                                                 | 15.6                                           |                                                 | 15.6                                            | 12.5                             | 12.5                                            |                    | 12.5             | 25.0              |           |            |
| 84   |                                                 | Zn <sub>3</sub> Mo <sub>2</sub> O <sub>9</sub> |                                                 | Al <sub>2</sub> Mo <sub>3</sub> O <sub>12</sub> | HfMo <sub>2</sub> O <sub>8</sub> |                                                 | MnMoO <sub>4</sub> | MgF <sub>2</sub> | CaCo <sub>3</sub> |           |            |
|      |                                                 | 13.3                                           |                                                 | 13.3                                            | 13.3                             |                                                 | 13.3               | 2.2              | 16.7              | 27.9      |            |
| 85   |                                                 | ZnMoO <sub>4</sub>                             |                                                 | Al <sub>2</sub> Mo <sub>3</sub> O <sub>12</sub> |                                  | Ta <sub>2</sub> Mo <sub>3</sub> O <sub>14</sub> | MnMoO <sub>4</sub> | MgF <sub>2</sub> | SrCo <sub>3</sub> |           |            |
|      |                                                 | 7.0                                            |                                                 | 7.0                                             |                                  | 7.0                                             | 13.9               | 34.8             | 30.0              | 0.3       |            |
| 86   |                                                 | ZnMo <sub>2</sub> O <sub>7</sub>               |                                                 |                                                 | ZrMo <sub>2</sub> O <sub>8</sub> | Nb <sub>2</sub> Mo <sub>3</sub> O <sub>14</sub> | MnMoO <sub>4</sub> | CaF <sub>2</sub> | SrCo <sub>3</sub> |           |            |
|      |                                                 | 13.6                                           |                                                 |                                                 | 13.6                             | 13.6                                            | 13.6               | 36.2             | 0.4               | 9.0       |            |
| 87   |                                                 |                                                | Tb <sub>2</sub> MoO <sub>6</sub>                | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> |                    | CaF <sub>2</sub> | SrCo <sub>3</sub> |           |            |
|      |                                                 |                                                | 11.5                                            | 15.4                                            | 11.5                             | 15.4                                            |                    | 7.7              | 15.4              |           |            |
| 88   |                                                 | Dy <sub>2</sub> MoO <sub>6</sub>               |                                                 | Al <sub>2</sub> Mo <sub>3</sub> O <sub>12</sub> | ZrMo <sub>2</sub> O <sub>8</sub> |                                                 | MnMoO <sub>4</sub> | CaF <sub>2</sub> | SrCo <sub>3</sub> |           |            |
|      |                                                 | 13.3                                           |                                                 | 13.3                                            | 13.3                             |                                                 | 13.3               | 13.3             | 13.4              | 20.1      |            |
| 89   |                                                 | Ho <sub>2</sub> MoO <sub>6</sub>               |                                                 | Al <sub>2</sub> Mo <sub>3</sub> O <sub>12</sub> |                                  | Nb <sub>2</sub> Mo <sub>3</sub> O <sub>14</sub> | MnMoO <sub>4</sub> | CaF <sub>2</sub> | SrCo <sub>3</sub> |           |            |
|      |                                                 | 11.8                                           |                                                 | 11.8                                            |                                  | 11.8                                            | 17.6               | 5.9              | 17.6              | 23.5      |            |
| 90   |                                                 | Er <sub>6</sub> MoO <sub>12</sub>              |                                                 |                                                 | HfMo <sub>2</sub> O <sub>8</sub> | Ta <sub>2</sub> Mo <sub>3</sub> O <sub>14</sub> | MnMoO <sub>4</sub> | CaF <sub>2</sub> | SrCo <sub>3</sub> |           |            |
|      |                                                 | 12.4                                           |                                                 |                                                 | 12.4                             | 12.4                                            | 12.4               | 2.0              | 22.4              | 26.0      |            |
| 91   |                                                 |                                                |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> | SrF <sub>2</sub> | BaCo <sub>3</sub> |           |            |
|      |                                                 |                                                |                                                 | 9.9                                             | 19.8                             | 9.9                                             | 9.9                | 0.5              | 0.5               |           |            |
| 92   | MgMoO <sub>4</sub>                              | Zn <sub>3</sub> Mo <sub>2</sub> O <sub>9</sub> | Tm <sub>3</sub> Mo <sub>2</sub> O <sub>12</sub> | Al <sub>2</sub> Mo <sub>3</sub> O <sub>12</sub> | HfMo <sub>2</sub> O <sub>8</sub> |                                                 |                    | SrF <sub>2</sub> | BaCo <sub>3</sub> |           |            |
| 8.3  |                                                 | 16.7                                           | 8.3                                             | 8.3                                             | 8.3                              |                                                 |                    | 8.3              | 8.4               |           |            |
| 93   | CaMoO <sub>4</sub>                              | ZaMoO <sub>4</sub>                             | Yb <sub>6</sub> MoO <sub>12</sub>               | Al <sub>2</sub> Mo <sub>3</sub> O <sub>12</sub> |                                  | Ta <sub>2</sub> Mo <sub>3</sub> O <sub>14</sub> |                    | SrF <sub>2</sub> | BaCo <sub>3</sub> |           |            |
| 7.1  |                                                 | 14.3                                           | 14.3                                            | 7.1                                             |                                  | 7.1                                             |                    | 14.3             | 14.3              |           |            |
| 94   | SrMoO <sub>4</sub>                              | ZnMo <sub>2</sub> O <sub>7</sub>               | Lu <sub>6</sub> MoO <sub>12</sub>               | Al <sub>2</sub> Mo <sub>3</sub> O <sub>12</sub> |                                  |                                                 | MnMoO <sub>4</sub> | SrF <sub>2</sub> | BaCo <sub>3</sub> |           |            |
| 12.5 |                                                 | 12.5                                           | 12.5                                            | 6.3                                             |                                  |                                                 | 6.3                | 12.5             | 18.7              | 18.7      |            |
| 95   | BaMoO <sub>4</sub>                              | Zn <sub>3</sub> Mo <sub>2</sub> O <sub>9</sub> | Y <sub>2</sub> Mo <sub>3</sub> O <sub>12</sub>  |                                                 | ZrMo <sub>2</sub> O <sub>8</sub> | Nb <sub>2</sub> Mo <sub>3</sub> O <sub>14</sub> |                    | SrF <sub>2</sub> | BaCo <sub>3</sub> |           |            |
| 10.9 |                                                 | 5.5                                            | 10.9                                            |                                                 | 10.9                             | 10.9                                            |                    | 23.5             | 21.9              |           |            |
| 96   | Mg <sub>2</sub> Mo <sub>3</sub> O <sub>11</sub> | ZnMoO <sub>4</sub>                             | La <sub>2</sub> MoO <sub>6</sub>                |                                                 | HfMo <sub>2</sub> O <sub>8</sub> |                                                 | MnMoO <sub>4</sub> | BaF <sub>2</sub> | BaCo <sub>3</sub> |           |            |
| 13.3 |                                                 | 10.6                                           | 13.3                                            |                                                 | 13.3                             | 13.3                                            |                    | 0.3              | 33.3              |           |            |
| 97   | Ca <sub>3</sub> MoO <sub>6</sub>                | ZnMo <sub>2</sub> O <sub>7</sub>               | Pr <sub>2</sub> Mo <sub>3</sub> O <sub>12</sub> |                                                 |                                  | Ta <sub>2</sub> Mo <sub>3</sub> O <sub>14</sub> | MnMoO <sub>4</sub> | BaF <sub>2</sub> | MgCo <sub>3</sub> |           |            |
| 9.0  |                                                 | 9.0                                            | 9.0                                             |                                                 |                                  | 9.0                                             | 9.0                | 9.2              | 0.5               |           |            |
| 98   | Sr <sub>3</sub> MoO <sub>6</sub>                | Zn <sub>3</sub> Mo <sub>2</sub> O <sub>9</sub> |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> |                    | BaF <sub>2</sub> | MgCo <sub>3</sub> |           |            |
| 7.7  |                                                 | 7.7                                            |                                                 | 15.4                                            | 7.7                              | 7.7                                             |                    | 15.4             | 7.6               |           |            |
| 99   | Ba <sub>3</sub> MoO <sub>6</sub>                | ZnMoO <sub>4</sub>                             |                                                 | Al <sub>2</sub> Mo <sub>3</sub> O <sub>12</sub> | HfMo <sub>2</sub> O <sub>8</sub> |                                                 | MnMoO <sub>4</sub> | BaF <sub>2</sub> | MgCo <sub>3</sub> |           |            |
| 6.7  |                                                 | 13.3                                           |                                                 | 13.3                                            | 6.7                              |                                                 | 6.7                | 20.0             | 13.3              |           |            |
| 100  | MgMoO <sub>4</sub>                              | ZnMo <sub>2</sub> O <sub>7</sub>               |                                                 | Al <sub>2</sub> Mo <sub>3</sub> O <sub>12</sub> |                                  | Ta <sub>2</sub> Mo <sub>3</sub> O <sub>14</sub> | MnMoO <sub>4</sub> | BaF <sub>2</sub> | MgCo <sub>3</sub> |           |            |
| 5.8  |                                                 | 11.6                                           |                                                 | 11.6                                            |                                  | 11.6                                            | 5.8                | 11.6             | 24.8              | 17.2      |            |
| 101  | CaMoO <sub>4</sub>                              | Zn <sub>3</sub> Mo <sub>2</sub> O <sub>9</sub> |                                                 |                                                 | ZrMo <sub>2</sub> O <sub>8</sub> | Nb <sub>2</sub> Mo <sub>3</sub> O <sub>14</sub> | MnMoO <sub>4</sub> | MgF <sub>2</sub> | MgCo <sub>3</sub> |           |            |
| 14.2 |                                                 | 14.2                                           |                                                 |                                                 | 14.2                             | 14.2                                            | 7.1                | 7.1              | 0.4               | 28.6      |            |
| 102  | SrMoO <sub>4</sub>                              |                                                | Ce <sub>6</sub> MoO <sub>12</sub>               | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> |                    | MgF <sub>2</sub> | MgCo <sub>3</sub> |           |            |
| 12.5 |                                                 | 12.5                                           | 12.5                                            | 12.5                                            | 12.5                             | 12.5                                            |                    | 6.2              | 31.3              |           |            |
| 103  | BaMoO <sub>4</sub>                              |                                                | Pr <sub>2</sub> MoO <sub>6</sub>                | Al <sub>2</sub> Mo <sub>3</sub> O <sub>12</sub> | ZrMo <sub>2</sub> O <sub>8</sub> |                                                 | MnMoO <sub>4</sub> | MgF <sub>2</sub> | CaCo <sub>3</sub> |           |            |
| 8.3  |                                                 | 8.3                                            | 8.3                                             | 8.3                                             | 8.3                              |                                                 | 8.3                | 41.5             | 16.6              | 0.4       |            |
| 104  | Mg <sub>2</sub> Mo <sub>3</sub> O <sub>11</sub> |                                                | Nd <sub>2</sub> Mo <sub>3</sub> O <sub>12</sub> | Al <sub>2</sub> Mo <sub>3</sub> O <sub>12</sub> |                                  | Nb <sub>2</sub> Mo <sub>3</sub> O <sub>14</sub> | MnMoO <sub>4</sub> | MgF <sub>2</sub> | CaCo <sub>3</sub> |           |            |
| 7.1  |                                                 | 7.1                                            | 7.1                                             | 7.1                                             |                                  | 7.1                                             | 14.3               | 28.6             | 21.5              | 7.7       |            |
| 105  | Ca <sub>3</sub> MoO <sub>6</sub>                |                                                | Sm <sub>2</sub> Mo <sub>2</sub> O <sub>7</sub>  |                                                 | HfMo <sub>2</sub> O <sub>8</sub> | Ta <sub>2</sub> Mo <sub>3</sub> O <sub>14</sub> | MnMoO <sub>4</sub> | MgF <sub>2</sub> | CaCo <sub>3</sub> |           |            |
| 6.1  |                                                 | 6.1                                            | 6.1                                             |                                                 | 6.1                              | 12.3                                            | 12.3               | 18.4             | 26.4              | 12.3      |            |
| 106  | Sr <sub>3</sub> MoO <sub>6</sub>                |                                                |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> | CaF <sub>2</sub> | CaCo <sub>3</sub> |           |            |
| 7.7  |                                                 |                                                |                                                 | 15.3                                            | 15.3                             | 15.3                                            | 7.7                | 15.3             | 0.4               | 23.0      |            |
| 107  |                                                 | ZnMoO <sub>4</sub>                             | Eu <sub>6</sub> MoO <sub>12</sub>               | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> |                    | CaF <sub>2</sub> | CaCo <sub>3</sub> |           |            |
|      |                                                 | 6.7                                            | 13.3                                            | 13.3                                            | 13.3                             | 13.3                                            |                    | 6.7              | 26.7              |           |            |
| 108  |                                                 | ZnMo <sub>2</sub> O <sub>7</sub>               | Gd <sub>2</sub> MoO <sub>6</sub>                | Al <sub>2</sub> Mo <sub>3</sub> O <sub>12</sub> | ZrMo <sub>2</sub> O <sub>8</sub> |                                                 | MnMoO <sub>4</sub> | CaF <sub>2</sub> | CaCo <sub>3</sub> |           |            |
|      |                                                 | 9.4                                            | 11.8                                            | 11.8                                            | 11.8                             | 11.8                                            |                    | 11.7             | 29.4              |           |            |
| 109  |                                                 | Zn <sub>3</sub> Mo <sub>2</sub> O <sub>9</sub> | Tb <sub>2</sub> Mo <sub>3</sub> O <sub>12</sub> | Al <sub>2</sub> Mo <sub>3</sub> O <sub>12</sub> |                                  | Nb <sub>2</sub> Mo <sub>3</sub> O <sub>14</sub> | MnMoO <sub>4</sub> | CaF <sub>2</sub> | SrCo <sub>3</sub> |           |            |
|      |                                                 | 7.7                                            | 7.7                                             | 7.7                                             |                                  | 7.7                                             | 7.7                | 30.3             | 22.9              | 0.3       |            |
| 110  |                                                 | ZnMoO <sub>4</sub>                             | Dy <sub>6</sub> MoO <sub>12</sub>               |                                                 | HfMo <sub>2</sub> O <sub>8</sub> | Ta <sub>2</sub> Mo <sub>3</sub> O <sub>14</sub> | MnMoO <sub>4</sub> | CaF <sub>2</sub> | SrCo <sub>3</sub> |           |            |
|      |                                                 | 6.5                                            | 13.1                                            |                                                 | 6.5                              | 6.5                                             | 6.5                | 26.2             | 28.1              | 6.6       |            |
| 111  |                                                 | ZnMo <sub>2</sub> O <sub>7</sub>               |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> | SrF <sub>2</sub> | SrCo <sub>3</sub> |           |            |
|      |                                                 | 16.6                                           |                                                 | 16.6                                            | 8.3                              | 8.3                                             | 8.3                | 24.9             | 0.4               | 16.6      |            |
| 112  |                                                 |                                                | Ho <sub>6</sub> MoO <sub>12</sub>               | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> | MnMoO <sub>4</sub> | SrF <sub>2</sub> | SrCo <sub>3</sub> |           |            |
|      |                                                 |                                                | 14.3                                            | 14.3                                            | 14.3                             | 7.1                                             | 7.1                | 7.1              | 21.5              |           |            |
| 113  | MgMoO <sub>4</sub>                              | Zn <sub>3</sub> Mo <sub>2</sub> O <sub>9</sub> | Er <sub>2</sub> MoO <sub>6</sub>                | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> |                    | SrF <sub>2</sub> | SrCo <sub>3</sub> |           |            |
| 6.3  |                                                 | 12.5                                           | 12.5                                            | 12.5                                            | 6.3                              | 6.3                                             |                    | 12.4             | 24.9              |           |            |
| 114  | CaMoO <sub>4</sub>                              | ZnMoO <sub>4</sub>                             | Tm <sub>2</sub> MoO <sub>6</sub>                | Al <sub>2</sub> Mo <sub>3</sub> O <sub>12</sub> | HfMo <sub>2</sub> O <sub>8</sub> |                                                 | MnMoO <sub>4</sub> | SrF <sub>2</sub> | SrCo <sub>3</sub> |           |            |
| 5.6  |                                                 | 11.1                                           | 11.1                                            | 20                                              | 8.9                              |                                                 | 9.6                | 2.2              | 16.7              | 27.7      |            |
| 115  | SrMoO <sub>4</sub>                              | ZnMo <sub>2</sub> O <sub>7</sub>               | Yb <sub>6</sub> MoO <sub>12</sub>               | Al <sub>2</sub> Mo <sub>3</sub> O <sub>12</sub> |                                  | Ta <sub>2</sub> Mo <sub>3</sub> O <sub>14</sub> | MnMoO <sub>4</sub> | SrF <sub>2</sub> | BaCo <sub>3</sub> |           |            |
| 3.5  |                                                 | 3.5                                            | 7.0                                             | 7.0                                             |                                  | 7.0                                             | 7.0                | 34.8             | 29.9              | 0.3       |            |
| 116  | BaMoO <sub>4</sub>                              | Zn <sub>3</sub> Mo <sub>2</sub> O <sub>9</sub> | Lu <sub>6</sub> MoO <sub>12</sub>               |                                                 | ZrMo <sub>2</sub> O <sub>8</sub> | Nb <sub>2</sub> Mo <sub>3</sub> O <sub>14</sub> | MnMoO <sub>4</sub> | BaF <sub>2</sub> | BaCo <sub>3</sub> |           |            |
| 9.0  |                                                 | 9.0                                            | 9.0                                             |                                                 | 9.0                              | 9.0                                             | 9.0                | 36.3             | 0.5               | 9.2       |            |
| 117  | Mg <sub>2</sub> Mo <sub>3</sub> O <sub>11</sub> | ZnMoO <sub>4</sub>                             |                                                 | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> | MnMoO <sub>4</sub> | BaF <sub>2</sub> | BaCo <sub>3</sub> |           |            |
| 15.4 |                                                 | 7.7                                            |                                                 | 7.7                                             | 7.7                              | 7.7                                             | 7.7                | 23.1             | 7.7               | 15.3      |            |
| 118  | Ca <sub>3</sub> MoO <sub>6</sub>                |                                                | Y <sub>2</sub> Mo <sub>3</sub> O <sub>12</sub>  | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> | BaF <sub>2</sub> | BaCo <sub>3</sub> |           |            |
| 13.3 |                                                 |                                                | 13.3                                            | 6.7                                             | 6.7                              | 6.7                                             | 6.7                | 13.3             | 13.3              | 20.0      |            |
| 119  |                                                 | ZnMo <sub>2</sub> O <sub>7</sub>               | La <sub>2</sub> MoO <sub>6</sub>                | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> | MnMoO <sub>4</sub> | BaF <sub>2</sub> | BaCo <sub>3</sub> |           |            |
|      |                                                 | 11.8                                           | 11.8                                            | 11.8                                            | 5.9                              | 5.9                                             | 5.9                | 5.8              | 17.6              | 23.5      |            |

TABLE 9-continued

(Ex. 1-plural Groups)

| Nos | A                                       | B                                                     | C                                     | D                                                      | E                                        | F                                                       | G                         | Glass |            | Flourides                | Carbonates                |
|-----|-----------------------------------------|-------------------------------------------------------|---------------------------------------|--------------------------------------------------------|------------------------------------------|---------------------------------------------------------|---------------------------|-------|------------|--------------------------|---------------------------|
|     |                                         |                                                       |                                       |                                                        |                                          |                                                         |                           | A.    | B          |                          |                           |
| 120 | Sr <sub>3</sub> MoO <sub>6</sub><br>5.2 | Zn <sub>3</sub> Mo <sub>2</sub> O <sub>9</sub><br>5.2 | Mo <sub>2</sub> O <sub>8</sub><br>5.2 | Al <sub>2</sub> Mo <sub>3</sub> O <sub>12</sub><br>9.2 | ZrMo <sub>2</sub> O <sub>8</sub><br>10.3 | Nb <sub>2</sub> Mo <sub>3</sub> O <sub>14</sub><br>10.3 | MnMoO <sub>4</sub><br>8.3 |       | BaF<br>2.1 | BaF <sub>2</sub><br>22.3 | BaCo <sub>3</sub><br>25.9 |

The respective samples of the aforesaid components were heat-treated at 1000° C. for 1 hour in a gaseous atmosphere consisting of 98.5% by volume of nitrogen (N<sub>2</sub>) and 1.5% by volume of hydrogen mill and dried to obtain the heat-treated resistor material powders having a particle size of 10 μm and composed of the glass, the molybdates of the corresponding elements and the fluorides of alkaline earth metals.

The respective samples were then mixed with the carbonates of alkaline earth metals in the proportions specified in the tables. After mixing 25 parts by weight of the organic vehicle (90 parts by weight of butyl carbitol plus 10 parts by weight of ethyl cellulose) were added to and mixed with 100 parts by weight of the resulting powdery mixtures in a ball mill to obtain the respective resistor material pastes.

On the other hand, 8 parts by weight of polyvinyl butyral, 8 parts by weight of diethyl phthalate, 0.5 parts by weight of oleic acid, 10 parts by weight of acetone, 20 parts by weight of isopropyl alcohol and 20 parts by weight of methyl ethyl ketone were added to and mixed with 100 parts by weight of ceramic material powders consisting of 40.0% by weight of Al<sub>2</sub>O<sub>3</sub>, 35.0% by weight of SiO<sub>2</sub>, 13.0% by weight of B<sub>2</sub>O<sub>3</sub>, 7.0% by weight of CaO and 5.0% by weight of MgO by means of a ball mill to prepare a slurry, which was defoamed. Thereafter, the slurry was formed by the doctor blade process into a long ceramic green sheet of 200 μm in thickness. Cut out of this ceramic green sheet were a green sheet piece of 9 mm×9 mm and a green sheet piece of 6 mm×9 mm.

As shown in FIG. 1, printed on the aforesaid green sheet 1 piece 1 of 9 mm×9 mm was a conductive material paste by means of screen printing, which was obtained by adding as the organic vehicle 20 parts by weight of butyl carbitol and 5 parts by weight of ethyl cellulose to 95 parts by weight of copper powders and 5 parts by weight of glass frit, followed by three-roll milling. The conductive paste printed ceramic green sheet piece 1 was dried at 125° C. for 10 minutes to form a conductive material film 2. Next, each of the aforesaid respective resistive material pastes was similarly screen-printed on the aforesaid green sheet piece 1 by the screen process, and was dried at 125° C. for 10 minutes to form a resistor material film 3 for a thick-film resistor.

Then, the aforesaid green sheet piece 4 of 6 mm×9 mm was laminated upon the green sheet piece 1, as shown by a chain dash, at 100° C. and 150 Kg/cm<sup>2</sup>. Subsequently, the laminated product was heated at 400° to 500° C. in an oxidizing atmosphere of, e.g., air to decompose and burn off the organics remaining in the green sheet pieces 1,4, the conductive film 2 and the resistive film 3.

After decomposing the organics in this manner, they were fired at 950° C. for 1 hour in a gaseous mixture consisting of 98.5% by volume of N<sub>2</sub> and 1.5% by volume of H<sub>2</sub> to obtain an integral multilayered ceramic board having a porcelain 1a formed of the sintered body

10 of the green sheet piece 1, a porcelain layer 4a formed of the sintered body of the green sheet piece 4, a thick-film conductor 2a, formed of the sintered body of the conductive film 2 and a thick-film resistor 3a formed of the sintered resistive film 3 located between the layers 1 and 4, as illustrated in FIG. 3. With regard to this multilayered ceramic board, such warping or swelling as shown in FIGS. 4 and 5 were not found, as will be described later.

The thus obtained multilayered ceramic board was 20 polished in its layer direction to expose the resistor layer to view, which was then analyzed by X-ray diffraction (Cu K alpha rays). The results of Sample No. 1 obtained are shown in FIG. 6, from which the presence of the molybdate of the corresponding element could be ascertained. FIG. 7 is also a TEM photograph taken of said sample, which shows the acicular particles that are the reduction product of the molybdate of magnesium. In the photograph, the molybdate of magnesium is shown by a black portion on the left side, and the glass is indicated by a gray portion on the upper side. It is to be noted that the sample, of which a TEM photograph was taken, was prepared by cutting the multilayered ceramic board in the sectional direction to a band of 200 μm in width, and polishing the band to a thickness of 30 about 20 μm, followed by thinning with an ion milling device. Although not illustrated and described, similar results could also be confirmed with respect to other samples.

Next, the resistance values (R<sub>25</sub>) and (R<sub>125</sub>) of the 40 thick-film resistor 3a at 25° C. and at the time when heated to 125° C. were measured with a digital multimeter, and the temperature coefficient of resistance (TCR) was calculated from the following equation:

$$TCR = \frac{R_{125} - R_{25}}{R_{25}} \times 10000 \text{ (ppm/}^{\circ}\text{C.)}$$

The measured resistance values R<sub>25</sub> and calculated 50 values TCR are shown in Table 10 for the compositions of Table 2 and, similarly, in Tables 11 to 17 for the compositions of Tables 3 to 9.

After the obtained multilayered ceramic board had been permitted to stand at 60° C. and a relative humidity of 95% for 1000 hours, its resistance at 25° C. was measured to determine the rate of change with respect to the resistance at 25° C. Just as mentioned above, the results are shown in the tables.

With resistor material samples obtained by removing the carbonates and fluorides of alkaline earth metals, 60 and by removing the former only from the aforesaid respective resistor material samples, multilayered ceramic boards were prepared and measured in the same manner as mentioned above. The results are set forth in Table 10 to 17 with the sample numbers corresponding to the sample numbers of the 1st column in the 2nd and 65 3rd columns of Tables 10 to 17.

TABLE 10

(Characteristic values corresponding to the sample in Table 2)

| Nos | Example 1                                         |               |                                  | Carbonate-Free                                    |               |                                  | Carbonate & Fluoride-Free                         |               |                                  |
|-----|---------------------------------------------------|---------------|----------------------------------|---------------------------------------------------|---------------|----------------------------------|---------------------------------------------------|---------------|----------------------------------|
|     | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) |
| 1   | 8.35 × 10 <sup>3</sup>                            | -286          | <±2                              | 22.6 × 10 <sup>3</sup>                            | -511          | <±2                              | 18.5 × 10 <sup>3</sup>                            | -831          | <±2                              |
| 2   | 5.28 × 10 <sup>3</sup>                            | -252          | "                                | 14.9 × 10 <sup>3</sup>                            | -496          | "                                | 9.24 × 10 <sup>3</sup>                            | -529          | "                                |
| 3   | 2.15 × 10 <sup>3</sup>                            | -192          | "                                | 72.3 × 10 <sup>3</sup>                            | -424          | "                                | 4.11 × 10 <sup>3</sup>                            | -508          | "                                |
| 4   | 1.02 × 10 <sup>3</sup>                            | -161          | "                                | 4.55 × 10 <sup>3</sup>                            | -326          | "                                | 2.36 × 10 <sup>3</sup>                            | -456          | "                                |
| 5   | 6.49 × 10 <sup>3</sup>                            | -274          | "                                | 13.8 × 10 <sup>3</sup>                            | -405          | "                                | 9.21 × 10 <sup>3</sup>                            | -530          | "                                |
| 6   | 1.58 × 10 <sup>3</sup>                            | -173          | "                                | 6.98 × 10 <sup>3</sup>                            | -369          | "                                | 4.07 × 10 <sup>3</sup>                            | -511          | "                                |
| 7   | 3.58 × 10 <sup>3</sup>                            | -248          | "                                | 10.2 × 10 <sup>3</sup>                            | -502          | "                                | 12.6 × 10 <sup>3</sup>                            | -542          | "                                |
| 8   | 2.73 × 10 <sup>3</sup>                            | -205          | "                                | 8.24 × 10 <sup>3</sup>                            | -498          | "                                | 2.03 × 10 <sup>3</sup>                            | -501          | "                                |
| 9   | 1.03 × 10 <sup>3</sup>                            | -168          | "                                | 7.44 × 10 <sup>3</sup>                            | -472          | "                                | 1.99 × 10 <sup>3</sup>                            | -499          | "                                |
| 10  | 1.18 × 10 <sup>3</sup>                            | -177          | "                                | 8.34 × 10 <sup>3</sup>                            | -499          | "                                | 4.07 × 10 <sup>3</sup>                            | -511          | "                                |
| 11  | 899                                               | -89           | "                                | 5.21 × 10 <sup>3</sup>                            | -470          | "                                | 2.03 × 10 <sup>3</sup>                            | -501          | "                                |
| 12  | 925                                               | -97           | "                                | 4.49 × 10 <sup>3</sup>                            | -462          | "                                | 1.97 × 10 <sup>3</sup>                            | -498          | "                                |
| 13  | 676                                               | -25           | "                                | 3.32 × 10 <sup>3</sup>                            | -454          | "                                | 3.12 × 10 <sup>3</sup>                            | -505          | "                                |
| 14  | 4.03 × 10 <sup>3</sup>                            | -270          | "                                | 11.5 × 10 <sup>3</sup>                            | -504          | "                                | 12.6 × 10 <sup>3</sup>                            | -542          | "                                |
| 15  | 2.88 × 10 <sup>3</sup>                            | -211          | "                                | 8.27 × 10 <sup>3</sup>                            | -498          | "                                | 2.03 × 10 <sup>3</sup>                            | -501          | "                                |
| 16  | 2.91 × 10 <sup>3</sup>                            | -218          | "                                | 7.98 × 10 <sup>3</sup>                            | -483          | "                                | 1.99 × 10 <sup>3</sup>                            | -499          | "                                |
| 17  | 3.10 × 10 <sup>3</sup>                            | -229          | "                                | 8.20 × 10 <sup>3</sup>                            | -497          | "                                | 4.07 × 10 <sup>3</sup>                            | -511          | "                                |
| 18  | 1.03 × 10 <sup>3</sup>                            | -159          | "                                | 7.52 × 10 <sup>3</sup>                            | -474          | "                                | 2.03 × 10 <sup>3</sup>                            | -501          | "                                |
| 19  | 1.57 × 10 <sup>3</sup>                            | -198          | "                                | 8.01 × 10 <sup>3</sup>                            | -487          | "                                | 1.97 × 10 <sup>3</sup>                            | -498          | "                                |
| 20  | 755                                               | -71           | "                                | 8.13 × 10 <sup>3</sup>                            | -492          | "                                | 3.12 × 10 <sup>3</sup>                            | -505          | "                                |
| 21  | 980                                               | -135          | "                                | 8.28 × 10 <sup>3</sup>                            | -498          | "                                | 4.07 × 10 <sup>3</sup>                            | -511          | "                                |
| 22  | 805                                               | -75           | "                                | 7.73 × 10 <sup>3</sup>                            | -482          | "                                | 1.97 × 10 <sup>3</sup>                            | -498          | "                                |
| 23  | 953                                               | -109          | "                                | 7.99 × 10 <sup>3</sup>                            | -494          | "                                | 4.07 × 10 <sup>3</sup>                            | -511          | "                                |
| 24  | 785                                               | -70           | "                                | 7.66 × 10 <sup>3</sup>                            | -475          | "                                | 1.97 × 10 <sup>3</sup>                            | -498          | "                                |
| 25  | 1.09 × 10 <sup>3</sup>                            | -171          | "                                | 11.9 × 10 <sup>3</sup>                            | -510          | "                                | 4.07 × 10 <sup>3</sup>                            | -511          | "                                |
| 26  | 867                                               | -81           | "                                | 7.92 × 10 <sup>3</sup>                            | -482          | "                                | 1.97 × 10 <sup>3</sup>                            | -498          | "                                |
| 27  | 4.73 × 10 <sup>3</sup>                            | -281          | "                                | 8.10 × 10 <sup>3</sup>                            | -491          | "                                | 2.42 × 10 <sup>3</sup>                            | -503          | "                                |
| 28  | 1.13 × 10 <sup>3</sup>                            | -125          | "                                | 7.50 × 10 <sup>3</sup>                            | -472          | "                                | 2.03 × 10 <sup>3</sup>                            | -501          | "                                |
| 29  | 3.00 × 10 <sup>3</sup>                            | -229          | "                                | 8.06 × 10 <sup>3</sup>                            | -488          | "                                | 2.42 × 10 <sup>3</sup>                            | -503          | "                                |
| 30  | 854                                               | -77           | "                                | 7.14 × 10 <sup>3</sup>                            | -452          | "                                | 2.03 × 10 <sup>3</sup>                            | -501          | "                                |
| 31  | 3.95 × 10 <sup>3</sup>                            | -248          | "                                | 8.09 × 10 <sup>3</sup>                            | -489          | "                                | 2.42 × 10 <sup>3</sup>                            | -503          | "                                |
| 32  | 953                                               | -98           | "                                | 7.21 × 10 <sup>3</sup>                            | -463          | "                                | 2.03 × 10 <sup>3</sup>                            | -501          | "                                |
| 33  | 3.02 × 10 <sup>3</sup>                            | -221          | "                                | 7.75 × 10 <sup>3</sup>                            | -484          | "                                | 2.03 × 10 <sup>3</sup>                            | -507          | "                                |
| 34  | 3.77 × 10 <sup>3</sup>                            | -248          | "                                | 8.15 × 10 <sup>3</sup>                            | -492          | "                                | 4.07 × 10 <sup>3</sup>                            | -511          | "                                |
| 35  | 9.34 × 10 <sup>3</sup>                            | 233           | "                                | 14.6 × 10 <sup>3</sup>                            | 502           | "                                | 12.9 × 10 <sup>3</sup>                            | -744          | "                                |
| 36  | 5.68 × 10 <sup>3</sup>                            | 164           | "                                | 9.28 × 10 <sup>3</sup>                            | 321           | "                                | 7.11 × 10 <sup>3</sup>                            | -516          | "                                |
| 37  | 1.04 × 10 <sup>3</sup>                            | 98            | "                                | 4.67 × 10 <sup>3</sup>                            | 216           | "                                | 2.07 × 10 <sup>3</sup>                            | -440          | "                                |
| 38  | 923                                               | 87            | "                                | 3.34 × 10 <sup>3</sup>                            | 173           | "                                | 1.09 × 10 <sup>3</sup>                            | -395          | "                                |
| 39  | 3.24 × 10 <sup>3</sup>                            | 121           | "                                | 8.89 × 10 <sup>3</sup>                            | 288           | "                                | 7.14 × 10 <sup>3</sup>                            | -512          | "                                |
| 40  | 1.89 × 10 <sup>3</sup>                            | 113           | "                                | 5.11 × 10 <sup>3</sup>                            | 244           | "                                | 2.06 × 10 <sup>3</sup>                            | -438          | "                                |
| 41  | 2.05 × 10 <sup>3</sup>                            | -153          | "                                | 5.14 × 10 <sup>3</sup>                            | -478          | "                                | 5.23 × 10 <sup>3</sup>                            | -482          | "                                |
| 42  | 1.03 × 10 <sup>3</sup>                            | -108          | "                                | 2.05 × 10 <sup>3</sup>                            | -418          | "                                | 1.52 × 10 <sup>3</sup>                            | -421          | "                                |
| 43  | 847                                               | -83           | "                                | 1.23 × 10 <sup>3</sup>                            | -384          | "                                | 1.14 × 10 <sup>3</sup>                            | -397          | "                                |
| 44  | 980                                               | -89           | "                                | 1.62 × 10 <sup>3</sup>                            | -392          | "                                | 2.07 × 10 <sup>3</sup>                            | -440          | "                                |
| 45  | 658                                               | -41           | "                                | 1.54 × 10 <sup>3</sup>                            | -388          | "                                | 1.48 × 10 <sup>3</sup>                            | -420          | "                                |
| 46  | 723                                               | -37           | "                                | 1.47 × 10 <sup>3</sup>                            | -384          | "                                | 1.21 × 10 <sup>3</sup>                            | -399          | "                                |
| 47  | 521                                               | -5            | "                                | 1.14 × 10 <sup>3</sup>                            | -381          | "                                | 1.10 × 10 <sup>3</sup>                            | -395          | "                                |
| 48  | 1.23 × 10 <sup>3</sup>                            | -98           | "                                | 2.09 × 10 <sup>3</sup>                            | -436          | "                                | 2.07 × 10 <sup>3</sup>                            | -440          | "                                |
| 49  | 705                                               | -59           | "                                | 1.32 × 10 <sup>3</sup>                            | -383          | "                                | 1.21 × 10 <sup>3</sup>                            | -399          | "                                |
| 50  | 915                                               | -78           | "                                | 2.10 × 10 <sup>3</sup>                            | -434          | "                                | 2.07 × 10 <sup>3</sup>                            | -440          | "                                |
| 51  | 625                                               | -38           | "                                | 1.25 × 10 <sup>3</sup>                            | -382          | "                                | 1.21 × 10 <sup>3</sup>                            | -399          | "                                |
| 52  | 1.01 × 10 <sup>3</sup>                            | -95           | "                                | 2.13 × 10 <sup>3</sup>                            | -438          | "                                | 2.07 × 10 <sup>3</sup>                            | -440          | "                                |
| 53  | 688                                               | -50           | "                                | 1.82 × 10 <sup>3</sup>                            | -401          | "                                | 1.21 × 10 <sup>3</sup>                            | -399          | "                                |
| 54  | 3.77 × 10 <sup>3</sup>                            | -230          | "                                | 4.05 × 10 <sup>3</sup>                            | -444          | "                                | 1.54 × 10 <sup>3</sup>                            | -422          | "                                |
| 55  | 991                                               | -100          | "                                | 2.03 × 10 <sup>3</sup>                            | -417          | "                                | 1.48 × 10 <sup>3</sup>                            | -420          | "                                |
| 56  | 2.01 × 10 <sup>3</sup>                            | -131          | "                                | 3.49 × 10 <sup>3</sup>                            | -421          | "                                | 1.54 × 10 <sup>3</sup>                            | -422          | "                                |
| 57  | 795                                               | -50           | "                                | 2.09 × 10 <sup>3</sup>                            | -418          | "                                | 1.48 × 10 <sup>3</sup>                            | -420          | "                                |
| 58  | 2.95 × 10 <sup>3</sup>                            | -185          | "                                | 3.63 × 10 <sup>3</sup>                            | -423          | "                                | 1.54 × 10 <sup>3</sup>                            | -422          | "                                |
| 59  | 888                                               | -55           | "                                | 2.02 × 10 <sup>3</sup>                            | -417          | "                                | 1.48 × 10 <sup>3</sup>                            | -420          | "                                |
| 60  | 1.45 × 10 <sup>3</sup>                            | -129          | "                                | 3.51 × 10 <sup>3</sup>                            | -421          | "                                | 1.48 × 10 <sup>3</sup>                            | -420          | "                                |
| 61  | 1.01 × 10 <sup>3</sup>                            | -120          | "                                | 4.25 × 10 <sup>3</sup>                            | -445          | "                                | 2.07 × 10 <sup>3</sup>                            | -440          | "                                |
| 62  | 1.63 × 10 <sup>3</sup>                            | -136          | "                                | 4.50 × 10 <sup>3</sup>                            | 369           | "                                | 2.22 × 10 <sup>3</sup>                            | -451          | "                                |
| 63  | 2.49 × 10 <sup>3</sup>                            | -203          | "                                | 4.82 × 10 <sup>3</sup>                            | -458          | "                                | 4.08 × 10 <sup>3</sup>                            | -462          | "                                |
| 64  | 30.2 × 10 <sup>3</sup>                            | +32           | "                                | 70.5 × 10 <sup>3</sup>                            | -321          | "                                | 97.5 × 10 <sup>3</sup>                            | -829          | "                                |
| 65  | 27.9 × 10 <sup>3</sup>                            | +49           | "                                | 59.7 × 10 <sup>3</sup>                            | -286          | "                                | 25.6 × 10 <sup>3</sup>                            | -519          | "                                |
| 66  | 18.4 × 10 <sup>3</sup>                            | +116          | "                                | 36.5 × 10 <sup>3</sup>                            | -224          | "                                | 12.3 × 10 <sup>3</sup>                            | -268          | "                                |
| 67  | 2.54 × 10 <sup>3</sup>                            | +223          | "                                | 4.39 × 10 <sup>3</sup>                            | -63           | "                                | 1.86 × 10 <sup>3</sup>                            | -85           | "                                |
| 68  | 26.8 × 10 <sup>3</sup>                            | +52           | "                                | 49.3 × 10 <sup>3</sup>                            | -218          | "                                | 27.4 × 10 <sup>3</sup>                            | -436          | "                                |
| 69  | 22.4 × 10 <sup>3</sup>                            | +73           | "                                | 37.2 × 10 <sup>3</sup>                            | -163          | "                                | 12.4 × 10 <sup>3</sup>                            | -270          | "                                |
| 70  | 40.5 × 10 <sup>3</sup>                            | +52           | "                                | 62.7 × 10 <sup>3</sup>                            | -462          | "                                | 42.3 × 10 <sup>3</sup>                            | -639          | "                                |
| 71  | 32.5 × 10 <sup>3</sup>                            | +80           | "                                | 45.6 × 10 <sup>3</sup>                            | -233          | "                                | 8.26 × 10 <sup>3</sup>                            | -248          | "                                |
| 72  | 14.8 × 10 <sup>3</sup>                            | +125          | "                                | 32.8 × 10 <sup>3</sup>                            | -196          | "                                | 7.42 × 10 <sup>3</sup>                            | -236          | "                                |
| 73  | 17.3 × 10 <sup>3</sup>                            | +103          | "                                | 40.5 × 10 <sup>3</sup>                            | -214          | "                                | 12.4 × 10 <sup>3</sup>                            | -270          | "                                |
| 74  | 7.25 × 10 <sup>3</sup>                            | +178          | "                                | 47.6 × 10 <sup>3</sup>                            | -240          | "                                | 8.26 × 10 <sup>3</sup>                            | -248          | "                                |
| 75  | 9.00 × 10 <sup>3</sup>                            | +175          | "                                | 42.1 × 10 <sup>3</sup>                            | -221          | "                                | 6.98 × 10 <sup>3</sup>                            | -230          | "                                |

TABLE 10-continued

(Characteristic values corresponding to the sample in Table 2)

| Nos | Example 1                                         |               |                                  | Carbonate-Free                                    |               |                                  | Carbonate & Fluoride-Free                         |               |                                  |
|-----|---------------------------------------------------|---------------|----------------------------------|---------------------------------------------------|---------------|----------------------------------|---------------------------------------------------|---------------|----------------------------------|
|     | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) |
| 76  | 856                                               | +255          | "                                | 2.04 × 10 <sup>3</sup>                            | -99           | "                                | 2.23 × 10 <sup>3</sup>                            | -103          | "                                |
| 77  | 43.1 × 10 <sup>3</sup>                            | +26           | "                                | 59.4 × 10 <sup>3</sup>                            | -398          | "                                | 42.3 × 10 <sup>3</sup>                            | -639          | "                                |
| 78  | 35.1 × 10 <sup>3</sup>                            | +62           | "                                | 41.8 × 10 <sup>3</sup>                            | -218          | "                                | 8.26 × 10 <sup>3</sup>                            | -248          | "                                |
| 79  | 19.4 × 10 <sup>3</sup>                            | +79           | "                                | 34.5 × 10 <sup>3</sup>                            | -199          | "                                | 7.42 × 10 <sup>3</sup>                            | -236          | "                                |
| 80  | 21.7 × 10 <sup>3</sup>                            | +88           | "                                | 43.2 × 10 <sup>3</sup>                            | -224          | "                                | 12.4 × 10 <sup>3</sup>                            | -270          | "                                |
| 81  | 9.85 × 10 <sup>3</sup>                            | +102          | "                                | 32.9 × 10 <sup>3</sup>                            | -198          | "                                | 8.26 × 10 <sup>3</sup>                            | -248          | "                                |
| 82  | 10.6 × 10 <sup>3</sup>                            | +105          | "                                | 30.5 × 10 <sup>3</sup>                            | -186          | "                                | 6.98 × 10 <sup>3</sup>                            | -230          | "                                |
| 83  | 1.03 × 10 <sup>3</sup>                            | +205          | "                                | 1.85 × 10 <sup>3</sup>                            | -87           | "                                | 2.23 × 10 <sup>3</sup>                            | -103          | "                                |
| 84  | 20.5 × 10 <sup>3</sup>                            | +95           | "                                | 44.6 × 10 <sup>3</sup>                            | -225          | "                                | 12.4 × 10 <sup>3</sup>                            | -270          | "                                |
| 85  | 12.3 × 10 <sup>3</sup>                            | +120          | "                                | 31.2 × 10 <sup>3</sup>                            | -196          | "                                | 6.98 × 10 <sup>3</sup>                            | -230          | "                                |
| 86  | 16.1 × 10 <sup>3</sup>                            | +111          | "                                | 38.7 × 10 <sup>3</sup>                            | -210          | "                                | 12.4 × 10 <sup>3</sup>                            | -270          | "                                |
| 87  | 6.99 × 10 <sup>3</sup>                            | +181          | "                                | 30.9 × 10 <sup>3</sup>                            | -187          | "                                | 6.98 × 10 <sup>3</sup>                            | -230          | "                                |
| 88  | 19.7 × 10 <sup>3</sup>                            | +98           | "                                | 50.2 × 10 <sup>3</sup>                            | -246          | "                                | 12.4 × 10 <sup>3</sup>                            | -270          | "                                |
| 89  | 10.8 × 10 <sup>3</sup>                            | +179          | "                                | 29.6 × 10 <sup>3</sup>                            | -185          | "                                | 6.98 × 10 <sup>3</sup>                            | -230          | "                                |
| 90  | 42.7 × 10 <sup>3</sup>                            | -55           | "                                | 51.3 × 10 <sup>3</sup>                            | -248          | "                                | 8.82 × 10 <sup>3</sup>                            | -252          | "                                |
| 91  | 10.3 × 10 <sup>3</sup>                            | +149          | "                                | 21.6 × 10 <sup>3</sup>                            | -152          | "                                | 8.26 × 10 <sup>3</sup>                            | -248          | "                                |
| 92  | 39.5 × 10 <sup>3</sup>                            | -60           | "                                | 54.9 × 10 <sup>3</sup>                            | -250          | "                                | 8.82 × 10 <sup>3</sup>                            | -252          | "                                |
| 93  | 8.08 × 10 <sup>3</sup>                            | +153          | "                                | 27.4 × 10 <sup>3</sup>                            | -172          | "                                | 8.26 × 10 <sup>3</sup>                            | -248          | "                                |
| 94  | 40.9 × 10 <sup>3</sup>                            | -39           | "                                | 48.6 × 10 <sup>3</sup>                            | -245          | "                                | 8.82 × 10 <sup>3</sup>                            | -252          | "                                |
| 95  | 8.91 × 10 <sup>3</sup>                            | +160          | "                                | 28.2 × 10 <sup>3</sup>                            | -180          | "                                | 8.26 × 10 <sup>3</sup>                            | -248          | "                                |
| 96  | 34.4 × 10 <sup>3</sup>                            | +71           | "                                | 42.5 × 10 <sup>3</sup>                            | -222          | "                                | 8.26 × 10 <sup>3</sup>                            | -248          | "                                |
| 97  | 20.9 × 10 <sup>3</sup>                            | +95           | "                                | 50.0 × 10 <sup>3</sup>                            | -246          | "                                | 12.4 × 10 <sup>3</sup>                            | -270          | "                                |
| 98  | 68.2 × 10 <sup>3</sup>                            | -234          | "                                | 97.6 × 10 <sup>3</sup>                            | -463          | "                                | 100.6 × 10 <sup>3</sup>                           | -957          | "                                |
| 99  | 27.3 × 10 <sup>3</sup>                            | -92           | "                                | 46.5 × 10 <sup>3</sup>                            | -413          | "                                | 32.4 × 10 <sup>3</sup>                            | -607          | "                                |
| 100 | 20.8 × 10 <sup>3</sup>                            | -74           | "                                | 34.8 × 10 <sup>3</sup>                            | -296          | "                                | 21.4 × 10 <sup>3</sup>                            | -483          | "                                |
| 101 | 6.24 × 10 <sup>3</sup>                            | -25           | "                                | 10.7 × 10 <sup>3</sup>                            | -152          | "                                | 5.37 × 10 <sup>3</sup>                            | -195          | "                                |
| 102 | 27.6 × 10 <sup>3</sup>                            | -96           | "                                | 35.2 × 10 <sup>3</sup>                            | -274          | "                                | 32.9 × 10 <sup>3</sup>                            | -436          | "                                |
| 103 | 18.8 × 10 <sup>3</sup>                            | -48           | "                                | 29.6 × 10 <sup>3</sup>                            | -304          | "                                | 21.1 × 10 <sup>3</sup>                            | -490          | "                                |
| 104 | 45.4 × 10 <sup>3</sup>                            | -127          | "                                | 63.2 × 10 <sup>3</sup>                            | -512          | "                                | 68.2 × 10 <sup>3</sup>                            | -802          | "                                |
| 105 | 36.6 × 10 <sup>3</sup>                            | -83           | "                                | 45.2 × 10 <sup>3</sup>                            | -262          | "                                | 12.5 × 10 <sup>3</sup>                            | -271          | "                                |
| 106 | 19.6 × 10 <sup>3</sup>                            | -18           | "                                | 30.4 × 10 <sup>3</sup>                            | -241          | "                                | 7.24 × 10 <sup>3</sup>                            | -243          | "                                |
| 107 | 22.1 × 10 <sup>3</sup>                            | -77           | "                                | 51.3 × 10 <sup>3</sup>                            | -462          | "                                | 21.4 × 10 <sup>3</sup>                            | -483          | "                                |
| 108 | 9.90 × 10 <sup>3</sup>                            | -55           | "                                | 30.3 × 10 <sup>3</sup>                            | -241          | "                                | 6.96 × 10 <sup>3</sup>                            | -338          | "                                |
| 109 | 12.3 × 10 <sup>3</sup>                            | -37           | "                                | 17.7 × 10 <sup>3</sup>                            | -200          | "                                | 6.12 × 10 <sup>3</sup>                            | -219          | "                                |
| 110 | 1.87 × 10 <sup>3</sup>                            | -60           | "                                | 32.8 × 10 <sup>3</sup>                            | -254          | "                                | 8.63 × 10 <sup>3</sup>                            | -262          | "                                |
| 111 | 20.8 × 10 <sup>3</sup>                            | -75           | "                                | 54.2 × 10 <sup>3</sup>                            | -472          | "                                | 21.1 × 10 <sup>3</sup>                            | -490          | "                                |
| 112 | 9.85 × 10 <sup>3</sup>                            | -28           | "                                | 45.3 × 10 <sup>3</sup>                            | -264          | "                                | 12.3 × 10 <sup>3</sup>                            | -270          | "                                |
| 113 | 18.6 × 10 <sup>3</sup>                            | -60           | "                                | 56.3 × 10 <sup>3</sup>                            | -481          | "                                | 21.1 × 10 <sup>3</sup>                            | -490          | "                                |
| 114 | 9.12 × 10 <sup>3</sup>                            | -29           | "                                | 17.4 × 10 <sup>3</sup>                            | -198          | "                                | 6.12 × 10 <sup>3</sup>                            | -219          | "                                |
| 115 | 21.2 × 10 <sup>3</sup>                            | -68           | "                                | 54.3 × 10 <sup>3</sup>                            | -472          | "                                | 21.4 × 10 <sup>3</sup>                            | -483          | "                                |
| 116 | 11.5 × 10 <sup>3</sup>                            | -35           | "                                | 18.6 × 10 <sup>3</sup>                            | -209          | "                                | 6.12 × 10 <sup>3</sup>                            | -219          | "                                |
| 117 | 43.6 × 10 <sup>3</sup>                            | -188          | "                                | 47.9 × 10 <sup>3</sup>                            | -306          | "                                | 14.6 × 10 <sup>3</sup>                            | -302          | "                                |
| 118 | 11.5 × 10 <sup>3</sup>                            | -58           | "                                | 28.9 × 10 <sup>3</sup>                            | -225          | "                                | 6.96 × 10 <sup>3</sup>                            | -233          | "                                |
| 119 | 38.5 × 10 <sup>3</sup>                            | -107          | "                                | 44.6 × 10 <sup>3</sup>                            | -292          | "                                | 14.6 × 10 <sup>3</sup>                            | -302          | "                                |
| 120 | 9.05 × 10 <sup>3</sup>                            | -51           | "                                | 29.3 × 10 <sup>3</sup>                            | -230          | "                                | 6.96 × 10 <sup>3</sup>                            | -233          | "                                |
| 121 | 34.5 × 10 <sup>3</sup>                            | -95           | "                                | 42.3 × 10 <sup>3</sup>                            | -290          | "                                | 14.6 × 10 <sup>3</sup>                            | -302          | "                                |
| 122 | 7.88 × 10 <sup>3</sup>                            | -50           | "                                | 29.5 × 10 <sup>3</sup>                            | -231          | "                                | 6.96 × 10 <sup>3</sup>                            | -233          | "                                |
| 123 | 38.3 × 10 <sup>3</sup>                            | -107          | "                                | 30.2 × 10 <sup>3</sup>                            | -236          | "                                | 6.96 × 10 <sup>3</sup>                            | -233          | "                                |
| 124 | 22.5 × 10 <sup>3</sup>                            | -89           | "                                | 55.4 × 10 <sup>3</sup>                            | -472          | "                                | 21.4 × 10 <sup>3</sup>                            | -483          | "                                |
| 125 | 4.73 × 10 <sup>3</sup>                            | -42           | "                                | 48.6 × 10 <sup>3</sup>                            | -321          | "                                | 3.62 × 10 <sup>3</sup>                            | -138          | "                                |
| 126 | 21.9 × 10 <sup>3</sup>                            | -55           | "                                | 48.6 × 10 <sup>3</sup>                            | -321          | "                                | 16.9 × 10 <sup>3</sup>                            | -324          | "                                |
| 127 | 2.22 × 10 <sup>3</sup>                            | -126          | "                                | 3.48 × 10 <sup>3</sup>                            | -324          | "                                | 2.36 × 10 <sup>3</sup>                            | -626          | "                                |
| 128 | 1.76 × 10 <sup>3</sup>                            | -83           | "                                | 2.32 × 10 <sup>3</sup>                            | -302          | "                                | 1.90 × 10 <sup>3</sup>                            | -490          | "                                |
| 129 | 893                                               | +64           | "                                | 1.26 × 10 <sup>3</sup>                            | -236          | "                                | 619                                               | -251          | "                                |
| 130 | 562                                               | +52           | "                                | 763                                               | -103          | "                                | 488                                               | +55           | "                                |
| 131 | 2.04 × 10 <sup>3</sup>                            | -109          | "                                | 2.88 × 10 <sup>3</sup>                            | -318          | "                                | 1.92 × 10 <sup>3</sup>                            | -505          | "                                |
| 132 | 724                                               | -63           | "                                | 846                                               | -193          | "                                | 621                                               | -250          | "                                |
| 133 | 841                                               | -216          | "                                | 1.25 × 10 <sup>3</sup>                            | -493          | "                                | 2.35 × 10 <sup>3</sup>                            | -732          | "                                |
| 134 | 803                                               | -185          | "                                | 1.09 × 10 <sup>3</sup>                            | -240          | "                                | 492                                               | -241          | "                                |
| 135 | 596                                               | -107          | "                                | 954                                               | -236          | "                                | 468                                               | -238          | "                                |
| 136 | 608                                               | -106          | "                                | 1.12 × 10 <sup>3</sup>                            | -248          | "                                | 621                                               | -250          | "                                |
| 137 | 442                                               | +56           | "                                | 974                                               | -238          | "                                | 492                                               | -241          | "                                |
| 138 | 438                                               | +58           | "                                | 968                                               | -237          | "                                | 474                                               | -239          | "                                |
| 139 | 396                                               | +95           | "                                | 942                                               | -232          | "                                | 442                                               | -235          | "                                |
| 140 | 839                                               | -238          | "                                | 1.22 × 10 <sup>3</sup>                            | -487          | "                                | 2.35 × 10 <sup>3</sup>                            | -732          | "                                |
| 141 | 798                                               | -198          | "                                | 1.10 × 10 <sup>3</sup>                            | -242          | "                                | 492                                               | -241          | "                                |
| 142 | 597                                               | -115          | "                                | 969                                               | -237          | "                                | 468                                               | -238          | "                                |
| 143 | 603                                               | -118          | "                                | 1.14 × 10 <sup>3</sup>                            | -248          | "                                | 621                                               | -250          | "                                |
| 144 | 438                                               | +5            | "                                | 975                                               | -238          | "                                | 492                                               | -241          | "                                |
| 145 | 441                                               | -15           | "                                | 965                                               | -237          | "                                | 474                                               | -239          | "                                |
| 146 | 390                                               | +21           | "                                | 948                                               | -233          | "                                | 442                                               | -235          | "                                |
| 147 | 705                                               | -159          | "                                | 1.16 × 10 <sup>3</sup>                            | -249          | "                                | 621                                               | -250          | "                                |
| 148 | 509                                               | -56           | "                                | 964                                               | -236          | "                                | 474                                               | -239          | "                                |
| 149 | 617                                               | -111          | "                                | 1.13 × 10 <sup>3</sup>                            | -248          | "                                | 621                                               | -250          | "                                |
| 150 | 459                                               | +41           | "                                | 968                                               | -237          | "                                | 474                                               | -239          | "                                |

TABLE 10-continued

(Characteristic values corresponding to the sample in Table 2)

| Nos | Example 1                                         |                                           | Carbonate-Free                                    |                                           |                                                   | Carbonate & Fluoride-Free                 |                                                   |                                           |
|-----|---------------------------------------------------|-------------------------------------------|---------------------------------------------------|-------------------------------------------|---------------------------------------------------|-------------------------------------------|---------------------------------------------------|-------------------------------------------|
|     | Resistance value at 25° C.<br>R <sub>25</sub> (Ω) | Rate of Change in Resistance<br>(ppm/°C.) | Resistance value at 25° C.<br>R <sub>25</sub> (Ω) | Rate of Change in Resistance<br>(ppm/°C.) | Resistance value at 25° C.<br>R <sub>25</sub> (Ω) | Rate of Change in Resistance<br>(ppm/°C.) | Resistance value at 25° C.<br>R <sub>25</sub> (Ω) | Rate of Change in Resistance<br>(ppm/°C.) |
| 151 | 668                                               | -140                                      | "                                                 | 1.18 × 10 <sup>3</sup>                    | -252                                              | "                                         | 621                                               | -250                                      |
| 152 | 481                                               | +36                                       | "                                                 | 970                                       | -237                                              | "                                         | 474                                               | -239                                      |
| 153 | 636                                               | -119                                      | "                                                 | 973                                       | -237                                              | "                                         | 470                                               | -238                                      |
| 154 | 481                                               | -5                                        | "                                                 | 976                                       | -238                                              | "                                         | 492                                               | -241                                      |
| 155 | 578                                               | -106                                      | "                                                 | 975                                       | -239                                              | "                                         | 470                                               | -238                                      |
| 156 | 425                                               | -9                                        | "                                                 | 977                                       | -238                                              | "                                         | 492                                               | -241                                      |
| 157 | 615                                               | -120                                      | "                                                 | 982                                       | -240                                              | "                                         | 470                                               | -238                                      |
| 158 | 469                                               | -20                                       | "                                                 | 974                                       | -239                                              | "                                         | 492                                               | -241                                      |
| 159 | 846                                               | -221                                      | "                                                 | 1.01 × 10 <sup>3</sup>                    | -243                                              | "                                         | 492                                               | -241                                      |
| 160 | 641                                               | -152                                      | "                                                 | 977                                       | -239                                              | "                                         | 621                                               | -239                                      |
| 161 | 3.95 × 10 <sup>3</sup>                            | -212                                      | "                                                 | 8.94 × 10 <sup>3</sup>                    | -324                                              | "                                         | 4.66 × 10 <sup>3</sup>                            | -677                                      |
| 162 | 3.23 × 10 <sup>3</sup>                            | -186                                      | "                                                 | 6.62 × 10 <sup>3</sup>                    | -295                                              | "                                         | 3.51 × 10 <sup>3</sup>                            | -525                                      |
| 163 | 1.24 × 10 <sup>3</sup>                            | -1.52                                     | "                                                 | 4.63 × 10 <sup>3</sup>                    | -251                                              | "                                         | 1.19 × 10 <sup>3</sup>                            | -400                                      |
| 164 | 886                                               | -82                                       | "                                                 | 1.64 × 10 <sup>3</sup>                    | -183                                              | "                                         | 728                                               | -305                                      |
| 165 | 3.65 × 10 <sup>3</sup>                            | -205                                      | "                                                 | 6.49 × 10 <sup>3</sup>                    | -294                                              | "                                         | 3.54 × 10 <sup>3</sup>                            | -520                                      |
| 166 | 2.02 × 10 <sup>3</sup>                            | -163                                      | "                                                 | 3.28 × 10 <sup>3</sup>                    | -198                                              | "                                         | 1.22 × 10 <sup>3</sup>                            | -398                                      |
| 167 | 852                                               | -235                                      | "                                                 | 2.62 × 10 <sup>3</sup>                    | -498                                              | "                                         | 4.12 × 10 <sup>3</sup>                            | -612                                      |
| 168 | 814                                               | -204                                      | "                                                 | 2.18 × 10 <sup>3</sup>                    | -352                                              | "                                         | 983                                               | -354                                      |
| 169 | 605                                               | -113                                      | "                                                 | 1.94 × 10 <sup>3</sup>                    | -331                                              | "                                         | 842                                               | -332                                      |
| 170 | 619                                               | -119                                      | "                                                 | 2.25 × 10 <sup>3</sup>                    | -397                                              | "                                         | 1.19 × 10 <sup>3</sup>                            | -400                                      |
| 171 | 453                                               | -55                                       | "                                                 | 2.10 × 10 <sup>3</sup>                    | -357                                              | "                                         | 983                                               | -354                                      |
| 172 | 449                                               | -51                                       | "                                                 | 1.65 × 10 <sup>3</sup>                    | -321                                              | "                                         | 815                                               | -324                                      |
| 173 | 407                                               | -32                                       | "                                                 | 1.42 × 10 <sup>3</sup>                    | -304                                              | "                                         | 734                                               | -307                                      |
| 174 | 634                                               | -124                                      | "                                                 | 2.24 × 10 <sup>3</sup>                    | -397                                              | " -1.19 × 10 <sup>3</sup>                 | -400                                              | "                                         |
| 175 | 463                                               | -60                                       | "                                                 | 1.70 × 10 <sup>3</sup>                    | -322                                              | "                                         | 815                                               | -324                                      |
| 176 | 594                                               | -108                                      | "                                                 | 2.21 × 10 <sup>3</sup>                    | -396                                              | "                                         | 1.19 × 10 <sup>3</sup>                            | -400                                      |
| 177 | 426                                               | -49                                       | "                                                 | 1.51 × 10 <sup>3</sup>                    | -320                                              | "                                         | 815                                               | -324                                      |
| 178 | 581                                               | -94                                       | "                                                 | 2.28 × 10 <sup>3</sup>                    | -399                                              | "                                         | 1.19 × 10 <sup>3</sup>                            | -400                                      |
| 179 | 407                                               | -35                                       | "                                                 | 1.60 × 10 <sup>3</sup>                    | -321                                              | "                                         | 815                                               | -324                                      |
| 180 | 664                                               | -185                                      | "                                                 | 2.18 × 10 <sup>3</sup>                    | -369                                              | "                                         | 997                                               | -400                                      |
| 181 | 499                                               | -115                                      | "                                                 | 1.99 × 10 <sup>3</sup>                    | -353                                              | "                                         | 983                                               | -324                                      |
| 182 | 617                                               | -124                                      | "                                                 | 2.12 × 10 <sup>3</sup>                    | -367                                              | "                                         | 997                                               | -368                                      |
| 183 | 469                                               | -100                                      | "                                                 | 2.10 × 10 <sup>3</sup>                    | -352                                              | "                                         | 983                                               | -354                                      |
| 184 | 631                                               | -153                                      | "                                                 | 2.21 × 10 <sup>3</sup>                    | -370                                              | "                                         | 997                                               | -368                                      |
| 185 | 481                                               | -85                                       | "                                                 | 2.09 × 10 <sup>3</sup>                    | -352                                              | "                                         | 983                                               | -354                                      |
| 186 | 837                                               | -236                                      | "                                                 | 2.07 × 10 <sup>3</sup>                    | -356                                              | "                                         | 983                                               | -354                                      |
| 187 | 639                                               | -161                                      | "                                                 | 2.30 × 10 <sup>3</sup>                    | -398                                              | "                                         | 1.19 × 10 <sup>3</sup>                            | -400                                      |
| 188 | 592                                               | -83                                       | "                                                 | 1.03 × 10 <sup>3</sup>                    | -203                                              | "                                         | 608                                               | -252                                      |
| 189 | 453                                               | -40                                       | "                                                 | 1.99 × 10 <sup>3</sup>                    | -338                                              | "                                         | 906                                               | -341                                      |
| 190 | 875                                               | -109                                      | "                                                 | 1.58 × 10 <sup>3</sup>                    | -163                                              | "                                         | 706                                               | +148                                      |
| 191 | 652                                               | -17                                       | "                                                 | 1.36 × 10 <sup>3</sup>                    | -124                                              | "                                         | 518                                               | +287                                      |
| 192 | 426                                               | +74                                       | "                                                 | 924                                       | +320                                              | "                                         | 270                                               | +401                                      |
| 193 | 349                                               | +108                                      | "                                                 | 763                                       | +263                                              | "                                         | 196                                               | +428                                      |
| 194 | 775                                               | -28                                       | "                                                 | 1.40 × 10 <sup>3</sup>                    | +318                                              | "                                         | 520                                               | +290                                      |
| 195 | 328                                               | +107                                      | "                                                 | 863                                       | +318                                              | "                                         | 270                                               | +505                                      |
| 196 | 525                                               | +55                                       | "                                                 | 683                                       | +184                                              | "                                         | 652                                               | +182                                      |
| 197 | 490                                               | +83                                       | "                                                 | 820                                       | +428                                              | "                                         | 235                                               | +582                                      |
| 198 | 321                                               | +105                                      | "                                                 | 852                                       | +462                                              | "                                         | 213                                               | +589                                      |
| 199 | 285                                               | +118                                      | "                                                 | 802                                       | +412                                              | "                                         | 270                                               | +505                                      |
| 200 | 141                                               | +267                                      | "                                                 | 830                                       | +445                                              | "                                         | 224                                               | +584                                      |
| 201 | 94                                                | +300                                      | "                                                 | 860                                       | +482                                              | "                                         | 202                                               | +598                                      |
| 202 | 341                                               | +108                                      | "                                                 | 801                                       | +410                                              | "                                         | 270                                               | +505                                      |
| 203 | 310                                               | +111                                      | "                                                 | 802                                       | +411                                              | "                                         | 270                                               | +505                                      |
| 204 | 335                                               | +105                                      | "                                                 | 801                                       | +409                                              | "                                         | 270                                               | +505                                      |
| 205 | 182                                               | +250                                      | "                                                 | 835                                       | +452                                              | "                                         | 224                                               | +584                                      |
| 206 | 131                                               | +273                                      | "                                                 | 854                                       | +463                                              | "                                         | 224                                               | +584                                      |
| 207 | 115                                               | +295                                      | "                                                 | 857                                       | +471                                              | "                                         | 224                                               | +505                                      |
| 208 | 503                                               | +90                                       | "                                                 | 822                                       | +430                                              | "                                         | 232                                               | +584                                      |
| 209 | 495                                               | +88                                       | "                                                 | 818                                       | +425                                              | "                                         | 232                                               | +582                                      |
| 210 | 508                                               | +97                                       | "                                                 | 824                                       | +438                                              | "                                         | 232                                               | +582                                      |
| 211 | 932                                               | -83                                       | "                                                 | 1.65 × 10 <sup>3</sup>                    | -164                                              | "                                         | 761                                               | +108                                      |
| 212 | 729                                               | -65                                       | "                                                 | 1.29 × 10 <sup>3</sup>                    | -142                                              | "                                         | 588                                               | +144                                      |
| 213 | 544                                               | +86                                       | "                                                 | 962                                       | +242                                              | "                                         | 380                                               | +273                                      |
| 214 | 428                                               | +132                                      | "                                                 | 743                                       | +264                                              | "                                         | 254                                               | +326                                      |
| 215 | 583                                               | +25                                       | "                                                 | 721                                       | +124                                              | "                                         | 675                                               | +126                                      |
| 216 | 512                                               | +28                                       | "                                                 | 542                                       | +300                                              | "                                         | 289                                               | +302                                      |
| 217 | 351                                               | +100                                      | "                                                 | 628                                       | +272                                              | "                                         | 380                                               | +273                                      |
| 218 | 296                                               | +233                                      | "                                                 | 423                                       | +316                                              | "                                         | 265                                               | +318                                      |
| 219 | 181                                               | +279                                      | "                                                 | 446                                       | +313                                              | "                                         | 274                                               | +314                                      |
| 220 | 120                                               | +286                                      | "                                                 | 404                                       | +318                                              | "                                         | 260                                               | +320                                      |
| 221 | 329                                               | +109                                      | "                                                 | 635                                       | +271                                              | "                                         | 380                                               | +273                                      |
| 222 | 318                                               | +96                                       | "                                                 | 648                                       | +270                                              | "                                         | 380                                               | +273                                      |
| 223 | 342                                               | +108                                      | "                                                 | 672                                       | +272                                              | "                                         | 380                                               | +273                                      |
| 224 | 245                                               | +240                                      | "                                                 | 405                                       | +310                                              | "                                         | 274                                               | +314                                      |

TABLE 10-continued

| Nos | Example 1                  |                              |                            | Carbonate-Free               |                            |                              | Carbonate & Fluoride-Free  |                              |                            |
|-----|----------------------------|------------------------------|----------------------------|------------------------------|----------------------------|------------------------------|----------------------------|------------------------------|----------------------------|
|     | Resistance value at 25° C. | Rate of Change in Resistance | Resistance value at 25° C. | Rate of Change in Resistance | Resistance value at 25° C. | Rate of Change in Resistance | Resistance value at 25° C. | Rate of Change in Resistance | Resistance value at 25° C. |
|     | R <sub>25</sub> (Ω)        | (ppm/°C.)                    | R <sub>25</sub> (Ω)        | (ppm/°C.)                    | R <sub>25</sub> (Ω)        | (ppm/°C.)                    | R <sub>25</sub> (Ω)        | (ppm/°C.)                    | R <sub>25</sub> (Ω)        |
| 225 | 195                        | +268                         | "                          | 453                          | +312                       | "                            | 274                        | +314                         | "                          |
| 226 | 212                        | +259                         | "                          | 398                          | +311                       | "                            | 274                        | +314                         | "                          |
| 227 | 325                        | +218                         | "                          | 436                          | +315                       | "                            | 265                        | +318                         | "                          |
| 228 | 331                        | +245                         | "                          | 425                          | +316                       | "                            | 265                        | +318                         | "                          |
| 229 | 319                        | +250                         | "                          | 411                          | +317                       | "                            | 265                        | +318                         | "                          |
| 230 | 824                        | -120                         | "                          | 1.32 × 10 <sup>3</sup>       | -216                       | "                            | 645                        | +107                         | "                          |
| 231 | 536                        | +31                          | "                          | 824                          | +103                       | "                            | 415                        | +209                         | "                          |
| 232 | 743                        | -21                          | "                          | 1.28 × 10 <sup>3</sup>       | -183                       | "                            | 645                        | +106                         | "                          |
| 233 | 526                        | +40                          | "                          | 832                          | +149                       | "                            | 410                        | +211                         | "                          |
| 234 | 721                        | -23                          | "                          | 1.42 × 10 <sup>3</sup>       | +156                       | "                            | 528                        | +158                         | "                          |
| 235 | 605                        | +12                          | "                          | 868                          | +360                       | "                            | 239                        | +362                         | "                          |
| 236 | 433                        | +183                         | "                          | 1.02 × 10 <sup>3</sup>       | +212                       | "                            | 410                        | +211                         | "                          |
| 237 | 380                        | +209                         | "                          | 675                          | +500                       | "                            | 203                        | +502                         | "                          |
| 238 | 350                        | +221                         | "                          | 623                          | +701                       | "                            | 191                        | +702                         | "                          |
| 239 | 211                        | +266                         | "                          | 543                          | +974                       | "                            | 182                        | +982                         | "                          |
| 240 | 505                        | +50                          | "                          | 1.32 × 10 <sup>3</sup>       | +208                       | "                            | 410                        | +211                         | "                          |
| 241 | 450                        | +61                          | "                          | 1.14 × 10 <sup>3</sup>       | +210                       | "                            | 410                        | +211                         | "                          |
| 242 | 475                        | +63                          | "                          | 1.06 × 10 <sup>3</sup>       | +211                       | "                            | 410                        | +211                         | "                          |
| 243 | 405                        | +179                         | "                          | 652                          | +698                       | "                            | 191                        | +702                         | "                          |
| 244 | 386                        | +205                         | "                          | 620                          | +701                       | "                            | 191                        | +702                         | "                          |
| 245 | 421                        | +185                         | "                          | 640                          | +699                       | "                            | 191                        | +702                         | "                          |
| 246 | 383                        | +207                         | "                          | 682                          | +484                       | "                            | 208                        | +486                         | "                          |
| 247 | 422                        | +199                         | "                          | 924                          | +302                       | "                            | 396                        | +304                         | "                          |
| 248 | 639                        | -161                         | "                          | 583                          | +105                       | "                            | 354                        | +294                         | "                          |
| 249 | 17.5 × 10 <sup>3</sup>     | -124                         | "                          | 25.8 × 10 <sup>3</sup>       | -321                       | "                            | 18.6 × 10 <sup>3</sup>     | -448                         | "                          |
| 250 | 10.5 × 10 <sup>3</sup>     | -79                          | "                          | 16.7 × 10 <sup>3</sup>       | -212                       | "                            | 11.9 × 10 <sup>3</sup>     | -507                         | "                          |
| 251 | 5.29 × 10 <sup>3</sup>     | -36                          | "                          | 9.24 × 10 <sup>3</sup>       | -143                       | "                            | 4.88 × 10 <sup>3</sup>     | -487                         | "                          |
| 252 | 21.6 × 10 <sup>3</sup>     | -144                         | "                          | 32.3 × 10 <sup>3</sup>       | -365                       | "                            | 20.6 × 10 <sup>3</sup>     | -449                         | "                          |
| 253 | 1.98 × 10 <sup>3</sup>     | +28                          | "                          | 7.62 × 10 <sup>3</sup>       | -62                        | "                            | 2.30 × 10 <sup>3</sup>     | -87                          | "                          |
| 254 | 12.4 × 10 <sup>3</sup>     | -106                         | "                          | 15.6 × 10 <sup>3</sup>       | -203                       | "                            | 7.08 × 10 <sup>3</sup>     | -328                         | "                          |
| 255 | 17.9 × 10 <sup>3</sup>     | -131                         | "                          | 24.8 × 10 <sup>3</sup>       | -272                       | "                            | 16.6 × 10 <sup>3</sup>     | -308                         | "                          |
| 256 | 16.8 × 10 <sup>3</sup>     | -129                         | "                          | 22.9 × 10 <sup>3</sup>       | -264                       | "                            | 14.5 × 10 <sup>3</sup>     | -381                         | "                          |
| 257 | 6.88 × 10 <sup>3</sup>     | -54                          | "                          | 13.9 × 10 <sup>3</sup>       | -179                       | "                            | 6.21 × 10 <sup>3</sup>     | -422                         | "                          |
| 258 | 6.02 × 10 <sup>3</sup>     | -42                          | "                          | 11.2 × 10 <sup>3</sup>       | -158                       | "                            | 5.49 × 10 <sup>3</sup>     | -456                         | "                          |
| 259 | 13.2 × 10 <sup>3</sup>     | -109                         | "                          | 22.4 × 10 <sup>3</sup>       | -252                       | "                            | 12.2 × 10 <sup>3</sup>     | -470                         | "                          |
| 260 | 16.4 × 10 <sup>3</sup>     | -120                         | "                          | 23.8 × 10 <sup>3</sup>       | -270                       | "                            | 14.6 × 10 <sup>3</sup>     | -485                         | "                          |
| 261 | 18.6 × 10 <sup>3</sup>     | -128                         | "                          | 42.6 × 10 <sup>3</sup>       | -391                       | "                            | 27.4 × 10 <sup>3</sup>     | -641                         | "                          |
| 262 | 9.64 × 10 <sup>3</sup>     | -94                          | "                          | 17.9 × 10 <sup>3</sup>       | -224                       | "                            | 8.61 × 10 <sup>3</sup>     | -588                         | "                          |
| 263 | 2.39 × 10 <sup>3</sup>     | +15                          | "                          | 6.93 × 10 <sup>3</sup>       | -891                       | "                            | 2.19 × 10 <sup>3</sup>     | -501                         | "                          |
| 264 | 1.68 × 10 <sup>3</sup>     | +32                          | "                          | 4.83 × 10 <sup>3</sup>       | -521                       | "                            | 1.55 × 10 <sup>3</sup>     | +57                          | "                          |
| 265 | -18.7 × 10 <sup>3</sup>    | -222                         | "                          | 24.5 × 10 <sup>3</sup>       | -342                       | "                            | 16.3 × 10 <sup>3</sup>     | -342                         | "                          |
| 266 | 8.38 × 10 <sup>3</sup>     | -124                         | "                          | 10.6 × 10 <sup>3</sup>       | -296                       | "                            | 7.35 × 10 <sup>3</sup>     | -296                         | "                          |
| 267 | 624                        | +10                          | "                          | 928                          | -42                        | "                            | 483                        | -42                          | "                          |
| 268 | 921                        | +35                          | "                          | 1.03 × 10 <sup>3</sup>       | -28                        | "                            | 826                        | -28                          | "                          |
| 269 | 3.21 × 10                  | -89                          | "                          | 4.28 × 10 <sup>3</sup>       | -251                       | "                            | 2.38 × 10 <sup>3</sup>     | -251                         | "                          |
| 270 | 3.3 × 10 <sup>3</sup>      | -98                          | "                          | 4.93 × 10 <sup>3</sup>       | -124                       | "                            | 2.88 × 10 <sup>3</sup>     | -256                         | "                          |
| 271 | 7.46 × 10 <sup>3</sup>     | -169                         | "                          | 18.3 × 10 <sup>3</sup>       | -405                       | "                            | 16.6 × 10 <sup>3</sup>     | -546                         | "                          |
| 272 | 1.39 × 10 <sup>3</sup>     | -132                         | "                          | 8.11 × 10 <sup>3</sup>       | -216                       | "                            | 14.5 × 10 <sup>3</sup>     | -367                         | "                          |
| 273 | 342                        | +23                          | "                          | 560                          | -51                        | "                            | 6.21 × 10 <sup>3</sup>     | -44                          | "                          |
| 274 | 694                        | -41                          | "                          | 925                          | -88                        | "                            | 5.49 × 10 <sup>3</sup>     | -109                         | "                          |
| 275 | 1.54 × 10 <sup>3</sup>     | -142                         | "                          | 3.00 × 10 <sup>3</sup>       | -295                       | "                            | 12.2 × 10 <sup>3</sup>     | -381                         | "                          |
| 276 | 1.03 × 10 <sup>3</sup>     | -95                          | "                          | 3.49 × 10 <sup>3</sup>       | -186                       | "                            | 14.6 × 10 <sup>3</sup>     | -242                         | "                          |

TABLE 11

| Nos | Example 1                  |                              |                            | Carbonate-Free               |                            |                              | Carbonate & Fluoride-Free  |                              |                            |
|-----|----------------------------|------------------------------|----------------------------|------------------------------|----------------------------|------------------------------|----------------------------|------------------------------|----------------------------|
|     | Resistance value at 25° C. | Rate of Change in Resistance | Resistance value at 25° C. | Rate of Change in Resistance | Resistance value at 25° C. | Rate of Change in Resistance | Resistance value at 25° C. | Rate of Change in Resistance | Resistance value at 25° C. |
|     | R <sub>25</sub> (Ω)        | (ppm/°C.)                    | R <sub>25</sub> (Ω)        | (ppm/°C.)                    | R <sub>25</sub> (Ω)        | (ppm/°C.)                    | R <sub>25</sub> (Ω)        | (ppm/°C.)                    | R <sub>25</sub> (Ω)        |
| 1   | 9.23 × 10 <sup>3</sup>     | -48                          | < ±2                       | 15.2 × 10 <sup>3</sup>       | -268                       | < ±2                         | 8.78 × 10 <sup>3</sup>     | -916                         | < ±2                       |
| 2   | 5.69 × 10 <sup>3</sup>     | +21                          | "                          | 7.94 × 10 <sup>3</sup>       | -196                       | "                            | 5.10 × 10 <sup>3</sup>     | -522                         | "                          |
| 3   | 3.48 × 10 <sup>3</sup>     | +163                         | "                          | 4.22 × 10 <sup>3</sup>       | -154                       | "                            | 3.16 × 10 <sup>3</sup>     | -398                         | "                          |
| 4   | 3.16 × 10 <sup>3</sup>     | +125                         | "                          | 4.09 × 10 <sup>3</sup>       | -150                       | "                            | 3.05 × 10 <sup>3</sup>     | -216                         | "                          |
| 5   | 5.74 × 10 <sup>3</sup>     | +12                          | "                          | 8.26 × 10 <sup>3</sup>       | -214                       | "                            | 5.17 × 10 <sup>3</sup>     | -529                         | "                          |
| 6   | 3.52 × 10 <sup>3</sup>     | -174                         | "                          | 6.13 × 10 <sup>3</sup>       | -189                       | "                            | 3.22 × 10 <sup>3</sup>     | -402                         | "                          |
| 7   | 5.48 × 10 <sup>3</sup>     | +36                          | "                          | 5.63 × 10 <sup>3</sup>       | -171                       | "                            | 5.01 × 10 <sup>3</sup>     | -516                         | "                          |
| 8   | 5.16 × 10 <sup>3</sup>     | +38                          | "                          | 5.49 × 10 <sup>3</sup>       | -170                       | "                            | 2.82 × 10 <sup>3</sup>     | -201                         | "                          |
| 9   | 3.15 × 10 <sup>3</sup>     | +126                         | "                          | 4.98 × 10 <sup>3</sup>       | -166                       | "                            | 2.73 × 10 <sup>3</sup>     | -185                         | "                          |
| 10  | 3.23 × 10 <sup>3</sup>     | +150                         | "                          | 5.16 × 10 <sup>3</sup>       | -167                       | "                            | 3.04 × 10 <sup>3</sup>     | -215                         | "                          |
| 11  | 2.84 × 10 <sup>3</sup>     | +195                         | "                          | 4.62 × 10 <sup>3</sup>       | -162                       | "                            | 2.65 × 10 <sup>3</sup>     | -177                         | "                          |

TABLE 11-continued

(Characteristic values corresponding to the sample in Table 3)

| Nos | Example 1                  |               |                                  | Carbonate-Free             |               |                                  | Carbonate & Fluoride-Free  |               |                                  |
|-----|----------------------------|---------------|----------------------------------|----------------------------|---------------|----------------------------------|----------------------------|---------------|----------------------------------|
|     | Resistance value at 25° C. | TCR (ppm/°C.) | Rate of Change in Resistance (%) | Resistance value at 25° C. | TCR (ppm/°C.) | Rate of Change in Resistance (%) | Resistance value at 25° C. | TCR (ppm/°C.) | Rate of Change in Resistance (%) |
| 12  | $2.46 \times 10^3$         | +242          | "                                | $4.41 \times 10^3$         | -161          | "                                | $2.62 \times 10^3$         | -175          | "                                |
| 13  | $5.88 \times 10^3$         | +7            | "                                | $6.02 \times 10^3$         | -191          | "                                | $2.82 \times 10^3$         | -201          | "                                |
| 14  | $4.21 \times 10^3$         | +108          | "                                | $5.81 \times 10^3$         | -172          | "                                | $3.04 \times 10^3$         | -215          | "                                |
| 15  | $4.92 \times 10^3$         | +43           | "                                | $6.11 \times 10^3$         | -198          | "                                | $2.82 \times 10^3$         | -201          | "                                |
| 16  | $3.00 \times 10^3$         | +161          | "                                | $5.99 \times 10^3$         | -182          | "                                | $3.04 \times 10^3$         | -215          | "                                |
| 17  | $5.38 \times 10^3$         | +34           | "                                | $6.15 \times 10^3$         | -199          | "                                | $2.82 \times 10^3$         | -201          | "                                |
| 18  | $3.81 \times 10^3$         | +136          | "                                | $6.01 \times 10^3$         | -188          | "                                | $3.04 \times 10^3$         | -215          | "                                |
| 19  | $2.84 \times 10^3$         | +167          | "                                | $5.85 \times 10^3$         | -180          | "                                | $2.73 \times 10^3$         | -185          | "                                |
| 20  | $2.40 \times 10^3$         | +193          | "                                | $5.65 \times 10^3$         | -173          | "                                | $2.65 \times 10^3$         | -177          | "                                |
| 21  | $2.69 \times 10^3$         | +181          | "                                | $5.84 \times 10^3$         | -178          | "                                | $2.73 \times 10^3$         | -185          | "                                |
| 22  | $2.18 \times 10^3$         | +180          | "                                | $5.62 \times 10^3$         | -171          | "                                | $2.65 \times 10^3$         | -177          | "                                |
| 23  | $3.08 \times 10^3$         | +130          | "                                | $5.88 \times 10^3$         | -181          | "                                | $2.73 \times 10^3$         | -185          | "                                |
| 24  | $2.61 \times 10^3$         | +185          | "                                | $5.67 \times 10^3$         | -174          | "                                | $2.65 \times 10^3$         | -177          | "                                |
| 25  | $3.40 \times 10^3$         | +151          | "                                | $6.19 \times 10^3$         | -209          | "                                | $3.04 \times 10^3$         | -215          | "                                |
| 26  | $2.99 \times 10^3$         | +203          | "                                | $6.22 \times 10^3$         | -211          | "                                | $3.04 \times 10^3$         | -215          | "                                |
| 27  | $3.08 \times 10^3$         | +176          | "                                | $6.25 \times 10^3$         | -214          | "                                | $3.04 \times 10^3$         | -215          | "                                |
| 28  | $8.72 \times 10^3$         | -62           | "                                | $14.3 \times 10^3$         | -278          | "                                | $8.55 \times 10^3$         | -859          | "                                |
| 29  | $5.11 \times 10^3$         | +119          | "                                | $11.2 \times 10^3$         | -257          | "                                | $5.03 \times 10^3$         | -545          | "                                |
| 30  | $2.92 \times 10^3$         | +267          | "                                | $8.92 \times 10^3$         | -148          | "                                | $3.02 \times 10^3$         | -349          | "                                |
| 31  | $2.89 \times 10^3$         | +246          | "                                | $5.71 \times 10^3$         | -92           | "                                | $2.88 \times 10^3$         | -207          | "                                |
| 32  | $4.94 \times 10^3$         | +205          | "                                | $9.96 \times 10^3$         | -246          | "                                | $5.00 \times 10^3$         | -550          | "                                |
| 33  | $3.09 \times 10^3$         | +167          | "                                | $7.23 \times 10^3$         | -104          | "                                | $3.07 \times 10^3$         | -389          | "                                |
| 34  | $4.89 \times 10^3$         | +103          | "                                | $6.21 \times 10^3$         | -490          | "                                | $4.98 \times 10^3$         | -531          | "                                |
| 35  | $4.57 \times 10^3$         | +96           | "                                | $5.31 \times 10^3$         | -243          | "                                | $2.91 \times 10^3$         | -241          | "                                |
| 36  | $2.66 \times 10^3$         | +145          | "                                | $3.68 \times 10^3$         | -216          | "                                | $2.89 \times 10^3$         | -223          | "                                |
| 37  | $2.74 \times 10^3$         | +149          | "                                | $5.52 \times 10^3$         | -258          | "                                | $2.95 \times 10^3$         | -262          | "                                |
| 38  | $2.33 \times 10^3$         | +189          | "                                | $4.86 \times 10^3$         | -234          | "                                | $2.90 \times 10^3$         | -236          | "                                |
| 39  | $1.97 \times 10^3$         | +240          | "                                | $3.32 \times 10^3$         | -207          | "                                | $2.88 \times 10^3$         | -209          | "                                |
| 40  | $5.03 \times 10^3$         | +65           | "                                | $5.21 \times 10^3$         | -239          | "                                | $2.91 \times 10^3$         | -241          | "                                |
| 41  | $3.23 \times 10^3$         | +128          | "                                | $5.83 \times 10^3$         | -264          | "                                | $2.95 \times 10^3$         | -262          | "                                |
| 42  | $4.71 \times 10^3$         | +95           | "                                | $5.25 \times 10^3$         | -240          | "                                | $2.91 \times 10^3$         | -241          | "                                |
| 43  | $2.89 \times 10^3$         | +139          | "                                | $5.75 \times 10^3$         | -261          | "                                | $2.95 \times 10^3$         | -262          | "                                |
| 44  | $4.88 \times 10^3$         | +81           | "                                | $4.98 \times 10^3$         | -238          | "                                | $2.91 \times 10^3$         | -241          | "                                |
| 45  | $3.05 \times 10^3$         | +129          | "                                | $5.67 \times 10^3$         | -259          | "                                | $2.95 \times 10^3$         | -262          | "                                |
| 46  | $3.20 \times 10^3$         | +103          | "                                | $4.65 \times 10^3$         | -225          | "                                | $2.89 \times 10^3$         | -223          | "                                |
| 47  | $2.87 \times 10^3$         | +151          | "                                | $4.61 \times 10^3$         | -235          | "                                | $2.90 \times 10^3$         | -236          | "                                |
| 48  | $2.44 \times 10^3$         | +140          | "                                | $3.81 \times 10^3$         | -220          | "                                | $2.89 \times 10^3$         | -223          | "                                |
| 49  | $2.08 \times 10^3$         | +183          | "                                | $4.77 \times 10^3$         | -223          | "                                | $2.90 \times 10^3$         | -236          | "                                |
| 50  | $2.85 \times 10^3$         | +160          | "                                | $4.68 \times 10^3$         | -227          | "                                | $2.89 \times 10^3$         | -223          | "                                |
| 51  | $2.54 \times 10^3$         | +179          | "                                | $4.87 \times 10^3$         | -234          | "                                | $2.90 \times 10^3$         | -236          | "                                |
| 52  | $4.68 \times 10^3$         | +89           | "                                | $5.30 \times 10^3$         | -243          | "                                | $2.91 \times 10^3$         | -241          | "                                |
| 53  | $4.70 \times 10^3$         | +95           | "                                | $5.32 \times 10^3$         | -245          | "                                | $2.91 \times 10^3$         | -241          | "                                |
| 54  | $4.77 \times 10^3$         | +78           | "                                | $5.46 \times 10^3$         | -261          | "                                | $2.91 \times 10^3$         | -241          | "                                |
| 55  | $7.16 \times 10^3$         | -163          | "                                | $9.33 \times 10^3$         | -462          | "                                | $7.28 \times 10^3$         | -298          | "                                |
| 56  | $4.81 \times 10^3$         | -82           | "                                | $6.42 \times 10^3$         | -419          | "                                | $4.99 \times 10^3$         | -636          | "                                |
| 57  | $7.22 \times 10^3$         | -184          | "                                | $10.2 \times 10^3$         | -497          | "                                | $7.30 \times 10^3$         | -936          | "                                |
| 58  | $4.93 \times 10^3$         | -93           | "                                | $7.21 \times 10^3$         | -444          | "                                | $5.05 \times 10^3$         | -640          | "                                |
| 59  | $6.13 \times 10^3$         | -121          | "                                | $8.25 \times 10^3$         | -498          | "                                | $7.02 \times 10^3$         | -887          | "                                |
| 60  | $6.01 \times 10^3$         | -105          | "                                | $8.43 \times 10^3$         | -499          | "                                | $3.42 \times 10^3$         | -524          | "                                |
| 61  | $3.87 \times 10^3$         | +53           | "                                | $7.91 \times 10^3$         | -497          | "                                | $3.21 \times 10^3$         | -502          | "                                |
| 62  | $3.62 \times 10^3$         | +77           | "                                | $7.62 \times 10^3$         | -496          | "                                | $4.67 \times 10^3$         | -611          | "                                |
| 63  | $3.14 \times 10^3$         | +68           | "                                | $6.41 \times 10^3$         | -490          | "                                | $3.33 \times 10^3$         | -512          | "                                |
| 64  | $3.00 \times 10^3$         | +85           | "                                | $6.15 \times 10^3$         | -489          | "                                | $2.64 \times 10^3$         | -499          | "                                |
| 65  | $6.24 \times 10^3$         | -135          | "                                | $7.32 \times 10^3$         | -495          | "                                | $3.42 \times 10^3$         | -524          | "                                |
| 66  | $4.07 \times 10^3$         | +5            | "                                | $7.04 \times 10^3$         | -494          | "                                | $4.67 \times 10^3$         | -611          | "                                |
| 67  | $5.85 \times 10^3$         | -85           | "                                | $6.02 \times 10^3$         | -488          | "                                | $3.42 \times 10^3$         | -524          | "                                |
| 68  | $3.41 \times 10^3$         | +58           | "                                | $6.52 \times 10^3$         | +491          | "                                | $4.67 \times 10^3$         | -611          | "                                |
| 69  | $5.67 \times 10^3$         | -18           | "                                | $5.88 \times 10^3$         | -487          | "                                | $3.42 \times 10^3$         | -524          | "                                |
| 70  | $3.29 \times 10^3$         | +60           | "                                | $6.72 \times 10^3$         | -492          | "                                | $4.67 \times 10^3$         | -611          | "                                |
| 71  | $4.33 \times 10^3$         | -52           | "                                | $6.83 \times 10^3$         | -493          | "                                | $3.21 \times 10^3$         | -502          | "                                |
| 72  | $3.68 \times 10^3$         | +21           | "                                | $6.39 \times 10^3$         | -490          | "                                | $3.33 \times 10^3$         | -512          | "                                |
| 73  | $3.99 \times 10^3$         | +18           | "                                | $4.86 \times 10^3$         | -468          | "                                | $3.21 \times 10^3$         | -468          | "                                |
| 74  | $3.31 \times 10^3$         | +28           | "                                | $5.25 \times 10^3$         | -478          | "                                | $3.33 \times 10^3$         | -478          | "                                |
| 75  | $4.18 \times 10^3$         | -20           | "                                | $5.06 \times 10^3$         | -472          | "                                | $3.21 \times 10^3$         | -472          | "                                |
| 76  | $3.54 \times 10^3$         | +40           | "                                | $5.45 \times 10^3$         | -479          | "                                | $3.33 \times 10^3$         | -479          | "                                |
| 77  | $3.08 \times 10^3$         | +72           | "                                | $5.61 \times 10^3$         | -481          | "                                | $3.33 \times 10^3$         | -481          | "                                |
| 78  | $3.20 \times 10^3$         | +70           | "                                | $5.24 \times 10^3$         | -478          | "                                | $3.33 \times 10^3$         | -478          | "                                |
| 79  | $3.49 \times 10^3$         | +20           | "                                | $5.16 \times 10^3$         | -476          | "                                | $3.33 \times 10^3$         | -476          | "                                |
| 80  | $3.10 \times 10^3$         | +166          | "                                | $4.74 \times 10^3$         | -467          | "                                | $3.00 \times 10^3$         | -467          | "                                |
| 81  | $4.02 \times 10^3$         | +172          | "                                | $6.14 \times 10^3$         | -492          | "                                | $3.82 \times 10^3$         | -477          | "                                |
| 82  | $3.48 \times 10^3$         | +159          | "                                | $3.98 \times 10^3$         | -398          | "                                | $3.04 \times 10^3$         | -501          | "                                |
| 83  | $3.84 \times 10^3$         | +144          | "                                | $4.52 \times 10^3$         | -456          | "                                | $3.16 \times 10^3$         | -504          | "                                |

TABLE 12

(Characteristic values corresponding to the sample in Table 4)

| Nos | Example 1                  |               |                                  | Carbonate-Free             |               |                                  | Carbonate & Fluoride-Free  |               |                                  |
|-----|----------------------------|---------------|----------------------------------|----------------------------|---------------|----------------------------------|----------------------------|---------------|----------------------------------|
|     | Resistance value at 25° C. | TCR (ppm/°C.) | Rate of Change in Resistance (%) | Resistance value at 25° C. | TCR (ppm/°C.) | Rate of Change in Resistance (%) | Resistance value at 25° C. | TCR (ppm/°C.) | Rate of Change in Resistance (%) |
| 1   | $20.3 \times 10^3$         | -289          | < ±2                             | $26.3 \times 10^3$         | -986          | < ±2                             | $25.4 \times 10^3$         | -986          | < ±2                             |
| 2   | $17.5 \times 10^3$         | -278          | "                                | $22.5 \times 10^3$         | -887          | "                                | $21.7 \times 10^3$         | -877          | "                                |
| 3   | $13.2 \times 10^3$         | -252          | "                                | $19.3 \times 10^3$         | -805          | "                                | $18.4 \times 10^3$         | -805          | "                                |
| 4   | $5.34 \times 10^3$         | -190          | "                                | $10.3 \times 10^3$         | -681          | "                                | $9.26 \times 10^3$         | -681          | "                                |
| 5   | $21.5 \times 10^3$         | -285          | "                                | $27.5 \times 10^3$         | -995          | "                                | $26.4 \times 10^3$         | -995          | "                                |
| 6   | $18.4 \times 10^3$         | -275          | "                                | $23.1 \times 10^3$         | -880          | "                                | $22.3 \times 10^3$         | -880          | "                                |
| 7   | $14.9 \times 10^3$         | -250          | "                                | $19.8 \times 10^3$         | -803          | "                                | $19.0 \times 10^3$         | -803          | "                                |
| 8   | $4.25 \times 10^3$         | -187          | "                                | $10.1 \times 10^3$         | -684          | "                                | $9.77 \times 10^3$         | -684          | "                                |
| 9   | $15.3 \times 10^3$         | -265          | "                                | $19.2 \times 10^3$         | -804          | "                                | $18.8 \times 10^3$         | -804          | "                                |
| 10  | $15.1 \times 10^3$         | -285          | "                                | $23.6 \times 10^3$         | -418          | "                                | $21.4 \times 10^3$         | -842          | "                                |
| 11  | $13.9 \times 10^3$         | -249          | "                                | $16.4 \times 10^3$         | -376          | "                                | $17.3 \times 10^3$         | -794          | "                                |
| 12  | $11.5 \times 10^3$         | -218          | "                                | $15.2 \times 10^3$         | -351          | "                                | $14.6 \times 10^3$         | -693          | "                                |
| 13  | $9.84 \times 10^3$         | -205          | "                                | $17.6 \times 10^3$         | -402          | "                                | $16.9 \times 10^3$         | -761          | "                                |
| 14  | $8.07 \times 10^3$         | -188          | "                                | $9.31 \times 10^3$         | -598          | "                                | $9.48 \times 10^3$         | -652          | "                                |
| 15  | $16.3 \times 10^3$         | -297          | "                                | $20.3 \times 10^3$         | -783          | "                                | $21.4 \times 10^3$         | -842          | "                                |
| 16  | $14.7 \times 10^3$         | -259          | "                                | $16.8 \times 10^3$         | -428          | "                                | $17.3 \times 10^3$         | -794          | "                                |
| 17  | $12.7 \times 10^3$         | -231          | "                                | $15.4 \times 10^3$         | -398          | "                                | $14.6 \times 10^3$         | -693          | "                                |
| 18  | $10.4 \times 10^3$         | -227          | "                                | $14.9 \times 10^3$         | -372          | "                                | $16.9 \times 10^3$         | -761          | "                                |
| 19  | $8.65 \times 10^3$         | -205          | "                                | $9.72 \times 10^3$         | -481          | "                                | $9.48 \times 10^3$         | -652          | "                                |
| 20  | $13.9 \times 10^3$         | -261          | "                                | $15.2 \times 10^3$         | -384          | "                                | $14.6 \times 10^3$         | -693          | "                                |
| 21  | $13.4 \times 10^3$         | -268          | "                                | $15.8 \times 10^3$         | -402          | "                                | $16.9 \times 10^3$         | -761          | "                                |
| 22  | $12.3 \times 10^3$         | -242          | "                                | $14.4 \times 10^3$         | -369          | "                                | $14.6 \times 10^3$         | -693          | "                                |
| 23  | $10.7 \times 10^3$         | -225          | "                                | $15.5 \times 10^3$         | -401          | "                                | $16.9 \times 10^3$         | -761          | "                                |
| 24  | $12.9 \times 10^3$         | -243          | "                                | $13.9 \times 10^3$         | -340          | "                                | $14.6 \times 10^3$         | -693          | "                                |
| 25  | $11.8 \times 10^3$         | -236          | "                                | $15.1 \times 10^3$         | -377          | "                                | $16.9 \times 10^3$         | -761          | "                                |
| 26  | $12.7 \times 10^3$         | -240          | "                                | $14.2 \times 10^3$         | -358          | "                                | $14.6 \times 10^3$         | -693          | "                                |
| 27  | $10.7 \times 10^3$         | -235          | "                                | $14.9 \times 10^3$         | -373          | "                                | $16.9 \times 10^3$         | -761          | "                                |
| 28  | $10.4 \times 10^3$         | -205          | "                                | $14.3 \times 10^3$         | -364          | "                                | $14.6 \times 10^3$         | -693          | "                                |
| 29  | $9.12 \times 10^3$         | -207          | "                                | $15.9 \times 10^3$         | -418          | "                                | $16.9 \times 10^3$         | -761          | "                                |
| 30  | $9.03 \times 10^3$         | -198          | "                                | $14.5 \times 10^3$         | -370          | "                                | $14.6 \times 10^3$         | -693          | "                                |
| 31  | $8.88 \times 10^3$         | -191          | "                                | $13.4 \times 10^3$         | -314          | "                                | $16.9 \times 10^3$         | -761          | "                                |
| 32  | $12.6 \times 10^3$         | -243          | "                                | $15.8 \times 10^3$         | -404          | "                                | $14.6 \times 10^3$         | -693          | "                                |
| 33  | $11.4 \times 10^3$         | -222          | "                                | $13.6 \times 10^3$         | -318          | "                                | $14.6 \times 10^3$         | -693          | "                                |
| 34  | $13.8 \times 10^3$         | -261          | "                                | $14.9 \times 10^3$         | -382          | "                                | $14.6 \times 10^3$         | -693          | "                                |
| 35  | $9.73 \times 10^3$         | -209          | "                                | $15.2 \times 10^3$         | -383          | "                                | $16.9 \times 10^3$         | -761          | "                                |

TABLE 13

(Characteristic values corresponding to the sample in Table 5)

| Nos | Example 1                  |               |                                  | Carbonate-Free             |               |                                  | Carbonate & Fluoride-Free  |               |                                  |
|-----|----------------------------|---------------|----------------------------------|----------------------------|---------------|----------------------------------|----------------------------|---------------|----------------------------------|
|     | Resistance value at 25° C. | TCR (ppm/°C.) | Rate of Change in Resistance (%) | Resistance value at 25° C. | TCR (ppm/°C.) | Rate of Change in Resistance (%) | Resistance value at 25° C. | TCR (ppm/°C.) | Rate of Change in Resistance (%) |
| 1   | $48.3 \times 10^3$         | -298          | < ±2                             | $53.8 \times 10^3$         | -483          | < ±2                             | $52.5 \times 10^3$         | -877          | < ±2                             |
| 2   | $14.8 \times 10^3$         | -273          | "                                | $19.5 \times 10^3$         | -395          | "                                | $18.9 \times 10^3$         | -580          | "                                |
| 3   | $2.54 \times 10^3$         | -93           | "                                | $6.23 \times 10^3$         | -315          | "                                | $5.81 \times 10^3$         | -416          | "                                |
| 4   | $2.19 \times 10^3$         | -90           | "                                | $3.15 \times 10^3$         | -310          | "                                | $2.30 \times 10^3$         | -304          | "                                |
| 5   | $16.2 \times 10^3$         | -279          | "                                | $20.5 \times 10^3$         | -403          | "                                | $19.3 \times 10^3$         | -576          | "                                |
| 6   | $2.80 \times 10^3$         | -95           | "                                | $6.34 \times 10^3$         | -392          | "                                | $5.79 \times 10^3$         | -415          | "                                |
| 7   | $20.1 \times 10^3$         | -292          | "                                | $26.3 \times 10^3$         | -425          | "                                | $25.3 \times 10^3$         | -685          | "                                |
| 8   | $18.5 \times 10^3$         | -281          | "                                | $22.1 \times 10^3$         | -410          | "                                | $21.6 \times 10^3$         | -675          | "                                |
| 9   | $8.78 \times 10^3$         | -195          | "                                | $9.56 \times 10^3$         | -380          | "                                | $9.26 \times 10^3$         | -525          | "                                |
| 10  | $7.96 \times 10^3$         | -197          | "                                | $9.02 \times 10^3$         | -378          | "                                | $8.92 \times 10^3$         | -518          | "                                |
| 11  | $2.01 \times 10^3$         | -105          | "                                | $3.25 \times 10^3$         | -309          | "                                | $3.03 \times 10^3$         | -403          | "                                |
| 12  | $2.00 \times 10^3$         | -98           | "                                | $2.89 \times 10^3$         | -305          | "                                | $2.84 \times 10^3$         | -398          | "                                |
| 13  | $1.12 \times 10^3$         | -45           | "                                | $2.18 \times 10^3$         | -303          | "                                | $2.13 \times 10^3$         | -387          | "                                |
| 14  | $24.3 \times 10^3$         | -298          | "                                | $26.9 \times 10^3$         | -432          | "                                | $25.3 \times 10^3$         | -685          | "                                |
| 15  | $21.8 \times 10^3$         | -290          | "                                | $23.0 \times 10^3$         | -415          | "                                | $21.6 \times 10^3$         | -675          | "                                |
| 16  | $9.95 \times 10^3$         | -225          | "                                | $9.82 \times 10^3$         | -392          | "                                | $9.26 \times 10^3$         | -525          | "                                |
| 17  | $9.03 \times 10^3$         | -221          | "                                | $9.03 \times 10^3$         | -381          | "                                | $8.92 \times 10^3$         | -518          | "                                |
| 18  | $4.68 \times 10^3$         | -185          | "                                | $3.25 \times 10^3$         | -363          | "                                | $3.03 \times 10^3$         | -403          | "                                |
| 19  | $4.41 \times 10^3$         | -168          | "                                | $3.01 \times 10^3$         | -314          | "                                | $2.84 \times 10^3$         | -398          | "                                |
| 20  | $1.85 \times 10^3$         | -62           | "                                | $2.21 \times 10^3$         | -309          | "                                | $2.13 \times 10^3$         | -387          | "                                |
| 21  | $10.08 \times 10^3$        | -223          | "                                | $9.83 \times 10^3$         | -392          | "                                | $9.26 \times 10^3$         | -525          | "                                |
| 22  | $2.38 \times 10^3$         | -114          | "                                | $3.21 \times 10^3$         | -365          | "                                | $3.03 \times 10^3$         | -403          | "                                |
| 23  | $8.14 \times 10^3$         | -186          | "                                | $9.56 \times 10^3$         | -353          | "                                | $9.26 \times 10^3$         | -525          | "                                |
| 24  | $1.95 \times 10^3$         | -106          | "                                | $3.14 \times 10^3$         | -358          | "                                | $3.03 \times 10^3$         | -403          | "                                |
| 25  | $7.68 \times 10^3$         | -181          | "                                | $9.54 \times 10^3$         | -393          | "                                | $9.26 \times 10^3$         | -525          | "                                |
| 26  | $1.88 \times 10^3$         | -99           | "                                | $3.17 \times 10^3$         | -374          | "                                | $3.03 \times 10^3$         | -403          | "                                |
| 27  | $9.84 \times 10^3$         | -200          | "                                | $9.02 \times 10^3$         | -362          | "                                | $8.92 \times 10^3$         | -518          | "                                |

TABLE 13-continued

(Characteristic values corresponding to the sample in Table 5)

| Nos | Example 1                  |               |                                  | Carbonate-Free             |               |                                  | Carbonate & Fluoride-Free  |               |                                  |
|-----|----------------------------|---------------|----------------------------------|----------------------------|---------------|----------------------------------|----------------------------|---------------|----------------------------------|
|     | Resistance value at 25° C. | TCR (ppm/°C.) | Rate of Change in Resistance (%) | Resistance value at 25° C. | TCR (ppm/°C.) | Rate of Change in Resistance (%) | Resistance value at 25° C. | TCR (ppm/°C.) | Rate of Change in Resistance (%) |
| 28  | $3.01 \times 10^3$         | -141          | "                                | $2.92 \times 10^3$         | -316          | "                                | $2.84 \times 10^3$         | -398          | "                                |
| 29  | $8.16 \times 10^3$         | -184          | "                                | $9.21 \times 10^3$         | -321          | "                                | $8.92 \times 10^3$         | -518          | "                                |
| 30  | $2.18 \times 10^3$         | -120          | "                                | $2.90 \times 10^3$         | -316          | "                                | $2.84 \times 10^3$         | -398          | "                                |
| 31  | $8.78 \times 10^3$         | -188          | "                                | $8.98 \times 10^3$         | -321          | "                                | $8.92 \times 10^3$         | -518          | "                                |
| 32  | $2.54 \times 10^3$         | -121          | "                                | $2.96 \times 10^3$         | -319          | "                                | $2.84 \times 10^3$         | -398          | "                                |
| 33  | $17.4 \times 10^3$         | -277          | "                                | $21.9 \times 10^3$         | -403          | "                                | $21.6 \times 10^3$         | -675          | "                                |
| 34  | $18.9 \times 10^3$         | -289          | "                                | $22.0 \times 10^3$         | -410          | "                                | $21.6 \times 10^3$         | -675          | "                                |
| 35  | $43.9 \times 10^3$         | -297          | "                                | $45.6 \times 10^3$         | -463          | "                                | $44.8 \times 10^3$         | -857          | "                                |
| 36  | $14.8 \times 10^3$         | -261          | "                                | $16.3 \times 10^3$         | -405          | "                                | $15.0 \times 10^3$         | -521          | "                                |
| 37  | $4.13 \times 10^3$         | -180          | "                                | $5.34 \times 10^3$         | -362          | "                                | $4.77 \times 10^3$         | -408          | "                                |
| 38  | $1.93 \times 10^3$         | -120          | "                                | $3.51 \times 10^3$         | -354          | "                                | $2.07 \times 10^3$         | -311          | "                                |
| 39  | $14.8 \times 10^3$         | -273          | "                                | $17.5 \times 10^3$         | -413          | "                                | $15.3 \times 10^3$         | -527          | "                                |
| 40  | $4.24 \times 10^3$         | -186          | "                                | $5.83 \times 10^3$         | -372          | "                                | $4.80 \times 10^3$         | -411          | "                                |
| 41  | $18.2 \times 10^3$         | -271          | "                                | $19.8 \times 10^3$         | -412          | "                                | $19.4 \times 10^3$         | -621          | "                                |
| 42  | $16.4 \times 10^3$         | -254          | "                                | $18.6 \times 10^3$         | -408          | "                                | $18.2 \times 10^3$         | -613          | "                                |
| 43  | $6.85 \times 10^3$         | -186          | "                                | $7.82 \times 10^3$         | -395          | "                                | $7.32 \times 10^3$         | -480          | "                                |
| 44  | $6.18 \times 10^3$         | -184          | "                                | $7.53 \times 10^3$         | -389          | "                                | $7.01 \times 10^3$         | -478          | "                                |
| 45  | $2.81 \times 10^3$         | -125          | "                                | $3.43 \times 10^3$         | -325          | "                                | $3.24 \times 10^3$         | -411          | "                                |
| 46  | $2.16 \times 10^3$         | -118          | "                                | $3.21 \times 10^3$         | -320          | "                                | $3.02 \times 10^3$         | -408          | "                                |
| 47  | 985                        | -15           | "                                | $1.53 \times 10^3$         | -302          | "                                | $1.21 \times 10^3$         | -398          | "                                |
| 48  | $7.90 \times 10^3$         | -197          | "                                | $7.42 \times 10^3$         | -380          | "                                | $7.32 \times 10^3$         | -480          | "                                |
| 49  | $4.11 \times 10^3$         | -174          | "                                | $3.28 \times 10^3$         | -328          | "                                | $3.24 \times 10^3$         | -411          | "                                |
| 50  | $6.99 \times 10^3$         | -181          | "                                | $7.38 \times 10^3$         | -375          | "                                | $7.32 \times 10^3$         | -480          | "                                |
| 51  | $3.05 \times 10^3$         | -155          | "                                | $3.80 \times 10^3$         | -331          | "                                | $3.24 \times 10^3$         | -411          | "                                |
| 52  | $7.41 \times 10^3$         | -192          | "                                | $7.36 \times 10^3$         | -375          | "                                | $7.32 \times 10^3$         | -480          | "                                |
| 53  | $3.40 \times 10^3$         | -148          | "                                | $3.92 \times 10^3$         | -380          | "                                | $3.24 \times 10^3$         | -411          | "                                |
| 54  | $7.10 \times 10^3$         | -189          | "                                | $7.21 \times 10^3$         | -369          | "                                | $7.01 \times 10^3$         | -478          | "                                |
| 55  | $2.99 \times 10^3$         | -133          | "                                | $3.56 \times 10^3$         | -345          | "                                | $3.02 \times 10^3$         | -408          | "                                |
| 56  | $5.84 \times 10^3$         | -170          | "                                | $7.26 \times 10^3$         | -361          | "                                | $7.01 \times 10^3$         | -478          | "                                |
| 57  | $1.95 \times 10^3$         | -119          | "                                | $3.21 \times 10^3$         | -353          | "                                | $3.02 \times 10^3$         | -408          | "                                |
| 58  | $6.65 \times 10^3$         | -179          | "                                | $7.36 \times 10^3$         | -372          | "                                | $7.01 \times 10^3$         | -478          | "                                |
| 59  | $2.45 \times 10^3$         | -130          | "                                | $3.25 \times 10^3$         | -350          | "                                | $3.02 \times 10^3$         | -408          | "                                |
| 60  | $18.6 \times 10^3$         | -283          | "                                | $19.3 \times 10^3$         | -403          | "                                | $18.2 \times 10^3$         | -613          | "                                |
| 61  | $19.1 \times 10^3$         | -290          | "                                | $18.6 \times 10^3$         | -410          | "                                | $18.2 \times 10^3$         | -613          | "                                |
| 62  | $1.66 \times 10^3$         | -105          | "                                | $2.10 \times 10^3$         | -380          | "                                | $2.06 \times 10^3$         | -487          | "                                |
| 63  | $1.59 \times 10^3$         | -100          | "                                | $2.24 \times 10^3$         | -383          | "                                | $2.15 \times 10^3$         | -498          | "                                |
| 64  | $1.76 \times 10^3$         | -109          | "                                | $1.98 \times 10^3$         | -375          | "                                | $1.92 \times 10^3$         | -478          | "                                |

TABLE 14

(Characteristic values corresponding to the sample in Table 6)

| Nos | Example 1                  |               |                                  | Carbonate-Free             |               |                                  | Carbonate & Fluoride-Free  |               |                                  |
|-----|----------------------------|---------------|----------------------------------|----------------------------|---------------|----------------------------------|----------------------------|---------------|----------------------------------|
|     | Resistance value at 25° C. | TCR (ppm/°C.) | Rate of Change in Resistance (%) | Resistance value at 25° C. | TCR (ppm/°C.) | Rate of Change in Resistance (%) | Resistance value at 25° C. | TCR (ppm/°C.) | Rate of Change in Resistance (%) |
| 1   | $83.6 \times 10^3$         | -300          | $< \pm 2$                        | $87.5 \times 10^3$         | -493          | $< \pm 2$                        | $84.3 \times 10^3$         | -989          | $< \pm 2$                        |
| 2   | $38.5 \times 10^3$         | -283          | "                                | $41.5 \times 10^3$         | -423          | "                                | $39.4 \times 10^3$         | -720          | "                                |
| 3   | $19.8 \times 10^3$         | -120          | "                                | $21.6 \times 10^3$         | -401          | "                                | $20.4 \times 10^3$         | -378          | "                                |
| 4   | $4.83 \times 10^3$         | +12           | "                                | $4.92 \times 10^3$         | -263          | "                                | $4.05 \times 10^3$         | -185          | "                                |
| 5   | $38.7 \times 10^3$         | -214          | "                                | $40.5 \times 10^3$         | -418          | "                                | $39.2 \times 10^3$         | -723          | "                                |
| 6   | $19.6 \times 10^3$         | -118          | "                                | $21.4 \times 10^3$         | -409          | "                                | $20.6 \times 10^3$         | -380          | "                                |
| 7   | $52.5 \times 10^3$         | -298          | "                                | $53.8 \times 10^3$         | -454          | "                                | $53.2 \times 10^3$         | -830          | "                                |
| 8   | $45.3 \times 10^3$         | -295          | "                                | $46.5 \times 10^3$         | -438          | "                                | $46.3 \times 10^3$         | -810          | "                                |
| 9   | $48.7 \times 10^3$         | -267          | "                                | $49.3 \times 10^3$         | -437          | "                                | $49.1 \times 10^3$         | -812          | "                                |
| 10  | $27.4 \times 10^3$         | -205          | "                                | $28.9 \times 10^3$         | -407          | "                                | $28.5 \times 10^3$         | -750          | "                                |
| 11  | $33.0 \times 10^3$         | -198          | "                                | $34.0 \times 10^3$         | -198          | "                                | $33.8 \times 10^3$         | -780          | "                                |
| 12  | $8.31 \times 10^3$         | +23           | "                                | $9.60 \times 10^3$         | -283          | "                                | $9.25 \times 10^3$         | -520          | "                                |
| 13  | $7.20 \times 10^3$         | +31           | "                                | $8.03 \times 10^3$         | -265          | "                                | $7.80 \times 10^3$         | -490          | "                                |
| 14  | $2.38 \times 10^3$         | +89           | "                                | $3.08 \times 10^3$         | -250          | "                                | $3.04 \times 10^3$         | -353          | "                                |
| 15  | $59.6 \times 10^3$         | -289          | "                                | $53.6 \times 10^3$         | -449          | "                                | $53.2 \times 10^3$         | -830          | "                                |
| 16  | $51.2 \times 10^3$         | -274          | "                                | $46.8 \times 10^3$         | -424          | "                                | $46.3 \times 10^3$         | -810          | "                                |
| 17  | $57.7 \times 10^3$         | -283          | "                                | $49.0 \times 10^3$         | -430          | "                                | $49.1 \times 10^3$         | -812          | "                                |
| 18  | $30.1 \times 10^3$         | -245          | "                                | $29.1 \times 10^3$         | -380          | "                                | $28.5 \times 10^3$         | -750          | "                                |
| 19  | $35.2 \times 10^3$         | -201          | "                                | $34.1 \times 10^3$         | -415          | "                                | $33.8 \times 10^3$         | -780          | "                                |
| 20  | $10.1 \times 10^3$         | -15           | "                                | $9.34 \times 10^3$         | -350          | "                                | $9.25 \times 10^3$         | -520          | "                                |
| 21  | $9.08 \times 10^3$         | -50           | "                                | $7.89 \times 10^3$         | -314          | "                                | $7.80 \times 10^3$         | -490          | "                                |
| 22  | $4.01 \times 10^3$         | +3            | "                                | $3.21 \times 10^3$         | -289          | "                                | $3.04 \times 10^3$         | -353          | "                                |
| 23  | $54.9 \times 10^3$         | -283          | "                                | $46.8 \times 10^3$         | -438          | "                                | $46.3 \times 10^3$         | -830          | "                                |
| 24  | $15.6 \times 10^3$         | -95           | "                                | $9.36 \times 10^3$         | -352          | "                                | $9.25 \times 10^3$         | -520          | "                                |
| 25  | $32.7 \times 10^3$         | -254          | "                                | $46.5 \times 10^3$         | -423          | "                                | $46.3 \times 10^3$         | -810          | "                                |

TABLE 14-continued

| Nos | Example 1                  |                              |     | Carbonate-Free             |                              |     | Carbonate & Fluoride-Free  |                              |     |
|-----|----------------------------|------------------------------|-----|----------------------------|------------------------------|-----|----------------------------|------------------------------|-----|
|     | Resistance value at 25° C. | Rate of Change in Resistance | TCR | Resistance value at 25° C. | Rate of Change in Resistance | TCR | Resistance value at 25° C. | Rate of Change in Resistance | TCR |
|     | R <sub>25</sub> (Ω)        | (ppm/°C.)                    | (%) | R <sub>25</sub> (Ω)        | (ppm/°C.)                    | (%) | R <sub>25</sub> (Ω)        | (ppm/°C.)                    | (%) |
| 26  | 5.23 × 10 <sup>3</sup>     | -18                          | "   | 9.30 × 10 <sup>3</sup>     | -273                         | "   | 9.25 × 10 <sup>3</sup>     | -520                         | "   |
| 27  | 47.4 × 10 <sup>3</sup>     | -270                         | "   | 46.5 × 10 <sup>3</sup>     | -430                         | "   | 46.3 × 10 <sup>3</sup>     | -830                         | "   |
| 28  | 9.98 × 10 <sup>3</sup>     | -78                          | "   | 9.31 × 10 <sup>3</sup>     | -360                         | "   | 9.25 × 10 <sup>3</sup>     | -520                         | "   |
| 29  | 47.3 × 10 <sup>3</sup>     | -272                         | "   | 33.9 × 10 <sup>3</sup>     | -416                         | "   | 33.8 × 10 <sup>3</sup>     | -780                         | "   |
| 30  | 18.0 × 10 <sup>3</sup>     | -105                         | "   | 9.35 × 10 <sup>3</sup>     | -370                         | "   | 9.25 × 10 <sup>3</sup>     | -520                         | "   |
| 31  | 35.2 × 10 <sup>3</sup>     | -187                         | "   | 33.2 × 10 <sup>3</sup>     | -421                         | "   | 33.8 × 10 <sup>3</sup>     | -780                         | "   |
| 32  | 9.51 × 10 <sup>3</sup>     | -5                           | "   | 8.93 × 10 <sup>3</sup>     | -320                         | "   | 9.25 × 10 <sup>3</sup>     | -520                         | "   |
| 33  | 37.0 × 10 <sup>3</sup>     | -201                         | "   | 34.1 × 10 <sup>3</sup>     | -431                         | "   | 33.8 × 10 <sup>3</sup>     | -780                         | "   |
| 34  | 11.3 × 10 <sup>3</sup>     | -11                          | "   | 9.25 × 10 <sup>3</sup>     | -368                         | "   | 9.25 × 10 <sup>3</sup>     | -520                         | "   |
| 35  | 46.8 × 10 <sup>3</sup>     | -300                         | "   | 45.9 × 10 <sup>3</sup>     | -433                         | "   | 46.3 × 10 <sup>3</sup>     | -810                         | "   |
| 36  | 48.5 × 10 <sup>3</sup>     | -295                         | "   | 46.4 × 10 <sup>3</sup>     | -430                         | "   | 46.3 × 10 <sup>3</sup>     | -810                         | "   |
| 37  | 43.3 × 10 <sup>3</sup>     | -280                         | "   | 46.8 × 10 <sup>3</sup>     | -435                         | "   | 46.3 × 10 <sup>3</sup>     | -810                         | "   |
| 38  | 42.9 × 10 <sup>3</sup>     | -283                         | "   | 45.8 × 10 <sup>3</sup>     | -429                         | "   | 46.3 × 10 <sup>3</sup>     | -810                         | "   |
| 39  | 67.1 × 10 <sup>3</sup>     | -299                         | "   | 71.2 × 10 <sup>3</sup>     | -498                         | "   | 70.1 × 10 <sup>3</sup>     | -995                         | "   |
| 40  | 25.6 × 10 <sup>3</sup>     | -154                         | "   | 29.3 × 10 <sup>3</sup>     | -408                         | "   | 28.4 × 10 <sup>3</sup>     | -788                         | "   |
| 41  | 16.8 × 10 <sup>3</sup>     | -121                         | "   | 18.1 × 10 <sup>3</sup>     | -374                         | "   | 17.7 × 10 <sup>3</sup>     | -385                         | "   |
| 42  | 2.13 × 10 <sup>3</sup>     | -62                          | "   | 3.21 × 10 <sup>3</sup>     | -270                         | "   | 2.95 × 10 <sup>3</sup>     | -207                         | "   |
| 43  | 27.1 × 10 <sup>3</sup>     | -156                         | "   | 29.5 × 10 <sup>3</sup>     | -412                         | "   | 28.2 × 10 <sup>3</sup>     | -790                         | "   |
| 44  | 16.4 × 10 <sup>3</sup>     | -128                         | "   | 18.4 × 10 <sup>3</sup>     | -368                         | "   | 17.6 × 10 <sup>3</sup>     | -381                         | "   |
| 45  | 45.5 × 10 <sup>3</sup>     | -284                         | "   | 48.9 × 10 <sup>3</sup>     | -425                         | "   | 48.6 × 10 <sup>3</sup>     | -825                         | "   |
| 46  | 37.9 × 10 <sup>3</sup>     | -217                         | "   | 39.0 × 10 <sup>3</sup>     | -416                         | "   | 38.2 × 10 <sup>3</sup>     | -810                         | "   |
| 47  | 41.5 × 10 <sup>3</sup>     | -254                         | "   | 42.8 × 10 <sup>3</sup>     | -421                         | "   | 42.1 × 10 <sup>3</sup>     | -819                         | "   |
| 48  | 19.8 × 10 <sup>3</sup>     | -101                         | "   | 20.8 × 10 <sup>3</sup>     | -382                         | "   | 20.3 × 10 <sup>3</sup>     | -780                         | "   |
| 49  | 25.5 × 10 <sup>3</sup>     | -137                         | "   | 26.5 × 10 <sup>3</sup>     | -393                         | "   | 26.3 × 10 <sup>3</sup>     | -789                         | "   |
| 50  | 5.11 × 10 <sup>3</sup>     | -95                          | "   | 6.23 × 10 <sup>3</sup>     | -283                         | "   | 6.03 × 10 <sup>3</sup>     | -310                         | "   |
| 51  | 4.78 × 10 <sup>3</sup>     | -73                          | "   | 5.34 × 10 <sup>3</sup>     | -279                         | "   | 5.05 × 10 <sup>3</sup>     | -308                         | "   |
| 52  | 1.09 × 10 <sup>3</sup>     | -25                          | "   | 2.10 × 10 <sup>3</sup>     | -268                         | "   | 2.09 × 10 <sup>3</sup>     | -280                         | "   |
| 53  | 6.95 × 10 <sup>3</sup>     | -105                         | "   | 5.21 × 10 <sup>3</sup>     | -280                         | "   | 5.05 × 10 <sup>3</sup>     | -310                         | "   |
| 54  | 39.4 × 10 <sup>3</sup>     | -219                         | "   | 38.4 × 10 <sup>3</sup>     | -420                         | "   | 38.2 × 10 <sup>3</sup>     | -815                         | "   |
| 55  | 38.1 × 10 <sup>3</sup>     | -183                         | "   | 38.6 × 10 <sup>3</sup>     | -425                         | "   | 38.2 × 10 <sup>3</sup>     | -804                         | "   |
| 56  | 36.8 × 10 <sup>3</sup>     | -195                         | "   | 37.9 × 10 <sup>3</sup>     | -418                         | "   | 38.2 × 10 <sup>3</sup>     | -809                         | "   |
| 57  | 26.5 × 10 <sup>3</sup>     | -295                         | "   | 28.8 × 10 <sup>3</sup>     | -489                         | "   | 27.1 × 10 <sup>3</sup>     | -849                         | "   |
| 58  | 16.2 × 10 <sup>3</sup>     | -286                         | "   | 18.2 × 10 <sup>3</sup>     | -465                         | "   | 17.1 × 10 <sup>3</sup>     | -452                         | "   |
| 59  | 6.81 × 10 <sup>3</sup>     | -267                         | "   | 7.43 × 10 <sup>3</sup>     | -378                         | "   | 7.34 × 10 <sup>3</sup>     | -424                         | "   |
| 60  | 22.4 × 10 <sup>3</sup>     | -284                         | "   | 24.8 × 10 <sup>3</sup>     | -412                         | "   | 23.7 × 10 <sup>3</sup>     | -784                         | "   |
| 61  | 13.8 × 10 <sup>3</sup>     | -253                         | "   | 15.4 × 10 <sup>3</sup>     | -324                         | "   | 14.6 × 10 <sup>3</sup>     | -382                         | "   |
| 62  | 5.32 × 10 <sup>3</sup>     | -218                         | "   | 5.92 × 10 <sup>3</sup>     | -295                         | "   | 5.82 × 10 <sup>3</sup>     | -316                         | "   |
| 63  | 41.6 × 10 <sup>3</sup>     | -254                         | "   | 43.8 × 10 <sup>3</sup>     | -454                         | "   | 42.5 × 10 <sup>3</sup>     | -573                         | "   |
| 64  | 27.2 × 10 <sup>3</sup>     | -180                         | "   | 29.6 × 10 <sup>3</sup>     | -398                         | "   | 28.8 × 10 <sup>3</sup>     | -375                         | "   |
| 65  | 9.53 × 10 <sup>3</sup>     | +88                          | "   | 8.95 × 10 <sup>3</sup>     | -314                         | "   | 9.82 × 10 <sup>3</sup>     | -306                         | "   |
| 66  | 23.4 × 10 <sup>3</sup>     | -263                         | "   | 25.3 × 10 <sup>3</sup>     | -263                         | "   | 24.0 × 10 <sup>3</sup>     | -501                         | "   |
| 67  | 14.1 × 10 <sup>3</sup>     | -201                         | "   | 15.9 × 10 <sup>3</sup>     | -201                         | "   | 15.4 × 10 <sup>3</sup>     | -328                         | "   |
| 68  | 5.73 × 10 <sup>3</sup>     | -88                          | "   | 6.25 × 10 <sup>3</sup>     | -254                         | "   | 6.15 × 10 <sup>3</sup>     | -287                         | "   |
| 69  | 24.1 × 10 <sup>3</sup>     | -526                         | "   | 26.4 × 10 <sup>3</sup>     | -526                         | "   | 25.7 × 10 <sup>3</sup>     | -526                         | "   |
| 70  | 15.2 × 10 <sup>3</sup>     | -349                         | "   | 15.2 × 10 <sup>3</sup>     | -349                         | "   | 16.6 × 10 <sup>3</sup>     | -349                         | "   |
| 71  | 6.69 × 10 <sup>3</sup>     | -104                         | "   | 7.41 × 10 <sup>3</sup>     | -295                         | "   | 7.32 × 10 <sup>3</sup>     | -324                         | "   |
| 72  | 38.6 × 10 <sup>3</sup>     | -253                         | "   | 40.3 × 10 <sup>3</sup>     | -418                         | "   | 39.4 × 10 <sup>3</sup>     | -485                         | "   |
| 73  | 27.5 × 10 <sup>3</sup>     | -180                         | "   | 29.5 × 10 <sup>3</sup>     | -384                         | "   | 28.4 × 10 <sup>3</sup>     | -366                         | "   |
| 74  | 8.32 × 10 <sup>3</sup>     | +91                          | "   | 9.14 × 10 <sup>3</sup>     | -214                         | "   | 9.03 × 10 <sup>3</sup>     | -343                         | "   |
| 75  | 30.4 × 10 <sup>3</sup>     | -284                         | "   | 32.4 × 10 <sup>3</sup>     | -462                         | "   | 31.0 × 10 <sup>3</sup>     | -796                         | "   |
| 76  | 18.6 × 10 <sup>3</sup>     | -235                         | "   | 20.5 × 10 <sup>3</sup>     | -390                         | "   | 19.5 × 10 <sup>3</sup>     | -391                         | "   |
| 77  | 7.71 × 10 <sup>3</sup>     | -203                         | "   | 8.21 × 10 <sup>3</sup>     | -283                         | "   | 8.64 × 10 <sup>3</sup>     | -312                         | "   |
| 78  | 39.6 × 10 <sup>3</sup>     | -180                         | "   | 41.6 × 10 <sup>3</sup>     | -254                         | "   | 40.8 × 10 <sup>3</sup>     | -299                         | "   |
| 79  | 31.5 × 10 <sup>3</sup>     | -174                         | "   | 33.5 × 10 <sup>3</sup>     | -209                         | "   | 32.2 × 10 <sup>3</sup>     | -284                         | "   |
| 80  | 8.54 × 10 <sup>3</sup>     | +95                          | "   | 9.15 × 10 <sup>3</sup>     | -196                         | "   | 9.03 × 10 <sup>3</sup>     | -254                         | "   |
| 81  | 33.4 × 10 <sup>3</sup>     | -263                         | "   | 35.3 × 10 <sup>3</sup>     | -435                         | "   | 34.3 × 10 <sup>3</sup>     | -511                         | "   |
| 82  | 19.6 × 10 <sup>3</sup>     | -242                         | "   | 21.9 × 10 <sup>3</sup>     | -353                         | "   | 20.8 × 10 <sup>3</sup>     | -360                         | "   |
| 83  | 7.51 × 10 <sup>3</sup>     | -195                         | "   | 8.24 × 10 <sup>3</sup>     | -286                         | "   | 8.20 × 10 <sup>3</sup>     | -313                         | "   |
| 84  | 44.8 × 10 <sup>3</sup>     | -294                         | "   | 46.8 × 10 <sup>3</sup>     | -463                         | "   | 45.5 × 10 <sup>3</sup>     | -775                         | "   |
| 85  | 32.8 × 10 <sup>3</sup>     | -281                         | "   | 34.3 × 10 <sup>3</sup>     | -401                         | "   | 33.1 × 10 <sup>3</sup>     | -381                         | "   |
| 86  | 9.11 × 10 <sup>3</sup>     | -240                         | "   | 9.8 × 10 <sup>3</sup>      | -2931                        | "   | 10.3 × 10 <sup>3</sup>     | -329                         | "   |
| 87  | 34.3 × 10 <sup>3</sup>     | -285                         | "   | 36.5 × 10 <sup>3</sup>     | -459                         | "   | 35.1 × 10 <sup>3</sup>     | -769                         | "   |
| 88  | 24.5 × 10 <sup>3</sup>     | -239                         | "   | 26.8 × 10 <sup>3</sup>     | -375                         | "   | 25.4 × 10 <sup>3</sup>     | -375                         | "   |
| 89  | 7.87 × 10 <sup>3</sup>     | -176                         | "   | 8.14 × 10 <sup>3</sup>     | -275                         | "   | 8.03 × 10 <sup>3</sup>     | -352                         | "   |
| 90  | 28.4 × 10 <sup>3</sup>     | -287                         | "   | 30.5 × 10 <sup>3</sup>     | -469                         | "   | 29.6 × 10 <sup>3</sup>     | -789                         | "   |
| 91  | 18.5 × 10 <sup>3</sup>     | -453                         | "   | 20.9 × 10 <sup>3</sup>     | -353                         | "   | 19.8 × 10 <sup>3</sup>     | -384                         | "   |
| 92  | 5.43 × 10 <sup>3</sup>     | -224                         | "   | 6.12 × 10 <sup>3</sup>     | -302                         | "   | 6.25 × 10 <sup>3</sup>     | -363                         | "   |
| 93  | 26.3 × 10 <sup>3</sup>     | -282                         | "   | 28.6 × 10 <sup>3</sup>     | -434                         | "   | 27.0 × 10 <sup>3</sup>     | -600                         | "   |
| 94  | 15.2 × 10 <sup>3</sup>     | -253                         | "   | 17.8 × 10 <sup>3</sup>     | -319                         | "   | 16.4 × 10 <sup>3</sup>     | -321                         | "   |
| 95  | 5.43 × 10 <sup>3</sup>     | -224                         | "   | 5.58 × 10 <sup>3</sup>     | -264                         | "   | 5.63 × 10 <sup>3</sup>     | -302                         | "   |
| 96  | 28.3 × 10 <sup>3</sup>     | -186                         | "   | 31.5 × 10 <sup>3</sup>     | -353                         | "   | 18.4 × 10 <sup>3</sup>     | -441                         | "   |
| 97  | 26.5 × 10 <sup>3</sup>     | -215                         | "   | 24.6 × 10 <sup>3</sup>     | -321                         | "   | 15.3 × 10 <sup>3</sup>     | -425                         | "   |
| 98  | 32.8 × 10 <sup>3</sup>     | -255                         | "   | 33.1 × 10 <sup>3</sup>     | -189                         | "   | 29.5 × 10 <sup>3</sup>     | -295                         | "   |
| 99  | 31.1 × 10 <sup>3</sup>     | -281                         | "   | 30.5 × 10 <sup>3</sup>     | -340                         | "   | 30.0 × 10 <sup>3</sup>     | -518                         | "   |

TABLE 14-continued

(Characteristic values corresponding to the sample in Table 6)

| Nos | Example 1                                      |                                            |     | Carbonate-Free                                 |               |     | Carbonate & Fluoride-Free                      |               |     |
|-----|------------------------------------------------|--------------------------------------------|-----|------------------------------------------------|---------------|-----|------------------------------------------------|---------------|-----|
|     | Resistance value at 25° C. R <sub>25</sub> (Ω) | Rate of Change in Resistance TCR (ppm/°C.) | (%) | Resistance value at 25° C. R <sub>25</sub> (Ω) | TCR (ppm/°C.) | (%) | Resistance value at 25° C. R <sub>25</sub> (Ω) | TCR (ppm/°C.) | (%) |
| 100 | $32.5 \times 10^3$                             | -296                                       | "   | $31.1 \times 10^3$                             | -290          | "   | $23.4 \times 10^3$                             | -399          | "   |
| 101 | $7.35 \times 10^3$                             | -58                                        | "   | $8.44 \times 10^3$                             | -159          | "   | $4.90 \times 10^3$                             | -365          | "   |
| 102 | $8.03 \times 10^3$                             | -103                                       | "   | $8.33 \times 10^3$                             | -353          | "   | $4.62 \times 10^3$                             | -521          | "   |
| 103 | $9.46 \times 10^3$                             | -59                                        | "   | $11.5 \times 10^3$                             | -197          | "   | $5.51 \times 10^3$                             | -403          | "   |
| 104 | $11.5 \times 10^3$                             | -206                                       | "   | $13.0 \times 10^3$                             | -395          | "   | $7.70 \times 10^3$                             | -530          | "   |
| 105 | $7.48 \times 10^3$                             | -251                                       | "   | $8.15 \times 10^3$                             | -420          | "   | $4.80 \times 10^3$                             | -565          | "   |

TABLE 15

(Characteristics values corresponding to the sample in Table 7)

| Nos | Example 1                                      |                                            |     | Carbonate-Free                                 |               |     | Carbonate & Fluoride-Free                      |               |     |
|-----|------------------------------------------------|--------------------------------------------|-----|------------------------------------------------|---------------|-----|------------------------------------------------|---------------|-----|
|     | Resistance value at 25° C. R <sub>25</sub> (Ω) | Rate of Change in Resistance TCR (ppm/°C.) | (%) | Resistance value at 25° C. R <sub>25</sub> (Ω) | TCR (ppm/°C.) | (%) | Resistance value at 25° C. R <sub>25</sub> (Ω) | TCR (ppm/°C.) | (%) |
| 1   | $2.03 \times 10^3$                             | +193                                       | <±2 | $8.01 \times 10^3$                             | +304          | <±2 | $2.87 \times 10^3$                             | +307          | <±2 |
| 2   | 923                                            | +210                                       | "   | $1.53 \times 10^3$                             | +318          | "   | $1.09 \times 10^3$                             | +395          | "   |
| 3   | 710                                            | +235                                       | "   | 811                                            | +412          | "   | 781                                            | +480          | "   |
| 4   | 493                                            | +280                                       | "   | 583                                            | +431          | "   | 527                                            | +545          | "   |
| 5   | 963                                            | +205                                       | "   | $1.23 \times 10^3$                             | +320          | "   | $1.05 \times 10^3$                             | +400          | "   |
| 6   | 720                                            | +215                                       | "   | 803                                            | +390          | "   | 780                                            | +475          | "   |
| 7   | 893                                            | +203                                       | "   | $1.99 \times 10^3$                             | +315          | "   | $1.96 \times 10^3$                             | +348          | "   |
| 8   | 818                                            | +218                                       | "   | 556                                            | +426          | "   | 545                                            | +529          | "   |
| 9   | 625                                            | +244                                       | "   | 701                                            | +405          | "   | 703                                            | +503          | "   |
| 10  | 631                                            | +241                                       | "   | 707                                            | +401          | "   | 703                                            | +503          | "   |
| 11  | 321                                            | +285                                       | "   | 572                                            | +4161         | "   | 566                                            | +514          | "   |
| 12  | 218                                            | +299                                       | "   | 503                                            | +386          | "   | 524                                            | +541          | "   |
| 13  | 595                                            | +275                                       | "   | 701                                            | +405          | "   | 703                                            | +503          | "   |
| 14  | 308                                            | +281                                       | "   | 572                                            | +416          | "   | 566                                            | +514          | "   |
| 15  | 583                                            | +276                                       | "   | 701                                            | +405          | "   | 703                                            | +503          | "   |
| 16  | 300                                            | +280                                       | "   | 572                                            | +416          | "   | 566                                            | +514          | "   |
| 17  | 610                                            | +279                                       | "   | 701                                            | +405          | "   | 703                                            | +503          | "   |
| 18  | 318                                            | +286                                       | "   | 572                                            | +416          | "   | 566                                            | +514          | "   |
| 19  | 925                                            | +203                                       | "   | 580                                            | +422          | "   | 545                                            | +529          | "   |
| 20  | 781                                            | +218                                       | "   | 699                                            | +403          | "   | 703                                            | +503          | "   |
| 21  | 785                                            | +228                                       | "   | 571                                            | +425          | "   | 545                                            | +529          | "   |
| 22  | 523                                            | +248                                       | "   | 678                                            | +409          | "   | 703                                            | +503          | "   |
| 23  | 712                                            | +251                                       | "   | 559                                            | +414          | "   | 545                                            | +529          | "   |
| 24  | 455                                            | +263                                       | "   | 650                                            | +400          | "   | 703                                            | +503          | "   |
| 25  | 585                                            | +269                                       | "   | 685                                            | +410          | "   | 703                                            | +503          | "   |
| 26  | 564                                            | +268                                       | "   | 671                                            | +405          | "   | 703                                            | +503          | "   |
| 27  | $5.85 \times 10^3$                             | -298                                       | "   | $7.25 \times 10^3$                             | -483          | "   | $6.14 \times 10^3$                             | -705          | "   |
| 28  | $3.23 \times 10^3$                             | -284                                       | "   | $4.26 \times 10^3$                             | -448          | "   | $3.88 \times 10^3$                             | -509          | "   |
| 29  | $1.84 \times 10^3$                             | -283                                       | "   | $2.62 \times 10^3$                             | -431          | "   | $2.17 \times 10^3$                             | -417          | "   |
| 30  | 814                                            | -163                                       | "   | 893                                            | -285          | "   | 866                                            | -284          | "   |
| 31  | $3.10 \times 10^3$                             | -276                                       | "   | $4.21 \times 10^3$                             | -451          | "   | $3.90 \times 10^3$                             | -515          | "   |
| 32  | $1.94 \times 10^3$                             | -284                                       | "   | $2.85 \times 10^3$                             | -436          | "   | $2.18 \times 10^3$                             | -421          | "   |
| 33  | $2.03 \times 10^3$                             | -299                                       | "   | $5.07 \times 10^3$                             | -452          | "   | $5.14 \times 10^3$                             | -618          | "   |
| 34  | $1.86 \times 10^3$                             | -286                                       | "   | $1.48 \times 10^3$                             | -303          | "   | $1.02 \times 10^3$                             | -326          | "   |
| 35  | $1.03 \times 10^3$                             | -251                                       | "   | $1.52 \times 10^3$                             | -301          | "   | $1.50 \times 10^3$                             | -347          | "   |
| 36  | $1.02 \times 10^3$                             | -233                                       | "   | $1.47 \times 10^3$                             | -316          | "   | $1.50 \times 10^3$                             | -347          | "   |
| 37  | 985                                            | -185                                       | "   | $1.14 \times 10^3$                             | -281          | "   | $1.07 \times 10^3$                             | -334          | "   |
| 38  | 818                                            | -135                                       | "   | 886                                            | -251          | "   | 902                                            | -295          | "   |
| 39  | $1.48 \times 10^3$                             | -281                                       | "   | $1.52 \times 10^3$                             | -301          | "   | $1.50 \times 10^3$                             | -347          | "   |
| 40  | $1.25 \times 10^3$                             | -220                                       | "   | $1.14 \times 10^3$                             | -281          | "   | $1.07 \times 10^3$                             | -334          | "   |
| 41  | $1.11 \times 10^3$                             | -256                                       | "   | $1.52 \times 10^3$                             | -301          | "   | $1.50 \times 10^3$                             | -347          | "   |
| 42  | $1.03 \times 10^3$                             | -188                                       | "   | $1.14 \times 10^3$                             | -281          | "   | $1.07 \times 10^3$                             | -334          | "   |
| 43  | $1.23 \times 10^3$                             | -248                                       | "   | $1.52 \times 10^3$                             | -301          | "   | $1.50 \times 10^3$                             | -347          | "   |
| 44  | $1.09 \times 10^3$                             | -195                                       | "   | $1.14 \times 10^3$                             | -281          | "   | $1.07 \times 10^3$                             | -334          | "   |
| 45  | $1.90 \times 10^3$                             | -299                                       | "   | $1.55 \times 10^3$                             | -314          | "   | $1.02 \times 10^3$                             | -326          | "   |
| 46  | $2.54 \times 10^3$                             | -273                                       | "   | $1.86 \times 10^3$                             | -295          | "   | $1.50 \times 10^3$                             | -314          | "   |
| 47  | $1.28 \times 10^3$                             | -249                                       | "   | $1.35 \times 10^3$                             | -288          | "   | $1.02 \times 10^3$                             | -326          | "   |
| 48  | 980                                            | -203                                       | "   | $1.38 \times 10^3$                             | -256          | "   | $1.50 \times 10^3$                             | -341          | "   |
| 49  | $2.05 \times 10^3$                             | -285                                       | "   | $1.56 \times 10^3$                             | -311          | "   | $1.02 \times 10^3$                             | -326          | "   |
| 50  | $1.76 \times 10^3$                             | -251                                       | "   | $1.67 \times 10^3$                             | -285          | "   | $1.50 \times 10^3$                             | -341          | "   |
| 51  | $1.24 \times 10^3$                             | -240                                       | "   | $1.58 \times 10^3$                             | -295          | "   | $1.50 \times 10^3$                             | -341          | "   |
| 52  | $1.48 \times 10^3$                             | -259                                       | "   | $1.55 \times 10^3$                             | -336          | "   | $1.50 \times 10^3$                             | -341          | "   |
| 53  | 703                                            | +112                                       | "   | 884                                            | +162          | "   | 830                                            | +261          | "   |
| 54  | 625                                            | +101                                       | "   | 878                                            | +156          | "   | 816                                            | +258          | "   |

TABLE 16

| NO | Example 1                                         |               |                                  | Carbonate-Free                                    |               |                                  | Carbonate & Fluoride-Free                         |               |                                  |
|----|---------------------------------------------------|---------------|----------------------------------|---------------------------------------------------|---------------|----------------------------------|---------------------------------------------------|---------------|----------------------------------|
|    | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) |
| 1  | 2.92 × 10 <sup>3</sup>                            | +118          | <±2                              | 3.46 × 10 <sup>3</sup>                            | +321          | <±2                              | 3.14 × 10 <sup>3</sup>                            | +357          | <±2                              |
| 2  | 1.16 × 10 <sup>3</sup>                            | +124          | "                                | 2.03 × 10 <sup>3</sup>                            | +403          | "                                | 1.77 × 10 <sup>3</sup>                            | +421          | "                                |
| 3  | 983                                               | +159          | "                                | 1.65 × 10 <sup>3</sup>                            | +463          | "                                | 1.05 × 10 <sup>3</sup>                            | +480          | "                                |
| 4  | 786                                               | +214          | "                                | 892                                               | +494          | "                                | 828                                               | +676          | "                                |
| 5  | 2.98 × 10 <sup>3</sup>                            | +120          | "                                | 3.84 × 10 <sup>3</sup>                            | +360          | "                                | 3.13 × 10 <sup>3</sup>                            | +362          | "                                |
| 6  | 1.26 × 10 <sup>3</sup>                            | +123          | "                                | 2.35 × 10 <sup>3</sup>                            | +420          | "                                | 1.81 × 10 <sup>3</sup>                            | +427          | "                                |
| 7  | 965                                               | +160          | "                                | 2.14 × 10 <sup>3</sup>                            | +430          | "                                | 1.09 × 10 <sup>3</sup>                            | +480          | "                                |
| 8  | 789                                               | +223          | "                                | 874                                               | +490          | "                                | 831                                               | +675          | "                                |
| 9  | 963                                               | +163          | "                                | 1.92 × 10 <sup>3</sup>                            | +453          | "                                | 1.07 × 10 <sup>3</sup>                            | +485          | "                                |
| 10 | 1.03 × 10 <sup>3</sup>                            | +123          | "                                | 1.86 × 10 <sup>3</sup>                            | +314          | "                                | 1.78 × 10 <sup>3</sup>                            | +512          | "                                |
| 11 | 925                                               | +155          | "                                | 1.02 × 10 <sup>3</sup>                            | +368          | "                                | 1.13 × 10 <sup>3</sup>                            | +567          | "                                |
| 12 | 833                                               | +202          | "                                | 983                                               | +480          | "                                | 925                                               | +624          | "                                |
| 13 | 805                                               | +248          | "                                | 854                                               | +475          | "                                | 835                                               | +675          | "                                |
| 14 | 744                                               | +249          | "                                | 821                                               | +485          | "                                | 815                                               | +685          | "                                |
| 15 | 635                                               | +255          | "                                | 735                                               | +492          | "                                | 740                                               | +702          | "                                |
| 16 | 2.00 × 10 <sup>3</sup>                            | +89           | "                                | 1.96 × 10 <sup>3</sup>                            | +303          | "                                | 1.78 × 10 <sup>3</sup>                            | +512          | "                                |
| 17 | 1.51 × 10 <sup>3</sup>                            | +115          | "                                | 1.82 × 10 <sup>3</sup>                            | +343          | "                                | 1.13 × 10 <sup>3</sup>                            | +567          | "                                |
| 18 | 1.14 × 10 <sup>3</sup>                            | +126          | "                                | 1.72 × 10 <sup>3</sup>                            | +392          | "                                | 925                                               | +624          | "                                |
| 19 | 1.02 × 10 <sup>3</sup>                            | +180          | "                                | 1.68 × 10 <sup>3</sup>                            | +403          | "                                | 835                                               | +675          | "                                |
| 20 | 921                                               | +205          | "                                | 956                                               | +424          | "                                | 815                                               | +685          | "                                |
| 21 | 829                                               | +238          | "                                | 912                                               | +490          | "                                | 740                                               | +702          | "                                |
| 22 | 1.05 × 10 <sup>3</sup>                            | +105          | "                                | 1.12 × 10 <sup>3</sup>                            | +390          | "                                | 925                                               | +624          | "                                |
| 23 | 921                                               | +150          | "                                | 985                                               | +436          | "                                | 815                                               | +685          | "                                |
| 24 | 884                                               | +136          | "                                | 925                                               | +453          | "                                | 925                                               | +624          | "                                |
| 25 | 795                                               | +181          | "                                | 894                                               | +483          | "                                | 815                                               | +685          | "                                |
| 26 | 935                                               | +161          | "                                | 913                                               | +409          | "                                | 925                                               | +624          | "                                |
| 27 | 880                                               | +180          | "                                | 862                                               | +490          | "                                | 815                                               | +685          | "                                |
| 28 | 706                                               | +223          | "                                | 752                                               | +493          | "                                | 835                                               | +675          | "                                |
| 29 | 641                                               | +244          | "                                | 680                                               | +496          | "                                | 815                                               | +685          | "                                |
| 30 | 654                                               | +249          | "                                | 672                                               | +495          | "                                | 835                                               | +675          | "                                |
| 31 | 606                                               | +250          | "                                | 632                                               | +480          | "                                | 815                                               | +685          | "                                |
| 32 | 753                                               | +195          | "                                | 690                                               | +476          | "                                | 835                                               | +675          | "                                |
| 33 | 706                                               | +203          | "                                | 683                                               | +481          | "                                | 815                                               | +685          | "                                |
| 34 | 1.08 × 10 <sup>3</sup>                            | +123          | "                                | 1.12 × 10 <sup>3</sup>                            | +373          | "                                | 1.13 × 10 <sup>3</sup>                            | +567          | "                                |
| 35 | 1.14 × 10 <sup>3</sup>                            | +106          | "                                | 1.14 × 10 <sup>3</sup>                            | +359          | "                                | 1.13 × 10 <sup>3</sup>                            | +567          | "                                |
| 36 | 929                                               | +192          | "                                | 953                                               | +393          | "                                | 956                                               | +634          | "                                |

TABLE 17

| Nos | Example 1                                         |               |                                  | Carbonate-Free                                    |               |                                  | Carbonate & Fluoride-Free                         |               |                                  |
|-----|---------------------------------------------------|---------------|----------------------------------|---------------------------------------------------|---------------|----------------------------------|---------------------------------------------------|---------------|----------------------------------|
|     | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) |
| 1   | 9.07 × 10 <sup>3</sup>                            | -276          | <±2                              | 9.56 × 10 <sup>3</sup>                            | -483          | <±2                              | 9.13 × 10 <sup>3</sup>                            | -528          | <±2                              |
| 2   | 20.2 × 10 <sup>3</sup>                            | -278          | "                                | 23.1 × 10 <sup>3</sup>                            | -495          | "                                | 21.4 × 10 <sup>3</sup>                            | -676          | "                                |
| 3   | 16.5 × 10 <sup>3</sup>                            | -289          | "                                | 19.4 × 10 <sup>3</sup>                            | -496          | "                                | 17.6 × 10 <sup>3</sup>                            | -805          | "                                |
| 4   | 2.45 × 10 <sup>3</sup>                            | -216          | "                                | 3.77 × 10 <sup>3</sup>                            | -350          | "                                | 2.86 × 10 <sup>3</sup>                            | -396          | "                                |
| 5   | 825                                               | +222          | "                                | 1.01 × 10 <sup>3</sup>                            | +362          | "                                | 888                                               | +380          | "                                |
| 6   | 4.01 × 10 <sup>3</sup>                            | -152          | "                                | 4.22 × 10 <sup>3</sup>                            | -249          | "                                | 4.18 × 10 <sup>3</sup>                            | -256          | "                                |
| 7   | 31.6 × 10 <sup>3</sup>                            | -292          | "                                | 34.0 × 10 <sup>3</sup>                            | -486          | "                                | 32.1 × 10 <sup>3</sup>                            | -929          | "                                |
| 8   | 18.5 × 10 <sup>3</sup>                            | -296          | "                                | 24.1 × 10 <sup>3</sup>                            | -493          | "                                | 20.0 × 10 <sup>3</sup>                            | -956          | "                                |
| 9   | 6.88 × 10 <sup>3</sup>                            | -277          | "                                | 8.03 × 10 <sup>3</sup>                            | -446          | "                                | 7.14 × 10 <sup>3</sup>                            | -530          | "                                |
| 10  | 2.55 × 10 <sup>3</sup>                            | -242          | "                                | 3.96 × 10 <sup>3</sup>                            | -387          | "                                | 3.04 × 10 <sup>3</sup>                            | -407          | "                                |
| 11  | 4.29 × 10 <sup>3</sup>                            | -269          | "                                | 4.93 × 10 <sup>3</sup>                            | -477          | "                                | 4.80 × 10 <sup>3</sup>                            | -628          | "                                |
| 12  | 7.68 × 10 <sup>3</sup>                            | -275          | "                                | 8.95 × 10 <sup>3</sup>                            | -467          | "                                | 8.11 × 10 <sup>3</sup>                            | -607          | "                                |
| 13  | 25.4 × 10 <sup>3</sup>                            | -293          | "                                | 29.4 × 10 <sup>3</sup>                            | -480          | "                                | 26.4 × 10 <sup>3</sup>                            | -814          | "                                |
| 14  | 27.9 × 10 <sup>3</sup>                            | -261          | "                                | 34.9 × 10 <sup>3</sup>                            | -417          | "                                | 29.6 × 10 <sup>3</sup>                            | -505          | "                                |
| 15  | 10.6 × 10 <sup>3</sup>                            | -116          | "                                | 16.9 × 10 <sup>3</sup>                            | -290          | "                                | 11.4 × 10 <sup>3</sup>                            | -334          | "                                |
| 16  | 13.9 × 10 <sup>3</sup>                            | -288          | "                                | 14.7 × 10 <sup>3</sup>                            | -491          | "                                | 14.1 × 10 <sup>3</sup>                            | -769          | "                                |
| 17  | 9.21 × 10 <sup>3</sup>                            | -287          | "                                | 11.9 × 10 <sup>3</sup>                            | -465          | "                                | 10.6 × 10 <sup>3</sup>                            | -582          | "                                |
| 18  | 3.85 × 10 <sup>3</sup>                            | -249          | "                                | 4.95 × 10 <sup>3</sup>                            | -425          | "                                | 4.18 × 10 <sup>3</sup>                            | -520          | "                                |
| 19  | 12.6 × 10 <sup>3</sup>                            | -234          | "                                | 16.6 × 10 <sup>3</sup>                            | -392          | "                                | 12.8 × 10 <sup>3</sup>                            | -477          | "                                |
| 20  | 9.44 × 10 <sup>3</sup>                            | -216          | "                                | 14.3 × 10 <sup>3</sup>                            | -401          | "                                | 10.0 × 10 <sup>3</sup>                            | -500          | "                                |
| 21  | 924                                               | -169          | "                                | 1.18 × 10 <sup>3</sup>                            | -373          | "                                | 1.01 × 10 <sup>3</sup>                            | -423          | "                                |
| 22  | 8.05 × 10 <sup>3</sup>                            | -264          | "                                | 9.02 × 10 <sup>3</sup>                            | -495          | "                                | 8.18 × 10 <sup>3</sup>                            | -677          | "                                |
| 23  | 4.02 × 10 <sup>3</sup>                            | -250          | "                                | 5.13 × 10 <sup>3</sup>                            | -388          | "                                | 4.43 × 10 <sup>3</sup>                            | -459          | "                                |
| 24  | 1.21 × 10 <sup>3</sup>                            | -234          | "                                | 2.07 × 10 <sup>3</sup>                            | -379          | "                                | 1.52 × 10 <sup>3</sup>                            | -533          | "                                |
| 25  | 5.09 × 10 <sup>3</sup>                            | -262          | "                                | 7.09 × 10 <sup>3</sup>                            | -416          | "                                | 5.24 × 10 <sup>3</sup>                            | -540          | "                                |
| 26  | 5.49 × 10 <sup>3</sup>                            | -270          | "                                | 5.92 × 10 <sup>3</sup>                            | -433          | "                                | 5.84 × 10 <sup>3</sup>                            | -574          | "                                |
| 27  | 18.4 × 10 <sup>3</sup>                            | -298          | "                                | 22.2 × 10 <sup>3</sup>                            | -482          | "                                | 20.5 × 10 <sup>3</sup>                            | -865          | "                                |
| 28  | 12.6 × 10 <sup>3</sup>                            | -186          | "                                | 15.6 × 10 <sup>3</sup>                            | -316          | "                                | 13.3 × 10 <sup>3</sup>                            | -414          | "                                |

TABLE 17-continued

| Nos | Example 1                  |               |                                  | Carbonate-Free             |               |                                  | Carbonate & Fluoride-Free  |               |                                  |
|-----|----------------------------|---------------|----------------------------------|----------------------------|---------------|----------------------------------|----------------------------|---------------|----------------------------------|
|     | Resistance value at 25° C. | TCR (ppm/°C.) | Rate of Change in Resistance (%) | Resistance value at 25° C. | TCR (ppm/°C.) | Rate of Change in Resistance (%) | Resistance value at 25° C. | TCR (ppm/°C.) | Rate of Change in Resistance (%) |
|     | R <sub>25</sub> (Ω)        | (ppm/°C.)     | (%)                              | R <sub>25</sub> (Ω)        | (ppm/°C.)     | (%)                              | R <sub>25</sub> (Ω)        | (ppm/°C.)     | (%)                              |
| 29  | 4.11 × 10 <sup>3</sup>     | -107          | "                                | 5.20 × 10 <sup>3</sup>     | -222          | "                                | 4.46 × 10 <sup>3</sup>     | -295          | "                                |
| 30  | 28.4 × 10 <sup>3</sup>     | -284          | "                                | 36.3 × 10 <sup>3</sup>     | -492          | "                                | 31.1 × 10 <sup>3</sup>     | -639          | "                                |
| 31  | 16.0 × 10 <sup>3</sup>     | -292          | "                                | 16.9 × 10 <sup>3</sup>     | -499          | "                                | 16.5 × 10 <sup>3</sup>     | -821          | "                                |
| 32  | 925                        | -106          | "                                | 995                        | -232          | "                                | 990                        | -259          | "                                |
| 33  | 7.96 × 10 <sup>3</sup>     | -295          | "                                | 10.3 × 10 <sup>3</sup>     | -486          | "                                | 8.24 × 10 <sup>3</sup>     | -795          | "                                |
| 34  | 3.82 × 10 <sup>3</sup>     | -264          | "                                | 5.28 × 10 <sup>3</sup>     | -378          | "                                | 4.33 × 10 <sup>3</sup>     | -496          | "                                |
| 35  | 1.02 × 10 <sup>3</sup>     | +96           | "                                | 2.05 × 10 <sup>3</sup>     | +89           | "                                | 1.14 × 10 <sup>3</sup>     | +125          | "                                |
| 36  | 524                        | +250          | "                                | 647                        | +370          | "                                | 628                        | +482          | "                                |
| 37  | 36.0 × 10 <sup>3</sup>     | -289          | "                                | 37.7 × 10 <sup>3</sup>     | -485          | "                                | 36.3 × 10 <sup>3</sup>     | -992          | "                                |
| 38  | 15.5 × 10 <sup>3</sup>     | -275          | "                                | 19.0 × 10 <sup>3</sup>     | -466          | "                                | 16.4 × 10 <sup>3</sup>     | -584          | "                                |
| 39  | 8.00 × 10 <sup>3</sup>     | -270          | "                                | 9.93 × 10 <sup>3</sup>     | -447          | "                                | 8.14 × 10 <sup>3</sup>     | -534          | "                                |
| 40  | 4.05 × 10 <sup>3</sup>     | -206          | "                                | 6.01 × 10 <sup>3</sup>     | -250          | "                                | 4.27 × 10 <sup>3</sup>     | -317          | "                                |
| 41  | 5.09 × 10 <sup>3</sup>     | -219          | "                                | 5.70 × 10 <sup>3</sup>     | -365          | "                                | 5.45 × 10 <sup>3</sup>     | -487          | "                                |
| 42  | 2.26 × 10 <sup>3</sup>     | -244          | "                                | 3.07 × 10 <sup>3</sup>     | -430          | "                                | 2.87 × 10 <sup>3</sup>     | -521          | "                                |
| 43  | 12.0 × 10 <sup>3</sup>     | -289          | "                                | 14.9 × 10 <sup>3</sup>     | -477          | "                                | 12.4 × 10 <sup>3</sup>     | -855          | "                                |
| 44  | 7.03 × 10 <sup>3</sup>     | -294          | "                                | 10.2 × 10 <sup>3</sup>     | -411          | "                                | 7.14 × 10 <sup>3</sup>     | -505          | "                                |
| 45  | 5.49 × 10 <sup>3</sup>     | -233          | "                                | 9.05 × 10 <sup>3</sup>     | -395          | "                                | 6.23 × 10 <sup>3</sup>     | -480          | "                                |
| 46  | 980                        | +204          | "                                | 1.30 × 10 <sup>3</sup>     | +285          | "                                | 1.19 × 10 <sup>3</sup>     | +329          | "                                |
| 47  | 6.97 × 10 <sup>3</sup>     | -288          | "                                | 9.66 × 10 <sup>3</sup>     | -483          | "                                | 8.11 × 10 <sup>3</sup>     | -683          | "                                |
| 48  | 2.79 × 10 <sup>3</sup>     | -195          | "                                | 5.11 × 10 <sup>3</sup>     | -303          | "                                | 3.18 × 10 <sup>3</sup>     | -359          | "                                |
| 49  | 20.6 × 10 <sup>3</sup>     | -289          | "                                | 24.7 × 10 <sup>3</sup>     | -480          | "                                | 22.4 × 10 <sup>3</sup>     | -805          | "                                |
| 50  | 15.4 × 10 <sup>3</sup>     | -221          | "                                | 21.3 × 10 <sup>3</sup>     | -419          | "                                | 17.7 × 10 <sup>3</sup>     | -551          | "                                |
| 51  | 5.82 × 10 <sup>3</sup>     | -125          | "                                | 7.10 × 10 <sup>3</sup>     | -344          | "                                | 7.01 × 10 <sup>3</sup>     | -384          | "                                |
| 52  | 4.02 × 10 <sup>3</sup>     | -128          | "                                | 6.09 × 10 <sup>3</sup>     | -285          | "                                | 4.98 × 10 <sup>3</sup>     | -399          | "                                |
| 53  | 2.77 × 10 <sup>3</sup>     | -105          | "                                | 4.95 × 10 <sup>3</sup>     | -216          | "                                | 3.03 × 10 <sup>3</sup>     | -304          | "                                |
| 54  | 5.29 × 10 <sup>3</sup>     | -212          | "                                | 9.22 × 10 <sup>3</sup>     | -382          | "                                | 6.18 × 10 <sup>3</sup>     | -454          | "                                |
| 55  | 10.5 × 10 <sup>3</sup>     | -277          | "                                | 15.6 × 10 <sup>3</sup>     | -495          | "                                | 11.4 × 10 <sup>3</sup>     | -882          | "                                |
| 56  | 3.00 × 10 <sup>3</sup>     | -212          | "                                | 3.18 × 10 <sup>3</sup>     | -212          | "                                | 3.05 × 10 <sup>3</sup>     | -309          | "                                |
| 57  | 13.6 × 10 <sup>3</sup>     | -266          | "                                | 16.2 × 10 <sup>3</sup>     | -423          | "                                | 14.9 × 10 <sup>3</sup>     | -529          | "                                |
| 58  | 11.2 × 10 <sup>3</sup>     | -221          | "                                | 14.5 × 10 <sup>3</sup>     | -326          | "                                | 13.4 × 10 <sup>3</sup>     | -418          | "                                |
| 59  | 2.01 × 10 <sup>3</sup>     | -106          | "                                | 4.22 × 10 <sup>3</sup>     | -210          | "                                | 2.16 × 10 <sup>3</sup>     | -293          | "                                |
| 60  | 3.12 × 10 <sup>3</sup>     | -121          | "                                | 5.67 × 10 <sup>3</sup>     | -199          | "                                | 3.39 × 10 <sup>3</sup>     | -305          | "                                |
| 61  | 15.7 × 10 <sup>3</sup>     | -296          | "                                | 16.9 × 10 <sup>3</sup>     | -491          | "                                | 16.3 × 10 <sup>3</sup>     | -867          | "                                |
| 62  | 10.7 × 10 <sup>3</sup>     | -291          | "                                | 12.6 × 10 <sup>3</sup>     | -482          | "                                | 11.0 × 10 <sup>3</sup>     | -797          | "                                |
| 63  | 1.04 × 10 <sup>3</sup>     | -200          | "                                | 2.09 × 10 <sup>3</sup>     | -275          | "                                | 1.19 × 10 <sup>3</sup>     | -312          | "                                |
| 64  | 2.55 × 10 <sup>3</sup>     | -212          | "                                | 4.11 × 10 <sup>3</sup>     | -346          | "                                | 2.76 × 10 <sup>3</sup>     | -425          | "                                |
| 65  | 2.84 × 10 <sup>3</sup>     | -209          | "                                | 5.71 × 10 <sup>3</sup>     | -315          | "                                | 3.19 × 10 <sup>3</sup>     | -404          | "                                |
| 66  | 21.9 × 10 <sup>3</sup>     | -225          | "                                | 2.18 × 10 <sup>3</sup>     | -303          | "                                | 2.05 × 10 <sup>3</sup>     | -377          | "                                |
| 67  | 6.05 × 10 <sup>3</sup>     | -234          | "                                | 24.9 × 10 <sup>3</sup>     | -473          | "                                | 22.8 × 10 <sup>3</sup>     | -676          | "                                |
| 68  | 5.79 × 10 <sup>3</sup>     | -277          | "                                | 8.07 × 10 <sup>3</sup>     | -493          | "                                | 6.39 × 10 <sup>3</sup>     | -820          | "                                |
| 69  | 13.5 × 10 <sup>3</sup>     | -280          | "                                | 18.8 × 10 <sup>3</sup>     | -469          | "                                | 15.7 × 10 <sup>3</sup>     | -796          | "                                |
| 70  | 10.1 × 10 <sup>3</sup>     | -225          | "                                | 14.7 × 10 <sup>3</sup>     | -407          | "                                | 11.6 × 10 <sup>3</sup>     | -491          | "                                |
| 71  | 1.85 × 10 <sup>3</sup>     | -174          | "                                | 2.41 × 10 <sup>3</sup>     | -312          | "                                | 2.35 × 10 <sup>3</sup>     | -353          | "                                |
| 72  | 94.8 × 10 <sup>3</sup>     | -88           | "                                | 1.80 × 10 <sup>3</sup>     | -243          | "                                | 1.07 × 10 <sup>3</sup>     | -307          | "                                |
| 73  | 15.2 × 10 <sup>3</sup>     | -285          | "                                | 20.3 × 10 <sup>3</sup>     | -469          | "                                | 16.2 × 10 <sup>3</sup>     | -751          | "                                |
| 74  | 17.9 × 10 <sup>3</sup>     | -290          | "                                | 24.9 × 10 <sup>3</sup>     | -473          | "                                | 20.5 × 10 <sup>3</sup>     | -787          | "                                |
| 75  | 1.85 × 10 <sup>3</sup>     | -192          | "                                | 4.85 × 10 <sup>3</sup>     | -315          | "                                | 2.16 × 10 <sup>3</sup>     | -356          | "                                |
| 76  | 1.44 × 10 <sup>3</sup>     | +221          | "                                | 2.03 × 10 <sup>3</sup>     | +357          | "                                | 1.99 × 10 <sup>3</sup>     | +420          | "                                |
| 77  | 3.79 × 10 <sup>3</sup>     | -236          | "                                | 5.96 × 10 <sup>3</sup>     | -405          | "                                | 4.24 × 10 <sup>3</sup>     | -485          | "                                |
| 78  | 7.00 × 10 <sup>3</sup>     | -250          | "                                | 9.53 × 10 <sup>3</sup>     | -436          | "                                | 7.14 × 10 <sup>3</sup>     | -652          | "                                |
| 79  | 7.89 × 10 <sup>3</sup>     | -262          | "                                | 10.2 × 10 <sup>3</sup>     | -449          | "                                | 8.53 × 10 <sup>3</sup>     | -645          | "                                |
| 80  | 13.4 × 10 <sup>3</sup>     | -249          | "                                | 17.9 × 10 <sup>3</sup>     | -415          | "                                | 15.3 × 10 <sup>3</sup>     | -577          | "                                |
| 81  | 6.03 × 10 <sup>3</sup>     | -260          | "                                | 6.33 × 10 <sup>3</sup>     | -382          | "                                | 6.21 × 10 <sup>3</sup>     | -514          | "                                |
| 82  | 3.09 × 10 <sup>3</sup>     | -263          | "                                | 5.11 × 10 <sup>3</sup>     | -425          | "                                | 4.02 × 10 <sup>3</sup>     | -520          | "                                |
| 83  | 1.72 × 10 <sup>3</sup>     | -187          | "                                | 4.07 × 10 <sup>3</sup>     | -249          | "                                | 2.00 × 10 <sup>3</sup>     | -348          | "                                |
| 84  | 3.85 × 10 <sup>3</sup>     | -179          | "                                | 7.35 × 10 <sup>3</sup>     | -235          | "                                | 4.11 × 10 <sup>3</sup>     | -380          | "                                |
| 85  | 9.11 × 10 <sup>3</sup>     | -296          | "                                | 14.5 × 10 <sup>3</sup>     | -489          | "                                | 10.6 × 10 <sup>3</sup>     | -925          | "                                |
| 86  | 6.04 × 10 <sup>3</sup>     | -236          | "                                | 6.41 × 10 <sup>3</sup>     | -415          | "                                | 6.22 × 10 <sup>3</sup>     | -545          | "                                |
| 87  | 10.5 × 10 <sup>3</sup>     | -277          | "                                | 14.2 × 10 <sup>3</sup>     | -495          | "                                | 12.9 × 10 <sup>3</sup>     | -889          | "                                |
| 88  | 17.7 × 10 <sup>3</sup>     | -281          | "                                | 23.4 × 10 <sup>3</sup>     | -479          | "                                | 19.5 × 10 <sup>3</sup>     | -826          | "                                |
| 89  | 6.75 × 10 <sup>3</sup>     | -267          | "                                | 10.7 × 10 <sup>3</sup>     | -452          | "                                | 8.19 × 10 <sup>3</sup>     | -695          | "                                |
| 90  | 2.29 × 10 <sup>3</sup>     | -216          | "                                | 5.33 × 10 <sup>3</sup>     | -326          | "                                | 3.14 × 10 <sup>3</sup>     | -459          | "                                |
| 91  | 16.5 × 10 <sup>3</sup>     | -241          | "                                | 17.9 × 10 <sup>3</sup>     | -473          | "                                | 17.4 × 10 <sup>3</sup>     | -626          | "                                |
| 92  | 15.6 × 10 <sup>3</sup>     | -270          | "                                | 21.4 × 10 <sup>3</sup>     | -470          | "                                | 18.6 × 10 <sup>3</sup>     | -893          | "                                |
| 93  | 18.3 × 10 <sup>3</sup>     | -281          | "                                | 24.0 × 10 <sup>3</sup>     | -475          | "                                | 21.5 × 10 <sup>3</sup>     | -884          | "                                |
| 94  | 15.4 × 10 <sup>3</sup>     | -290          | "                                | 23.6 × 10 <sup>3</sup>     | -468          | "                                | 19.9 × 10 <sup>3</sup>     | -834          | "                                |
| 95  | 4.02 × 10 <sup>3</sup>     | -287          | "                                | 7.12 × 10 <sup>3</sup>     | -356          | "                                | 4.15 × 10 <sup>3</sup>     | -477          | "                                |
| 96  | 1.89 × 10 <sup>3</sup>     | -162          | "                                | 3.01 × 10 <sup>3</sup>     | -250          | "                                | 2.90 × 10 <sup>3</sup>     | -299          | "                                |
| 97  | 20.3 × 10 <sup>3</sup>     | -273          | "                                | 24.7 × 10 <sup>3</sup>     | -493          | "                                | 22.4 × 10 <sup>3</sup>     | -805          | "                                |
| 98  | 10.1 × 10 <sup>3</sup>     | -269          | "                                | 13.3 × 10 <sup>3</sup>     | -452          | "                                | 11.5 × 10 <sup>3</sup>     | -603          | "                                |
| 99  | 6.25 × 10 <sup>3</sup>     | -216          | "                                | 9.69 × 10 <sup>3</sup>     | -395          | "                                | 7.18 × 10 <sup>3</sup>     | -525          | "                                |
| 100 | 3.80 × 10 <sup>3</sup>     | -207          | "                                | 6.18 × 10 <sup>3</sup>     | -376          | "                                | 3.87 × 10 <sup>3</sup>     | -489          | "                                |
| 101 | 1.15 × 10 <sup>3</sup>     | -149          | "                                | 1.82 × 10 <sup>3</sup>     | -288          | "                                | 1.72 × 10 <sup>3</sup>     | -360          | "                                |
| 102 | 12.8 × 10 <sup>3</sup>     | -280          | "                                | 16.7 × 10 <sup>3</sup>     | -481          | "                                | 14.4 × 10 <sup>3</sup>     | -863          | "                                |
| 103 | 18.3 × 10 <sup>3</sup>     | -226          | "                                | 23.0 × 10 <sup>3</sup>     | -432          | "                                | 19.1 × 10 <sup>3</sup>     | -590          | "                                |

TABLE 17-continued

(Characteristic value corresponding to the sample in Table 9)

| Nos | Example 1                                         |               | Carbonate-Free                   |                                                   |               | Carbonate & Fluoride-Free        |                                                   |               |                                  |
|-----|---------------------------------------------------|---------------|----------------------------------|---------------------------------------------------|---------------|----------------------------------|---------------------------------------------------|---------------|----------------------------------|
|     | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) |
| 104 | $21.4 \times 10^3$                                | -280          | "                                | $29.2 \times 10^3$                                | -476          | "                                | $25.6 \times 10^3$                                | -842          | "                                |
| 105 | $7.03 \times 10^3$                                | -216          | "                                | $12.6 \times 10^3$                                | -358          | "                                | $9.02 \times 10^3$                                | -492          | "                                |
| 106 | 969                                               | +70           | "                                | 992                                               | +148          | "                                | 983                                               | +196          | "                                |
| 107 | $3.00 \times 10^3$                                | -201          | "                                | $3.56 \times 10^3$                                | -388          | "                                | $3.14 \times 10^3$                                | -502          | "                                |
| 108 | $4.17 \times 10^3$                                | -212          | "                                | $7.23 \times 10^3$                                | -365          | "                                | $5.01 \times 10^3$                                | -483          | "                                |
| 109 | $5.84 \times 10^3$                                | -182          | "                                | $9.44 \times 10^3$                                | -250          | "                                | $6.24 \times 10^3$                                | -314          | "                                |
| 110 | $5.99 \times 10^3$                                | -209          | "                                | $10.1 \times 10^3$                                | -371          | "                                | $6.92 \times 10^3$                                | -505          | "                                |
| 111 | $7.03 \times 10^3$                                | -220          | "                                | $7.51 \times 10^3$                                | -428          | "                                | $7.44 \times 10^3$                                | -521          | "                                |
| 112 | $9.76 \times 10^3$                                | -254          | "                                | $13.4 \times 10^3$                                | -452          | "                                | $11.0 \times 10^3$                                | -647          | "                                |
| 113 | $4.01 \times 10^3$                                | -172          | "                                | $6.33 \times 10^3$                                | -333          | "                                | $4.56 \times 10^3$                                | -424          | "                                |
| 114 | $4.70 \times 10^3$                                | -225          | "                                | $6.49 \times 10^3$                                | -329          | "                                | $4.73 \times 10^3$                                | -412          | "                                |
| 115 | $9.54 \times 10^3$                                | -185          | "                                | $15.4 \times 10^3$                                | -376          | "                                | $10.2 \times 10^3$                                | -509          | "                                |
| 116 | $9.09 \times 10^3$                                | -196          | "                                | $9.29 \times 10^3$                                | -395          | "                                | $9.18 \times 10^3$                                | -518          | "                                |
| 117 | $6.19 \times 10^3$                                | -200          | "                                | $8.81 \times 10^3$                                | -400          | "                                | $7.02 \times 10^3$                                | -540          | "                                |
| 118 | $6.25 \times 10^3$                                | -225          | "                                | $9.24 \times 10^3$                                | -416          | "                                | $6.88 \times 10^3$                                | -523          | "                                |
| 119 | $5.87 \times 10^3$                                | -230          | "                                | $10.1 \times 10^3$                                | -420          | "                                | $6.90 \times 10^3$                                | -520          | "                                |
| 120 | $5.14 \times 10^3$                                | -209          | "                                | $9.91 \times 10^3$                                | -405          | "                                | $5.89 \times 10^3$                                | -509          | "                                |

## EXAMPLE 2

In accordance with Example 1, multilayered ceramic substrates were prepared, except that the molybdates,

25 specified in Table 18, were used without any heat treatment, and their R<sub>25</sub>, TCR and rate of changes in resistance were measured. The results are indicated in Table 19 with the corresponding sample numbers.

TABLE 18

(Ex. 2 - Composition in the case without heattreating Molybdates with others)

| NOs | Molybdate (wt. %)                                      | Glass B (wt. %) | Composition      |                  |                  |                  |                   |                   |
|-----|--------------------------------------------------------|-----------------|------------------|------------------|------------------|------------------|-------------------|-------------------|
|     |                                                        |                 | SrF <sub>2</sub> | BaF <sub>2</sub> | MgF <sub>2</sub> | CaF <sub>2</sub> | SrCO <sub>3</sub> | BaCO <sub>3</sub> |
| 1   | MgMoO <sub>4</sub>                                     | 40              | 59               |                  |                  | 0.5              |                   | 0.5               |
| 2   | CaMoO <sub>4</sub>                                     | 40              | 59               | 0.5              |                  |                  |                   | 0.5               |
| 3   | SrMoO <sub>4</sub>                                     | 40              | 59               |                  |                  | 0.5              | 0.5               |                   |
| 4   | BaMoO <sub>4</sub>                                     | 40              | 59               |                  | 0.5              |                  |                   | 0.5               |
| 5   | (Mg <sub>0.3</sub> Ca <sub>0.7</sub> )MoO <sub>4</sub> | 60              | 20               | 10               |                  |                  |                   | 10                |
| 6   | MgMoO <sub>4</sub>                                     | 30              | 20               |                  |                  | 10               | 10                |                   |
|     | Ca <sub>3</sub> MoO <sub>6</sub>                       | 30              |                  |                  |                  |                  |                   |                   |
| 7   | ZnMoO <sub>4</sub>                                     | 65              | 34               |                  |                  | 0.5              |                   | 0.5               |
| 8   | Al <sub>2</sub> Mo <sub>3</sub> O <sub>12</sub>        | 60              | 39               | 0.5              |                  |                  | 0.5               |                   |
| 9   | ZrMo <sub>2</sub> O <sub>8</sub>                       | 45              | 54               | 0.5              |                  |                  |                   | 0.5               |
| 10  | HfMo <sub>2</sub> O <sub>8</sub>                       | 45              | 54               |                  |                  | 0.5              | 0.5               |                   |
| 11  | Y <sub>6</sub> MoO <sub>12</sub>                       | 80              | 5                | 7.5              |                  |                  |                   | 7.5               |
| 12  | La <sub>6</sub> MoO <sub>12</sub>                      | 80              | 5                | 7.5              |                  |                  |                   | 7.5               |
| 13  | Ce <sub>6</sub> MoO <sub>12</sub>                      | 80              | 5                | 7.5              |                  |                  |                   | 7.5               |
| 14  | Pr <sub>6</sub> MoO <sub>12</sub>                      | 80              | 5                | 7.5              |                  |                  |                   | 7.5               |
| 15  | Nd <sub>6</sub> MoO <sub>12</sub>                      | 80              | 5                | 7.5              |                  |                  |                   | 7.5               |
| 16  | Sm <sub>6</sub> MoO <sub>12</sub>                      | 80              | 5                | 7.5              |                  |                  |                   | 7.5               |
| 17  | Eu <sub>6</sub> MoO <sub>12</sub>                      | 80              | 5                | 7.5              |                  |                  |                   | 7.5               |
| 18  | Gd <sub>6</sub> MoO <sub>12</sub>                      | 80              | 5                | 7.5              |                  |                  |                   | 7.5               |
| 19  | Tb <sub>6</sub> MoO <sub>12</sub>                      | 80              | 5                | 7.5              |                  |                  |                   | 7.5               |
| 20  | Dy <sub>6</sub> MoO <sub>12</sub>                      | 80              | 5                | 7.5              |                  |                  |                   | 7.5               |
| 21  | Ho <sub>6</sub> MoO <sub>12</sub>                      | 80              | 5                | 7.5              |                  |                  |                   | 7.5               |
| 22  | Er <sub>6</sub> MoO <sub>12</sub>                      | 80              | 5                | 7.5              |                  |                  |                   | 7.5               |
| 23  | Tm <sub>6</sub> MoO <sub>12</sub>                      | 80              | 5                | 7.5              |                  |                  |                   | 7.5               |
| 24  | Yb <sub>6</sub> MoO <sub>12</sub>                      | 80              | 5                | 7.5              |                  |                  |                   | 7.5               |
| 25  | Lu <sub>6</sub> MoO <sub>12</sub>                      | 80              | 5                | 7.5              |                  |                  |                   | 7.5               |
| 26  | Nb <sub>2</sub> Mo <sub>3</sub> O <sub>14</sub>        | 55              | 44               | 0.5              |                  |                  |                   | 0.5               |
| 27  | Ta <sub>2</sub> Mo <sub>3</sub> O <sub>14</sub>        | 55              | 44               |                  | 0.5              | 0.5              |                   |                   |
| 28  | MnMoO <sub>4</sub>                                     | 65              | 34               |                  | 0.5              | 0.5              |                   |                   |

fluorides and glass powders having the compositions

TABLE 19

(Characteristic value corresponding to the sample in Table 18)

| Nos | Example 2                                         |               |                                  | Fluoride-Free                                     |               |                                  |
|-----|---------------------------------------------------|---------------|----------------------------------|---------------------------------------------------|---------------|----------------------------------|
|     | Resistance value at 25° C.<br>R <sub>25</sub> (Ω) | TCR (ppm/°C.) | Rate of Change in Resistance (%) | Resistance value at 25° C.<br>R <sub>25</sub> (Ω) | TCR (ppm/°C.) | Rate of Change in Resistance (%) |
| 1   | $3.04 \times 10^3$                                | -1316         | <±2                              | $4.35 \times 10^3$                                | -1356         | <±2                              |
| 2   | $29.8 \times 10^3$                                | -1435         | "                                | $35.2 \times 10^3$                                | -1483         | "                                |

TABLE 19-continued

| Nos | Example 2                                       |               |                                  | Fluoride-Free                                   |               |                                  |
|-----|-------------------------------------------------|---------------|----------------------------------|-------------------------------------------------|---------------|----------------------------------|
|     | Resistance value at 25° C.<br>$R_{25} (\Omega)$ | TCR (ppm/°C.) | Rate of Change in Resistance (%) | Resistance value at 25° C.<br>$R_{25} (\Omega)$ | TCR (ppm/°C.) | Rate of Change in Resistance (%) |
| 3   | 674                                             | -1385         | "                                | 823                                             | -1411         | "                                |
| 4   | 388                                             | +1156         | "                                | 524                                             | +1192         | "                                |
| 5   | $8.44 \times 10^3$                              | -1384         | "                                | $9.83 \times 10^3$                              | -1401         | "                                |
| 6   | $6.24 \times 10^3$                              | -1309         | "                                | $7.29 \times 10^3$                              | -1328         | "                                |
| 7   | $4.80 \times 10^3$                              | -1370         | "                                | $5.63 \times 10^3$                              | -1412         | "                                |
| 8   | $11.6 \times 10^3$                              | -1462         | "                                | $12.5 \times 10^3$                              | -1489         | "                                |
| 9   | $17.4 \times 10^3$                              | -1615         | "                                | $18.9 \times 10^3$                              | -1676         | "                                |
| 10  | $15.4 \times 10^3$                              | -1468         | "                                | $16.2 \times 10^3$                              | +1498         | "                                |
| 11  | $5.95 \times 10^3$                              | -1216         | "                                | $6.82 \times 10^3$                              | -1273         | "                                |
| 12  | $5.03 \times 10^3$                              | -1206         | "                                | $6.23 \times 10^3$                              | -1256         | "                                |
| 13  | $3.95 \times 10^3$                              | -1195         | "                                | $4.36 \times 10^3$                              | +1232         | "                                |
| 14  | $3.88 \times 10^3$                              | -1192         | "                                | $4.21 \times 10^3$                              | -1213         | "                                |
| 15  | $4.99 \times 10^3$                              | -1312         | "                                | $5.36 \times 10^3$                              | -1363         | "                                |
| 16  | $3.79 \times 10^3$                              | -1369         | "                                | $4.31 \times 10^3$                              | -1401         | "                                |
| 17  | $4.05 \times 10^3$                              | -1287         | "                                | $5.01 \times 10^3$                              | -1302         | "                                |
| 18  | $7.61 \times 10^3$                              | -1305         | "                                | $8.34 \times 10^3$                              | +1363         | "                                |
| 19  | $7.18 \times 10^3$                              | -1269         | "                                | $8.05 \times 10^3$                              | -1272         | "                                |
| 20  | $7.33 \times 10^3$                              | -1050         | "                                | $8.65 \times 10^3$                              | -1080         | "                                |
| 21  | $7.18 \times 10^3$                              | -1182         | "                                | $8.23 \times 10^3$                              | -1210         | "                                |
| 22  | $7.85 \times 10^3$                              | -1324         | "                                | $8.41 \times 10^3$                              | -1363         | "                                |
| 23  | $6.94 \times 10^3$                              | -1306         | "                                | $7.81 \times 10^3$                              | +1353         | "                                |
| 24  | $6.03 \times 10^3$                              | -1244         | "                                | $7.03 \times 10^3$                              | -1286         | "                                |
| 25  | $4.67 \times 10^3$                              | -1195         | "                                | $5.63 \times 10^3$                              | -1215         | "                                |
| 26  | 625                                             | +1059         | "                                | 725                                             | +1080         | "                                |
| 27  | $1.45 \times 10^3$                              | -1345         | "                                | $2.03 \times 10^3$                              | -1376         | "                                |
| 28  | 905                                             | +1230         | "                                | $1.06 \times 10^3$                              | -1271         | "                                |

Comparison Example 1 (MoSi<sub>2</sub>-TaSi<sub>2</sub> Glass Base 30  
Resistor Material)

A mixture of 16 parts by weight of MoSi<sub>2</sub> with 9 parts by weight of TaSi<sub>2</sub> was heated at 1400° C. in vacuum. The resulting product was pulverized together with ethanol by alumina balls in a pot mill for 24 hours, and was dried to obtain fine powders having a particle size of 10  $\mu\text{m}$  or lower. Seventy five (75) parts by weight of glass frit consisting of BaO, B<sub>2</sub>O<sub>3</sub>, MgO, CaO and SiO<sub>2</sub> and 25 parts by weight of the organic vehicle (20 parts by weight of butyl carbitol plus 5 parts by weight of ethyl cellulose) were added to 25 parts by weight of the thus obtained fine powders, and were roll-milled to obtain a resistive paste.

Except that this resistive paste was used, a multilayered ceramic board was obtained in the same manner as in the foregoing examples.

As a result, the product obtained by forming the resistive film produced from said paste on a ceramic green sheet, heat-treating them for the decomposition of the organics and, thereafter, simultaneously sintering them could not be put to practical use, since it warped due to differences in the coefficients of expansion and shrinkage between both the sintered bodies, as illustrated in FIG. 4, and swelled due to the evolution of a gas by the decomposing reaction of MoSi<sub>2</sub> and TaSi<sub>2</sub>, as illustrated in FIG. 5. It is to be noted that 11a, 14a and 13a are a layer corresponding to the aforesaid layer 1a, a layer corresponding to the aforesaid layer 4a and a thick-film resistor corresponding to the aforesaid thick-film resistor 3a, respectively.

Comparison Example 2 (MoSi<sub>2</sub>-BaF<sub>2</sub> Glass Base Resistor Material)

Seventy (70) parts by weight of MoSi<sub>2</sub> and 20 parts by weight of BaF<sub>2</sub> were mixed with 10 parts by weight of glass frit comprising SiO<sub>2</sub>, ZnO, ZrO<sub>2</sub>, CaO and Al<sub>2</sub>O<sub>3</sub> by ball-milling, and the resulting powders were heat-treated at 1200° C. in an argon (Ar) gas atmosphere. Thereafter, the product was pulverized together with

ethanol for 24 hours by alumina balls in a pot mill, and was dried to obtain fine powders having a particle size of 10  $\mu\text{m}$  or lower.

Except that this resistive paste was used, a multilayered ceramic board was obtained in the same manner as in Example 1. Shown in Table 20 are the results of the R<sub>25</sub>, TCR and rate of change in resistance value of the thick-film resistor of the multilayered ceramic substrate, which were measured in the same manner as in Example 1.

TABLE 20

|             | Resistance Value R <sub>25</sub> at 25° C., Ohms | TCR ppm/°C. | Rate of Change in Resistance Value, % |
|-------------|--------------------------------------------------|-------------|---------------------------------------|
| Comp. Ex. 2 | 124.5                                            | +1120       | 9.7% increase                         |

From the above results, it has been found that the multilayered ceramic boards according to the examples all undergo neither warping nor swelling, and their rate of change in resistance value is within  $\pm 2\%$ , and that, in particular, the TCR of those having the resistor material heat-treated does not exceed  $\pm 500$  ppm/°C. in the case where the fluorides of alkaline earth metals are used and  $\pm 300$  ppm/°C. in the case where the carbonates of alkaline earth metals are used. It has been noted, on the other hand, that the multilayered ceramic board of Comp. Ex. 1 undergoes warping, whereas the multilayered ceramic board of Comp. Ex. 2 has its resistor showing a rate of change in resistance value that is four times higher and a TCR that is one order of magnitude higher.

Effects of the Invention

According to the present invention, there can be provided a sintered body containing at least one molybdate selected from at least one molybdate group selected from the groups (A) to (G) defined in the forego-

ing, with or without the fluoride of an alkaline earth metal, and an electrical resistor paste containing a resistive material for said sintered body and the carbonate of an alkaline earth metal. Accordingly, if the resistor material or paste for this sintered body is used and sintered along with a conductor material based on, e.g. a base metal and a ceramic green sheet in a nonoxidizing atmosphere to form a resistor, it is very unlikely that the sintered body may either warp or swell due to sintering. It is further possible not only to decrease a change-with-time of the resistance value esp. at a high humidity but also to reduce the temperature dependence coefficient of the resistance value of the resistor not to exceed  $\pm 300$  ppm/ $^{\circ}$ C., for instance.

Hence, it is possible to meet both the demands for 15 reductions in the size and cost of circuit boards having resistors incorporated thereinto and to provide excellent electronic parts to electronic equipment needing precise work.

Further, if the molybdate belonging to the aforesaid 20 groups (A) to (G), preferably with the fluoride of an alkaline earth metal are heat-treated with glass, it is then possible to decrease the absolute value of the temperature dependent coefficient of the resistor and add excellent 25 capabilities to electronic circuits needing precise performance, compared with the case where such any heat-treatment is not carried out.

What is claimed is:

1. An electrical resistor which is sintered body comprising bulk particles, acicular particles deposited onto 30 said bulk particles, a fluoride of an alkaline earth metal represented by the formula  $Me'F_2$ , wherein  $Me$  is an alkaline earth metal, and a glass layer, said bulk particles comprising at least one molybdate selected from the 35 group consisting of (A) to (G), and said acicular particles containing a reduction product of said molybdate:

- (A) 30-96 weight % molybdates of alkaline earth metals,
- (B) 55-95 weight % molybdates of zinc,
- (C) 50-96 weight % molybdates of elements Y, La, Ce, Pr, Nd, Sm, Eu, Gd, Tb, Dy, Ho, Er, Tm, BYb and Lu, and complex molybdates of two or more of said elements,
- (D) 35-96 weight % molybdates of aluminium,
- (E) 40-96 weight % molybdates of elements zirconium and hafnium, and complex molybdates thereof,
- (F) 45-96 weight % molybdates of elements niobium and tantalum, and complex molybdates thereof, and
- (G) 50-96 weight % molybdates of manganese.

2. The electrical resistor as defined in claim 17, wherein said bulk and acicular particles are obtained by sintering a resistor material containing as one of the main components at least one of the molybdate or molybdates selected from the molybdate group or groups consisting of (A) to (G) and its or their precursors.

3. The electrical resistor as defined in claim 17 or 18, wherein said acicular particles are a product obtained by the reduction of the surfaces of said bulk particles.

4. The electrical resistor as defined in claim 1, wherein the molybdates of alkaline earth metals are selected from the group consisting of  $MeMoO_4$ ,  $Me_3MoO_6$ ,  $Me_2MoO_5$ ,  $Me_2Mo_7$ ,  $MeMo_4O_{13}$ ,  $MeMo_7O_{24}$ ,  $MeMo_3O_{10}$ ,  $Me_2Mo_5$  and  $Me_2Mo_3O_{11}$ , wherein  $Me$  is an alkaline earth metal.

5. The electrical resistor as defined in claim 1, wherein the molybdates of alkaline earth metals are

selected from the group consisting of  $MgMoO_4$ ,  $CaMoO_4$ ,  $SrMoO_4$ ,  $BaMoO_4$ ,  $BaMo_2O_7$ ,  $BaMo_4O_{13}$ ,  $BaMo_7O_{24}$ ,  $BaMo_3O_{10}$ ,  $Ca_2MoO_6$ ,  $Sr_2MoO_6$ ,  $BaMoO_6$ ,  $Ba_2MoO_5$ , and  $Mg_2Mo_3O_{11}$ .

6. The electrical resistor as defined in claim 1, wherein the molybdates of alkaline earth metals are complex molybdates selected from the group consisting of

10  $(Mg_x Ca_y)MoO_4$ , provided that  $x+y=1$ ,

$(Ca_x Sr_y)MoO_4$ , provided that  $x+y=1$ ,

$(Mg_x Ba_y)MoO_4$ , provided that  $x+y=1$ ,

$(Mg_x Ca_y Ba_z)MoO_4$ , provided that  $x+y+z=1$ ,

$(Ca_x Sr_y Ba_z)MoO_4$ , provided that  $x+y+z=1$ ,

$(Mg_x Ca_y Sr_z Ba_w)MoO_4$ , provided that  $x+y+z+w=1$ ,

$(Ca_x Sr_y)MoO_6$ , provided that  $x+y=1$ , and

$(Sr_x Ba_y)MoO_6$ , provided that  $x+y=1$ .

7. The electrical resistor as defined in claim 1, wherein molybdates of zinc are selected from the group consisting of  $ZnMoO_4$ ,  $ZnMo_2O_7$  and  $Zn_3Mo_2O_9$ .

8. The electrical resistor as defined in claim 1, wherein complex molybdates of two or more of the elements of group (C) are selected from the group consisting of

30  $(Y_x Ce_y)MoO_{12}$ , provided that  $x+y=6$ ,

$(Pr_x Eu_y)MoO_{12}$ , provided that  $x+y=6$ ,

$(Gd_x Dy_y)MoO_{12}$ , provided that  $x+y=6$ , and

$(Ho_x Tm_y Yb_z)MoO_{12}$ , provided  $x+y+z=6$ .

9. The electrical resistor as defined in claim 1, wherein a molybdate of aluminium is  $Al_2Mo_3O_{12}$ .

10. The electrical resistor as defined in claim 1, wherein molybdates of group (E) are selected from the group consisting of  $ZrMo_2O_3$ ,  $HfMo_2O_8$  and  $(Zr_x Hf_y)Mo_2O_3$ , provided that  $x+y=1$ .

11. The electrical resistor as defined in claim 1, wherein molybdates of group (F) are selected from the group consisting of  $Nb_2Mo_3O_{14}$ ,  $Ta_2Mo_3O_{14}$  and  $(Nb_x Ta_y)Mo_3O_{14}$ , provided that  $x+y=1$ .

12. The electrical resistor as defined in claim 1, wherein a molybdate of manganese is  $MnMoO_4$ .

13. The electrical resistor as defined in claim 1, wherein the glass layer comprises glass components selected from the group consisting of 12 to 33% by weight  $SiO_2$ , 20 to 35% by weight  $B_2O_3$ , 13 to 33% by weight  $ZnO$ , 13 to 33% by weight  $SrO$ , 10 to 25% by weight  $Cao$  and 15 to 45% by weight  $ZrO_2$ .

14. The electrical resistor as defined in claim 1, wherein the molybdate is selected from the group consisting of 40-95 weight % (A), 65-95 weight % (B), 60-95 weight % (C), 45-95 weight % (O), 50-95 weight % (E), 55-95 weight % (F) and 65-95 weight % (G).

15. The electrical resistor as defined in claim 1, wherein the molybdate is selected from the group consisting of 30-95 weight % (A), 60-95 weight % (B), 55-95 weight % (C), 40-95 weight % (D), 40-95 weight % (E), 50-95 weight % (F) and 55-95 weight % (G).

\* \* \* \* \*